# EUROPEAN PATENT SPECIFICATION

(11) **EP 1 308 776 B1**
(45) Date of publication and mention of the grant of the patent: **15.08.2007**
(21) Application number: 02024554.4
(22) Date of filing: 04.11.2002
(51) Int. Cl.: G03C 1/498, G03C 7/305

(54) **Photothermographic material and method of thermal development of the same**
Photothermographisches Material und Verfahren zur thermischen Entwicklung von diesem
Matériau photothermographique et son procédé de développement thermique

(30) Priority: 05.11.2001 JP 2001339636; 08.11.2001 JP 2001342983; 09.11.2001 JP 2001344727; 29.11.2001 JP 2001364512; 29.03.2002 JP 2002096660; 29.03.2002 JP 2002097920
(43) Date of publication of application: 07.05.2003
(62) Divisional of application: 07010257.9
(73) Proprietor: FUJIFILM Corporation, Minato-ku Tokyo (JP)
(72) Inventor: Oka, Yutaka, Minami-Ashigara-shi, Kanagawa (JP); Ohzeki, Tomoyuki, Minami-Ashigara-shi, Kanagawa (JP); Yamane, Katsutoshi, Minami-Ashigara-shi, Kanagawa (JP); Yamamoto, Seiichi, Minami-Ashigara-shi, Kanagawa (JP); Yamada, Sumito, Minami-Ashigara-shi, Kanagawa (JP); Mifune, Hiroyuki, Minami-Ashigara-shi, Kanagawa (JP); Inaba, Tadashi, Minami-Ashigara-shi, Kanagawa (JP); Watanabe, Katsuyuki, Minami-Ashigara-shi, Kanagawa (JP); Yamada, Kohzaburoh, Minami-Ashigara-shi, Kanagawa (JP)
(74) Representative: HOFFMANN EITLE

(56) References cited:
- EP-A- 0 218 385
- EP-A- 0 851 284
- EP-A- 1 072 948
- EP-A- 1 168 064
- EP-A- 1 306 720
- US-A- 6 083 680
- DATABASE WPI Section Ch, Week 200008 Derwent Publications Ltd., London, GB; Class A89, AN 2000-091108 XP002250328 -& JP 11 327078 A (KONICA CORP), 26 November 1999 (1999-11-26)
- DATABASE WPI Section Ch, Week 200216 Derwent Publications Ltd., London, GB; Class E12, AN 2002-117427 XP002250329 -& JP 2001 272743 A (FUJI PHOTO FILM CO LTD), 5 October 2001 (2001-10-05)
- DATABASE WPI Section Ch, Week 198904 Derwent Publications Ltd., London, GB; Class G06, AN 1989-027484 XP002250330 -& JP 63 300234 A (KONISHIROKU PHOTO IND CO LTD), 7 December 1988 (1988-12-07)
- DATABASE WPI Section Ch, Week 197430 Derwent Publications Ltd., London, GB; Class E24, AN 1974-54584V XP002250331 & JP 49 025498 B (ORIENTAL PHOTO IND CO), 1 July 1974 (1974-07-01)
- DATABASE WPI Section Ch, Week 200045 Derwent Publications Ltd., London, GB; Class A14, AN 2000-501079 XP002250332 & JP 2000 171936 A (FUJI PHOTO FILM CO LTD), 23 June 2000 (2000-06-23)

## Description

### BACKGROUND OF THE INVENTION

### Field of the Invention:

The present invention relates to a photothermographic material and a method of thermal development of it. Precisely, the invention relates to a photothermographic material of which the advantages are that the printout images formed thereon are fogged little and the raw film storage stability thereof is good, and to a photothermographic material which comprises a silver halide emulsion having a silver iodide content and of which the advantages are that its sensitivity is extremely high and its image storability after developed is good, especially that its high sensitivity is supported by its low Dmin and high Dmax. The invention also relates to a method of thermal development of such a photothermographic material.

### Description of the Related Art:

In the field of photographic films for medical treatment, these days much desired is reducing the wastes of processing solutions for environmental protection and space saving. In that situation, required are techniques with photothermographic materials for medical diagnosis and photomechanical process capable of being efficiently exposed with laser image setters or laser imagers to form sharp and clear monochromatic images of high resolution. Such photothermographic materials could provide users with more simple photothermographic systems not requiring solution-type processing chemicals and therefore not polluting the environment.

The same applies to the field of ordinary photo-imaging materials, which, however, shall differ from those in the field of medical treatment. Specifically, photo-images for medical treatment must clarify the details of body parts and therefore must have sharp and good image quality with fine graininess. In addition, for easy diagnosis thereon, preferred are cold black images in the field of medical treatment. At present, various types of hard copy systems with pigment and dye, for example, ink jet printers and electrophotographic systems are available for ordinary image-forming systems. However, no one knows satisfactory systems for forming photo-images enough for medical treatment.

On the other hand, photothermographic systems with organic silver salts used therein are described, for example, in USP 3,152,904 and 3,457,075, and in B. Shely's "Thermally Processed Silver Systems" (Imaging Processes and Materials, Neblette, 8th Ed., compiled by Sturge, V. Walworth & A. Shepp, page 2, 1996).

In general, photothermographic materials have a photosensitive layer with a catalytically active amount of a photocatalyst (e.g., silver halide), a reducing agent, a reducible silver salt (e.g., organic silver salt), and optionally a toning agent for controlling silver tones being dispersed in a binder matrix in the layer. Photothermographic materials of that type are, after having been imagewise exposed, heated at a high temperature (for example, at 80°C or higher) to form black silver images through redox reaction between the silver halide or the reducible silver salt (serving as an oxidizing agent) and the reducing agent therein. In these, the redox reaction is accelerated by the catalytic action of the latent image of the exposed silver halide. Therefore, the black silver images are formed in the exposed area of the materials. This technique is disclosed in many references such as typically USP 2,910,377 and JP-B 43-4924, and an image-forming system with a photothermographic material for medical treatment, Fuji Medical Dry Imager FM-DPL has went on the market.

For producing thermal image-forming systems with organic silver salts therein, known are a method of using a solvent in forming the photosensitive layer therein, and a method of coating the substrate with a coating liquid that contains an aqueous dispersion of polymer particles serving as an essential binder, followed by drying it. The latter method does not require solvent recovery and therefore the equipment for it is simple. For these reasons, the latter method is favorable to industrial scale mass-production of the image-forming systems.

Not requiring image fixation after development, one serious problem with such image-forming systems with organic silver salts therein is that their image storability after development is not good, especially their printout images are often faded or fogged when left exposed to light. To solve the problem of printout image fogging, a method of using AgI formed through conversion of organic silver salts is disclosed in USP 6,143,488 and EP 0922995. However, the method disclosed of converting organic silver salts with iodine could not still satisfactorily improve the sensitivity of the photothermographic material to be in the image-forming systems, and it is not effective for planning practicable systems.

Other photothermographic materials that comprise AgI are described, for example, in W097-48014, WO 48015, USP 6,165,705, JP-A 8-297345 and Japanese Patent 2,785,129, but their sensitivity and fogging resistance are not still on a satisfactory level and all these are not practicable for laser exposure. Given that situation, desired is developing a method of more effectively using silver halides having such a high silver iodide content in practicable photothermographic materials.

Some means of increasing the sensitivity of silver iodide photographic emulsions are described in the Journal of Photographic Science, Vol. 8, page 119, 1960, ibid., Vol. 28, page 163, 1980; and in Photographic Science and Engineering, Vol. 5, page 216, 1961. For example, known is a method of sensitizing the photographic emulsions by dipping them in a halogen receptor such as sodium sulfite, pyrogallol or hydroquinone or in an aqueous solution of silver nitrate, or a method of sensitizing them with sulfur at pAg of 7.5. However, as in Examples shown hereinunder, the sensitizing effect of the halogen receptor is extremely low and is therefore unsatisfactory for photothermographic materials to which the invention is directed. Accordingly, it is desired to develop a technique effective for significantly increasing the sensitivity of photothermographic materials having a high silver iodide content.

JP-A 8-272024 discloses a technique of increasing the sensitivity of silver iodobromide emulsions having a low silver iodide content for color negative emulsions to be processed through liquid development or for emulsions for X-ray exposure, in which is specifically used a compound having a silver halide-adsorbing group and a reducing group or its precursor.

However, in such silver halide photographic materials to be processed through liquid development, the silver halide is generally reduced with a developing agent (reducing agent) that is in the processing liquid to thereby form a silver image, or the side-produced oxidation product of the developing agent is used for color image formation. Anyhow, in these, the basic reaction is reduction of silver halides with a developing agent. On the other hand, in photothermographic materials, the silver halide is only to form a latent image through exposure to light, and it is not reduced by the reducing agent in the materials. In such photothermographic materials, not the non-photosensitive organic silver salts but the silver ions applied thereto are reduced. The reducing agent for liquid development is an ionic reducing agent of, for example, hydroquinones or p-phenylenediamines, but that for photothermographic materials is generally a hindered phenol derivative known as a radical reactant.

As in the above, photographic materials for liquid development and photothermographic materials quite differ in point of the mechanism of development reaction (reduction) to occur therein, and in point of the series of compounds to be used for them. Accordingly, it should not be said that the compounds effective for liquid development are all the time directly effective for photothermographic materials. For example, the compounds described in the above-mentioned JP-A 8-272024 are not expected at all for photothermographic materials, and, needless-to-say, no one knows the applicability of the compounds to photothermographic materials with a high silver iodide emulsion therein and it is impossible for any one to expect the effect of the compounds in photothermographic materials.

As an ultra-hard image-forming agent for forming ultra-hard images, known are adsorbing group-having acylhydrazines. It is known that such adsorbing group-having acylhydrazines are effective for forming ultra-hard images also in photothermographic materials. This is because of the action of such acylhydrazines for infection development, and such acylhydrazines are effective for forming ultra-hard images in photothermographic materials but the graininess of the images formed is not good. Therefore, using such acylhydrazines in processing photothermographic materials will be suitable for processing them for making printing plates but is unsuitable at all for processing them for use in medical diagnosis. Accordingly, such adsorbing group-having acylhydrazines are unsuitable for the object of increasing the sensitivity of photographic silver halides having a high silver iodide content for forming high-quality images.

On the other hand, the recent tendency in the art is toward further small-sized exposure devices for thermal image-forming systems with organic silver salts therein, and it is much desired to further increase the sensitivity of photosensitive silver halides for the systems. After thermally developed, the density of the image area of thermal image-forming systems with organic silver salts therein often increases if the exposed photographic materials receive light while they are stored. For solving the problem in printout failure, it is known that reducing the photosensitive silver halide content of the photographic materials is effective.

However, the reduction in the photosensitive silver halide content of the photographic materials results in the reduction in the sensitivity of the photographic materials themselves and therefore the reduction in the maximum density of the images formed on the materials. Given that situation, it is desired to more effectively improve the storability of processed photothermographic materials not by the means of reducing the photosensitive silver halide content of the materials.

### SUMMARY OF THE INVENTION

The object of the present invention is to provide a high-sensitivity silver halide photothermographic material having a high silver iodide content and capable of forming high-quality images; to provide such a photothermographic material of which the advantages are that the maximum density of the images formed thereon is satisfactorily high, the raw film storage stability thereof is good, and the material is fogged little after thermally developed; to provide such a photothermographic material of which the advantages are that the optical image storability thereof is good after thermally developed, and the images formed thereon have a lowered Dmin and an increased Dmax; to provide such a silver halide photothermographic material of which the advantages are that it is rapidly developed and is stable irrespective of the time for development, and it gives images of good printout quality; and to provide a method of thermal development of such a photothermographic material.

The object of the invention is attained by the photothermographic material and the method of thermal development of it as specified in the appended claims and as referred to as the first to eleventh embodiment of the present invention.

### BRIEF DESCRIPTION OF THE DRAWINGS

Fig. 1 shows the light absorbance curve of a silver iodide emulsion.

### DESCRIPTION OF THE PREFERRED EMBODIMENTS

### Photothermographic Material, and Method of Thermal Development Thereof:

### - First Embodiment of Photothermographic Material -

The first embodiment of the photothermographic material of the present invention is described below.

A first embodiment of the present invention is a photothermographic material comprising a support having thereon a layer including at least a non-photosensitive organic silver salt, a photosensitive silver halide, a reducing agent and a binder, wherein the photosensitive silver halide has a mean silver iodide content of 5 to 100 mol % and further comprising at least one compound of the following general formula (I) mentioned below.

It is a matter of importance that the halogen composition of the photosensitive silver halide to be used in the first embodiment of the invention is a high silver iodide emulsion of which the silver iodide content falls between 5 mol% and 100 mol%. In general, the sensitivity of silver halides having such a high silver iodide content is low and the utility value thereof is therefore low.

Preferably, a part of the silver halide in the first embodiment of the invention has a phase capable of absorbing light through direct transition. It is well known that high silver iodide grains having a hexagonal-system wurtzite structure of a cubic-system zinc-blend structure realize light absorption through direct transition in the wavelength range of from 350 nm to 450 nm in which the silver halide grains are exposed to light. However, the sensitivity of the silver halide having such an absorption structure is generally low, and the utility value thereof in the field of photography is therefore low.

Through our studies, we, the present inventors have found that, when a compound of formula (I) as in the first embodiment of the invention is used in a photothermographic material that contains a non-photosensitive organic silver salt and a thermal developer, then the material may have a high sensitivity even though the photosensitive silver halide therein has a high silver iodide content, and may form sharp images.

Our studies have revealed that the grain size of the silver halide grains in the material is preferably at most 80 nm, more preferably 5 nm to 80 nm and especially preferably 5 nm to 70nm. Containing such small-size silver halide grains, the advantages of the material of the invention are more remarkable.

The contents of the invention are described in more detail hereinunder.

### <Compound of Formula (I)>

First described is the compound of formula (I) that shall be in the photothermographic material of the first embodiment of the invention.

In formula (I), X represents a silver halide-adsorbing group or a light-absorbing group that has at least one atom of N, S, P, Se and Te.

Preferably, X is a silver halide-adsorbing group that has at least one atom of N, S, P, Se and Te and has a silver ion ligand structure. The silver halide-adsorbing group that has such a silver ion ligand structure includes, for example, those of general formulae mentioned below.

General Formula (X-1) -G¹-Z¹-Y¹

wherein G¹ represents a divalent linking group, such as a substituted or unsubstituted alkylene, alkenylene, alkynylene or arylene group, SO₂, or a divalent heterocyclic group; Z¹ represents an atom or S, Se or Te; Y¹ represents a hydrogen atom, or a counter ion necessary in dissociation of Z¹ such as a sodium, potassium, lithium or ammonium ion.

The groups of formulae (X-2a) and (X-2b) have a 5- to 7-memberfed hetero ring or unsaturated ring. Za represents an atom of O, N, S, Se or Te; n¹ indicates an integer of from 0 to 3; and Y² represents a hydrogen atom, an alkyl group, an alkenyl group, an alkynyl group, or an aryl group.

General Formula (X-3) -Y³-(Z²)n²-Y⁴

wherein Z² represents an atom of S, Se or Te; n² indicates an integer of from 1 to 3; Y³ represents a divalent linking group, such as an alkylene group, an alkenylene group, an alkynylene group, an arylene group, or a divalent heterocyclic group; and Y⁴ represents an alkyl group, an aryl group, or a heterocyclic group. wherein Y⁵ and Y⁶ each independently represent an alkyl group, an alkenyl group, an arylene group, or a heterocyclic group. wherein Z³ represents an atom of S, Se or Te; E¹ represents a hydrogen atom, NH₂, NHY¹⁰, N(Y¹⁰)₂, NHN(Y¹⁰)₂, OY¹⁰ or SY¹⁰; E² represents a divalent linking group such as NH, NY¹⁰, NHNY¹⁰, O or S; Y⁷, Y⁸ and Y⁹ each independently represent a hydrogen atom, an alkyl group, an alkenyl group, an aryl group, or a heterocyclic group; Y⁸ and Y⁹ may be bonded to each other to form a ring; Y¹⁰ represents a hydrogen atom, an alkyl group, an alkenyl group, an aryl group, or a heterocyclic group. wherein Y¹¹ represents a divalent linking group such as an alkylene group, an alkenylene group, an alkynylene group, an arylene group or a divalent heterocyclic group; G² and J each independently represent COOY¹², SO₂Y¹², COY¹², SOY¹², CN, CHO or NO₂; and Y¹² represents an alkyl group, an alkenyl group, or an aryl group.

Formula (X-1) is described in detail. In the formula, the linking group for G¹ includes, for example, a substituted or unsubstituted, linear or branched alkylene group having from 1 to 20 carbon atoms (e.g., methylene, ethylene, trimethylene, propylene, tetramethylene, hexamethylene, 3-oxapentylene, 2-hydroxyrimethylene), a substituted or unsubstituted cyclic alkylene group having from 3 to 18 carbon atoms (e.g., cyclopropylene, cyclopentylene, cyclohexylene), a substituted or unsubstituted alkenylene group having from 2 to 20 carbon atoms (e.g., ethene, 2-butenylene) an alkynylene group having from 2 to 10 carbon atoms (e.g., ethynylene), a substituted or unsubstituted arylene group having from 6 to 20 carbon atoms (e.g., unsubstituted p-phenylene, unsubstituted 2,5-naphthylene).

The group SO₂ for G¹ in the formula may be -SO₂- alone, but including -SO₂- bonded to a substituted or unsubstituted, linear or branched alkylene group having from 1 to 10 carbon atoms, a substituted or unsubstituted cyclic alkylene group having from 3 to 6 carbon atoms, or an alkenylene group having from 2 to 10 carbon atoms.

The divalent heterocyclic group for G¹ in the formula includes may be unsubstituted or substituted with an alkylene group, an alkenylene group, an arylene group or a heterocyclic group, or may be benzo-condensed or naphtho-condensed (e.g., 2,3-tetrazole-diyl, 1,3-triazole-diyl, 1,2-imidazole-diyl, 3,5-oxadiazole-diyl, 2,4-thiadiazole-diyl, 1,5-benzimidazole-diyl, 2,5-benzothiazole-diyl, 2,5-benzoxazole-diyl, 2,5-pyrimidine-diyl, 3-phenyl-2,5-tetrazole-diyl, 2,5-pyridine-diyl, 2,4-furan-diyl, 1,3-piperidine-diyl, 2,4-morpholine-diyl).

In the formula, the alkylene group, the alkenylene group, the alkynylene group, the arylene group, the group SO₂ or the divalent heterocyclic group for G¹ may be substituted. Examples of the substituent by which the groups may be substituted are mentioned below. The substituent mentioned below is herein referred to as "substituent Y".

The substituent includes, for example, a halogen atom (e.g., fluorine, chlorine, bromine), an alkyl group (e.g., methyl, ethyl, isopropyl, n-propyl, tert-butyl), an alkenyl group (e.g., allyl, 2-butenyl), an alkynyl group (e.g., propargyl), an aralkyl group (e.g., benzyl), an aryl group (e.g., phenyl, naphthyl, 4-methylphenyl), a heterocyclic group (e.g., pyridyl, furyl, imidazolyl, piperidinyl, morpholyl), an alkoxy group (e.g., methoxy, ethoxy, butoxy, 2-ethylhexyloxy, ethoxyethoxy, methoxyethoxy), an aryloxy group (e.g., phenoxy, 2-naphthyloxy), an amino group (e.g., unsubstituted amino, dimethylamino, diethylamino, dipropylamino, dibutylamino, ethylamino, anilino), an acylamino group (e.g., acetylamino, benzoylamino), an ureido group (e.g., unsubstituted ureido, N-mcthylureido), an urethane group (e.g., methoxycarbonylamino, phenoxycarbonylamino), a sulfonylamino group (e.g., methylsulfonylamino, phenylsulfonylamino), a sulfamoyl group (e.g., unsubstituted sulfamoyl, N,N-dimethylsulfamoyl, N-phenylsulfamoyl), a carbamoyl group (e.g., unsubstituted carbamoyl, N,N-diethylcarbamoyl, N-phenylcarbamoyl), a sulfonyl group (e.g., mesyl, tosyl), a sulfinyl group (e.g., methylsulfinyl, phenylsulfinyl), an alkyloxycarbonyl group (e.g., methoxycarbonyl, ethoxycarbonyl), an aryloxycarbonyl group (e.g., phenoxycarbonyl), an acyl group (e.g., acetyl, benzoyl, formyl, pivaloyl), an acyloxy group (e.g., acetoxy, benzoyloxy), a phosphoramido group (e.g., N,N-diethylphosphoramido), a cyano group, a sulfo group, a thiosulfonyl group, a sulfinyl group, a carboxyl group, a hydroxyl group, a phosphono group, a nitro group, an ammonio group, a phosphonio group, a hydrazino group, a thiazolino group. In case where the group has two or more substituents, they may be the same or different. The substituents for these groups may be further substituted.

Preferred examples of formula (X-1) are mentioned below.

Preferably in formula (X-1), G¹ is a substituted or unsubstituted arylene group having from 6 to 10 carbon atoms, or a 5- to 7-membered heterocyclic group that is unsubstituted or bonded to an alkylene or arylene group, or is benzo-condensed or naphtho-condensed; Z¹ is S or Se; and Y¹ is a hydrogen atom or a sodium or potassium ion.

More preferably, G¹ is a substituted or unsubstituted arylene group having from 6 to 8 carbon atoms, o a 5- or 6-membefred heterocyclic group that is bonded to an arylene group or is benzo-coridensed. Most preferably, it is a 5- or 6-membered heterocyclic group that is bonded to an arylene group or is benzo-condensed. Even more preferably, Z¹ is S, and Y¹ is a hydrogen atom or a sodium ion.

Formulae (X-2a) and (X-2b) are described in detail.

The alkyl group, the alkenyl group and the alkynyl group for Y² in the formula include, for example, a substituted or unsubstituted, linear or branched alkyl group having from 1 to 10 carbon atoms (e.g., methyl, ethyl, isopropyl, n-propyl, n-butyl, tert-butyl, 2-pentyl, n-hexyl, n-octyl, tert-octyl, 2-ethylhexyl, 2-hydroxyethyl, 1-hydroxyethyl, diethylaminoethyl, n-butoxypropyl, methoxymethyl), a substituted or unsubstituted cyclic alkyl group having from 3 to 6 carbon atoms (e.g., cyclopropyl, cyclopentyl, cyclohexyl), an alkenyl group having from 2 to 10 carbon atoms (e.g., allyl, 2-butenyl, 3-pentenyl), an alkynyl group having from 2 to 10 carbon atoms (e.g., propargyl, 3-pentynyl), an aralkyl group having from 6 to 12 carbon atoms (e.g., benzyl). The aryl group for it is, for example, a substituted or unsubstituted aryl group having from 6 to 12 carbon atoms (e.g., hydroxyphenyl, 4-methylhydroxyphenyl).

Y² may be substituted with any of the substituents Y.

Preferred examples of formulae (X-2a) and (X-2b) are mentioned below.

Preferably in the formulae, Y² is a hydrogen atom, a substituted or unsubstituted alkyl group having from 1 to 6 carbon atoms, or a substituted or unsubstituted aryl group having from 6 to 10 carbon atoms; Za is O, N or S; and n¹ is from 1 to 3.

More preferably, Y² is a hydrogen atom or an alkyl group having from 1 to 4 carbon atoms; Za is N or S; and n¹ is 2 or 3.

Formula (X-3) is described in detail.

The linking group for Y³ in the formula includes, for example, a substituted or unsubstituted, linear or branched alkylene group having from 1 to 20 carbon atoms (e.g., methylene, ethylene, trimethylene, isopropylene, tetramethylene, hexamethylene, 3-oxapentylene, 2-hydroxytrimethylene), a substituted or unsubstituted cyclic alkylene group having from 3 to 18 carbon atoms (e.g., cyclopropylene, cyclopentylene, cyclohexylene), a substituted or unsubstituted alkenylene group having from 2 to 20 carbon atoms (e.g., ethene, 2-butenylene), an alkynylene group having from 2 to 10 carbon atoms (e.g., ethynylene), a substituted or unsubstituted arylene group having from 6 to 20 carbon atoms (e.g., unsubstituted p-phenylene, unsubstituted 2,5-naphthylene). The heterocyclic group for it may be unsubstituted or substituted with an alkylene group, alkenylene group or an arylene group, or further with an additional heterocyclic group (e.g., 2,5-pyridine-diyl, 3-phenyl-2,5-pyridine-diyl, 1,3-piperidine-diyl, 2,4-morpholine-diyl).

The alkyl group for Y⁴ in the formula includes, for example, a substituted or unsubstituted, linear or branched alkyl group having from 1 to 10 carbon atoms (e.g., methyl, ethyl, isopropyl, n-propyl, n-butyl, tert-butyl, 2-penthyl, n-hexyl, n-octyl, tert-octyl, 2-ethylhexyl, 2-hydroxyethyl, 1-hydroxyethyl, diethylaminoethyl, dibutylaminoethyl, n-butoxymethyl, methoxymethyl), a substituted or unsubstituted cyclic alkyl group having from 3 to 6 carbon atoms (e.g., cyclopropyl, cyclopentyl, cyclohexyl). The aryl group for it is, for example, a substituted or unsubstituted aryl group having from 6 to 12 carbon atoms (e.g., unsubstituted phenyl, 2-methylphenyl).

The heterocyclic group for it may be unsubstituted or substituted with an alkyl group, an alkenyl group or an aryl group or further with an additional heterocyclic group (e.g., pyridyl, 3-phenylpyridyl, piperidyl, morpholyl).

Y⁴ may be substituted with any of the substituents Y.

Preferred examples of formula (X-3) are mentioned below.

Preferably in the formula, Y³ is a substituted or unsubstituted alkylene group having from 1 to 6 carbon atoms, or a substituted or unsubstituted arylene group having from 6 to 10 carbon atoms; Y⁴ is a substituted or unsubstituted alkyl group having from 1 to 6 carbon atoms, or a substituted or unsubstituted aryl group having from 6 to 10 carbon atoms; Z² is S or Se; and n² is 1 or 2.

More preferably, Y³ is an alkylene group having from 1 to 4 carbon atoms; Y⁴ is an alkyl group having from 1 to 4 carbon atoms; Z² is S; and n² is 1.

Next described in detail is formula X-4).

In the formula, the alkyl group and the alkenyl group for Y⁵ and Y⁶ include, for example, a substituted or unsubstituted, linear or branched alkyl group having from 1 to 10 carbon atoms (e.g., methyl, ethyl, isopropyl, n-propyl, n-butyl, tert-butyl, 2-pentyl, n-hexyl, n-octyl, tert-octyl, 2-ethylhexyl, hydroxymethyl, 2-hydroxyethyl, 1-hydroxyethyl, diethylaminoethyl, dibutylaminoethyl, n-butoxymethyl, n-butoxypropyl, methoxymethyl), a substituted or unsubstituted cyclic alkyl group having from 3 to 6 carbon atoms (e.g., cyclopropyl, cyclopentyl, cyclohexyl), and an alkenyl group having from 2 to 10 carbon atoms (e.g., allyl, 2-butenyl, 3-pentenyl). The aryl group for them may be, for example, a substituted or unsubstituted aryl group having from 6 to 12 carbon atoms (e.g., unsubstituted phenyl, 4-methylphenyl); and the heterocyclic group may be unsubstituted or substituted with any of an alkylene group, an alkenylene group, an arylene group and an additional heterocyclic group (e.g., pyridyl, 3-phenylpyridyl, furyl, piperidyl, morpholino).

In the formula, Y⁵ and Y⁶ may be substituted with any of the substituents Y.

Preferred examples of formula (X-4) are mentioned below.

Preferably in the formula, Y⁵ and Y⁶ each are a substituted or unsubstituted alkyl group having from 1 to 6 carbon atoms, or a substituted or unsubstituted aryl group having from 6 to 10 carbon atoms.

More preferably, Y⁵ and Y⁶ each are an aryl group having from 6 to 8 carbon atoms.

Formulae (X-5a) and (X-5b) are described in detail. In these formulae, the group E¹ includes, for example, NH₂, NHCH₃, NHC₂H₅, NHPh, N(CH₃)₂, N(Ph)₂, NHNHC₃H₇, NHNHPh, OC₄H₉, OPh and SCH₃; and E² includes, for example, NH, NCH₃, NC₂H₅, NPh, NHNC₃H₇, and NHNPh. "Ph" herein indicates a phenyl group.

In formulae (X-5a) and (X-5b), the alkyl group and the alkenyl group for Y⁷, Y⁸ and Y⁹ include, for example, a substituted or unsubstituted, linear or branched alkyl group having from 1 to 10 carbon atoms (e.g., methyl, ethyl, isopropyl, n-propyl, n-butyl, tert-butyl, 2-pentyl, n-hexyl, n-octyl, tert-octyl, 2-ethylhexyl, hydroxymethyl, 2-hydroxyethyl, 1-hydroxyethyl, diethylaminoethyl, dibutylaminoethyl, n-butoxymethyl, n-butoxypropyl, methoxymethyl), a substituted or unsubstituted cyclic alkyl group having from 3 to 6 carbon atoms (e.g., cyclopropyl, cyclopentyl, cyclohexyl), and an alkenyl group having from 2 to 10 carbon atoms (e.g., allyl, 2-butenyl, 3-pentenyl). The aryl group for them may be, for example, a substituted or unsubstituted aryl group having from 6 to 12 carbon atoms (e.g., unsubstituted phenyl, 4-methylphenyl). The heterocyclic group for them may be unsubstituted or substituted with any of an alkylene group, an alkenylene group, an arylene group and an additional heterocyclic group (e.g., pyridyl, 3-phenylpyridyl, furyl, piperidyl, morpholyl).

In the formulae, Y⁷, Y⁸ and Y⁹ may be substituted with any of the substituents Y.

Preferred examples of formulae (X-5a) and (X-5b) are mentioned below.

Preferably in these formulae, E¹ is an alkyl-substituted or unsubstituted amino or alkoxy group; E² is an alkyl-substituted or unsubstituted amino-linking group; Y⁷, Y⁸ and Y⁹ each are a substituted or unsubstituted alkyl group having group 1 to 6 carbon atoms, or a substituted or unsubstituted arylene group having from 6 to 10 carbon atoms; and Z³ is S or Se.

More preferably, E¹ is an alkyl-substituted or unsubstituted amino group; E² is an alkyl-substituted or unsubstituted amino-linking group; Y⁷, Y⁸ and Y⁹ each are a substituted or unsubstituted alkyl group having group 1 to 4 carbon atoms; and Z³ is S.

Formulae (X-6a) and (X-6b) are described in detail.

In these formulae, the groups G² and J include, for example, COOCH₃, COOC₃H₇, COOC₆H₁₃, COOPh, SO₂CH₃, SO₂C₄H₉, COC₂H₅, COPh, SOCH₃, SOPh, CN, CHO and NO₂.

In these formulae, the linking group for Y¹¹ includes, for example, a substituted or unsubstituted, linear or branched alkylene group having from 1 to 20 carbon atoms (e.g., methylene, ethylene, trimethylene, propylene, tetramethylene, hexamethylene, 3-oxapentylene, 2-hydroxytrimethylene), a substituted or unsubstituted cyclic alkylene group having from 3 to 18 carbon atoms (e.g., cyclopropylene, cyclopentylene, cyclohexylenc), a substituted or unsubstituted alkenylene group having from 2 to 20 carbon atoms (e.g., ethene, 2-butenylene), an alkynylene group having from 2 to 10 carbon atoms (e.g., ethynylene), and a substituted or unsubstituted arylene group having from 6 to 20 carbon atoms (e.g., unsubstituted p-phenylene, unsubstituted 2,5-naphthylene).

In these formulae, the divalent heterocyclic group for Y¹¹ may be unsubstituted or substituted with any of an alkylene group, an alkenylene group, an arylene group and an additional heterocyclic group (e.g., 2,5-pyridine-diyl, 3-phenyl-2,5-pyridine-diyl, 2,4-furan-diyl, 1,3-piperidine-diyl, 2,4-morpholine-diyl).

In these formulae, Y¹¹ may be substituted with any of the substituents Y.

Preferred examples of formulae (X-6a) and (X-6b) are mentioned below.

Preferably in these formulae, G² and J each are a carboxylate or carbonyl residue having from 2 to 6 carbon atom; and Y¹¹ is a substituted or unsubstituted alkylene group having from 1 to 6 carbon atoms, or a substituted or unsubstituted arylene group having from 6 to 10 carbon atoms.

More preferably, G² and J each are a carboxylate residue having from 2 to 4 carbon atom; and Y¹¹ is a substituted or unsubstituted alkylene group having from 1 to 4 carbon atoms, or a substituted or unsubstituted arylene group having from 6 to 8 carbon atoms.

The silver halide-adsorbing group for X is more preferably any of formulae (X-1), (X-2a), (X-2b), (X-3), (X-5a), (X-5b), (3i-4), (X-6a) and (X-6b) in that order.

The light-absorbing group for X in formula (I) is described in detail.

The light-absorbing'group for X in formula (I) may be represented, for example, by the following general formula: wherein Z⁴ represents an atomic group necessary for forming a 5- or 6-membered, nitrogen-containing hetero ring; L², L³, L⁴ and L⁵ each represent a methine group; p¹ indicates 0 or 1; n³ falls between O and 3; M¹ represents a charge-equilibrating counter ion; and m² indicates a number necessary for neutralizing the charge of the molecule, falling between 0 and 10.

In the formula, the 5- or 6-membered, nitrogen-containing hetero ring for Z⁴ includes, for example, thiazoline, thiazole, benzothiazole, oxazoline, oxazole, benzoxazole, selenazoline, selenazole, benzoselenazole, 3,3-dialkylindolenine (e.g., 3,3-dimethylindolenine), imidazoline, imidazole, benzimidazole, 2-pyridine, 4-pyridine, 2-quinoline, 4-quinoline, 1-isoquinoline, 3-isoquinoline, imidazo[4,5-b]quinoxaline, oxadiazole, thiadiazole, tetrazole and pyrimidine nuclei.

The 5- or 6-membered, nitrogen-containing hetero ring for Z⁴ may be substituted with any of the substituents Y.

In the formula, L², L³, L⁴ and L⁵ each independently represent a methine group. The methine group for L², L³, L⁴ and L⁵ may be substituted. The substituent includes, for example, a substituted or unsubstituted alkyl group having from 1 to 15 carbon atoms (e.g., methyl, ethyl, 2-carboxyethyl), a substituted or unsubstituted aryl group having from 6 to 20 carbon atoms (e.g., phenyl, o-carboxyphenyl), a substituted or unsubstituted heterocyclic group having from 3 to 20 carbon atoms (e.g., N,N-diethylbarbituric residue), a halogen atom (e.g., chlorine, bromine, fluorine, iodine), an alkoxy group having from 1 to 15 carbon atoms (e.g., methoxy, ethoxy), an alkylthio group having from 1 to 15 carbon atoms (e.g., methylthio, ethylthio), an arylthio group having from 6 to 20 carbon atoms (e.g., phenylthio), and an amino group having from 0 to 15 carbon atoms (e.g., N,N-diphenylamino, N-methyl-N-phenylamino, N-methylpiperazino).

The methine group for these may form a ring together with the other methine group, or may also form a ring together with the other part of the formula.

In the formula, M¹ indicates the presence of a cation or anion optionally necessary for neutralizing the ionic charge of the light-absorbing group. Typical examples of the cation are inorganic cations such as hydrogen ion (H⁺) and alkali metal ions (e.g., sodium ion, potassium ion, lithium ion); and organic cations such as ammonium ions (e.g., ammonium ion, tetraalkylammonium ions, pyridinium ion, ethylpyridinium ion). The anion may also be any of an inorganic anion or an organic anion, including, for example, halide ions (e.g., fluoride ion, chloride ion, iodide ion), substituted arylsulfonate ions (e.g., p-toluenesulfonate ion, p-chlorobenzenesulfonate ion), aryldisulfonate ions (e.g., 1,3-benzenedisulfonate ion, 1,5-naphthalenedisulfonate ion, 2,6-naphthalenedisulfonate ion), alkylsulfate ions (e.g., methylsulfate ion), sulfate ion, thiocyanate ion, perchlorate ion, tetrafluoroborate ion, picrate ion, acetate ion, and trifluoromethanesulfonate ion. For the light-absorbing group, also usable are ionic polymers or counter-charged groups.

In this description, the sulfo group is represented by SO₃⁻, and the carboxyl group is by CO₂⁻; and when the counter ion is a hydrogen ion, they may be represented by SO₃H and CO₂H, respectively.

In the formula, m² indicates a number necessary for neutralizing the charge of the molecule. In case where the group of the formula is to indicate an internal salt, m is O.

Preferred examples of formula (X-7) are mentioned below.

Preferably in formula (X-7), Z⁴ indicates a benzoxazole nucleus, a benzothiazole nucleus, a benzimidazole nucleus or a quinoline nucleus; L², L³, L⁴ and L⁵ each represent an unsubstituted methine group; p¹ is 0; and n³ is 1 or 2.

More preferably, Z⁴ indicates a benzoxazole nucleus or a benzothiazole nucleus, and n^{s} is 0. Even more preferably, Z⁴ is a benzothiazole nucleus.

In formula (I), k is preferably 0 or 1, more preferably 1.

Examples of X in formula (I) are mentioned below, to which, however, X employable in the first embodiment of the invention is not limited.

The linking group for L in formula (I) is described in detail.

The linking group for L in formula (I) includes, for example, a substituted or unsubstituted, linear or branched alkylene group having from 1 to 20 carbon atoms (e.g., methylene, ethylene, trimethylene, propylene, tetramethylene, hexamethylene, 3-oxapentylene, 2-hydroxytrimethylene), a substituted or unsubstituted cyclic alkylene group having from 3 to 18 carbon atoms (e.g., cyclopropylene, cyclopentylene, cyclohexylene), a substituted or unsubstituted alkenylene group having from 2 to 20 carbon atoms (e.g., ethene, 2-butenylene), an alkynylene group having from 2 to 10 carbon atoms (e.g., ethynylene), a substituted or unsubstituted arylene group having from 6 to 20 carbon atoms (e.g., unsubstituted p-phenylene, unsubstituted 2,5-naphthylene), a heterocyclic linking group (e.g., 2,6-pyridine-diyl), a carbonyl group, a thiocarbonyl group, an imido group, a sulfonyl group, a sulfonyloxy group, an ester group, a thioester group, an amido group, an ether group, a thioether group, an amino group, an ureido group, a thioureido group, a thiosulfonyl group. These linking groups may be bonded to each other to form linking groups of different types.

L may be substituted with any of the substituents Y.

Preferably, the linking group L is an unsubstituted alkylene group having from 1 to 10 carbon atoms, or an alkylene group having from 1 to 10 carbon atoms and bonded to any of an amino group, an amido group, a thioether group, an ureido group or a sulfonyl group. More preferably, it is an unsubstituted alkylene group having from 1 to 6 carbon atoms, or an alkylene group having from 1 to 6 carbon atoms and bonded to any of an amino group, an amido group or a thioether group.

In formula (I), m is preferably 0 or 1, more preferably 1.

The electron-donating group A is described in detail.

In formula (I), the moiety (A - B) is, after oxidized or fragmented, releases an electron to form a radical A·, and the radical A· is then oxidized to release an electron. The reaction process to enhance the sensitivity of the photothermographic material of the invention is shown below. ${{A - B}_{\left({E}^{1}\right)}}_{0 ∼ 1.5 ⁢ V} ⁢ {\to }^{- {e}^{-}} A ⁢ {{\overline{ }}_{ }}^{\cdot +} ⁢ B \to {A}^{\cdot } ⁢ \left(+{B}^{+}\right) {\to }^{- {e}^{-}} {{{A}^{+}}_{\left({E}^{2}\right)}}_{≦ - 0.6 ⁢ V}$

In the compound of formula (I), A is electron-donating group. Preferably, therefore, the compound is so designed that the substituents on the aromatic group of any structure therein satisfy the electron-rich condition of A therein. For example, in case where the aromatic ring in the compound does not satisfy the electron-rich condition of A, it is desirable to introduce an electron-donating group into it; but on the contrary, in case where the aromatic ring has too many electrons like anthracene, it is desirable to introduce an electron-attracting group into it. In any case, it is desirable that the oxidation potential of the compound is well controlled in that manner.

Preferably, the group A is represented by any of the following general formulae (A-1), (A-2) and (A-3):

In formulae (A-1) and (A-2), Y¹², Y^{12'}, Y¹³ and Y^{13'} each independently represent a hydrogen atom, or a substituted or unsubstituted alkyl, aryl, alkylene or arylene group; Y¹⁴ and Y^{14'} each independently represent an alkyl group, COOH, a halogen atom, N(Y¹⁵)₂, OY¹⁵, SY¹⁵, CHO, COY¹⁵, COOY¹⁵, CONHY¹⁵, CON(Y¹⁵)₂, SO₃Y¹⁵, SO₂NHY¹⁵, SO₂NY¹⁵, SO₂Y¹⁵, SOY¹⁵, or CSY¹⁵; Ar¹ and Ar^{1'} each independently represent an aryl group or a heterocyclic group; Y¹² and Y¹³, Y¹² and Ar¹, Y^{12'} and Y^{13'}, and Y^{12'} and Ar^{1'} may be bonded to each other to form a ring; Q² and Q^{2'} each independently represent O, S, Se or Te; m³ and m⁴ each independently indicate 0 or 1; n⁴ falls between 1 and 3; L² represents N-R, N-Ar, O, S or Se, optionally having a 5- to 7-membered hetero ring or unsaturated ring; and Y¹⁵ represents a hydrogen atom, an alkyl group or an aryl group. The cyclic structure of formula (A-3) indicates a substituted or unsubstituted, 5- to 7-membered unsaturated ring or hetero ring.

Formulae (A-1), (A-2) and (A-3) are described in detail. In these formulae, the alkyl group for Y¹², Y^{12'}, Y¹³ and Y^{13'} includes, for example, a substituted or unsubstituted, linear or branched alkyl group having from 1 to 10 carbon atoms (e.g., methyl, ethyl, isopropyl, n-propyl, n-butyl, tert-butyl, 2-pentyl, n-hexyl n-octyl, tert-octyl, 2-ethylhexyl, 2-hydroxyethyl, 1-hydroxyethyl, diethylaminoethyl, dibutylaminoethyl, n-butoxymethyl, methoxymethyl), a substituted or unsubstituted cyclic alkyl group having from 3 to 6 carbon atoms (e.g., cyclopropyl, cyclopentyl, cyclohexyl). The aryl group for them may be, for example, a substituted or unsubstituted aryl group having from 6 to 12 carbon atoms (e.g., unsubstituted phenyl, 2-methylphenyl).

The alkylene group may be, for example, a substituted or unsubstituted, linear or branched alkylene group having from 1 to 10 carbon atoms (e.g., methylene, ethylene, trimethylene, tetramethylene, methoxyethylene); and the arylene group may be, for example, a substituted or unsubstituted arylene group having from 6 to 12 carbon atoms (e.g., unsubstituted phenylene, 2-methylphenylene, naphthylene).

In formulae (A-1) and (A-2), the groups Y¹⁴ and Y^{14'} include, for example, an alkyl group (e.g., methyl, ethyl, isopropyl, n-propyl, n-butyl, 2-pentyl, n-hexyl, n-octyl, 2-ethylhexyl, 2-hydroxyethyl, n-butoxymethyl), COOH, a halogen atom (e.g., fluorine, chlorine, bromine), OH, N(CH₃)₂, NPh₂, OCH₃, OPh, SCH₃, SPh, CHO, COCH₃, COPh, COOC₄H₉, COOCH₃, CONHC₂H₅, CON(CH₃)₂, SO₃CH₃, SO₃C₃H₇, SO₂NHCH₃, SO₂N(CH₃)₂, SO₂C₂H₅, SOCH₃, CSPh, CSCH₃.

Ar¹ and Ar^{1'} in formulae (A-1) and (A-2) include, for example, a substituted or unsubstituted aryl group having from 6 to 12 carbon atoms (e.g., phenyl, 2-methylphenyl, naphthyl), and a substituted or unsubstituted heterocyclic group (e.g., pyridyl, 3-phenylpyridyl, piperidyl, morpholyl).

L² in formulae (A-1) and (A-2) include, for example, NH, NCH₃, NC₄H₉, NC₃H₇(i), NPh, NPh-CH₃, O, S, Se, Te.

The cyclic structure of formula (A-3) includes an unsaturated 5- to 7-membered ring and a hetero ring (e.g., furyl, piperidyl, morpholyl).

Y¹², Y¹³, Y¹⁴, Ar¹, L², y^{12'}, Y^{13'}, Y^{14'}, Ar^{1'} in formulae (A-1) and (A-2), and the cyclic structure of formula (A-3) may be substituted with any of the substituents Y.

Preferred examples of formulae (A-1), (A-2) and (A-3) are mentioned below.

Preferably in formulae (A-1) and (A-2), Y¹², Y^{12'}, Y¹³ and Y^{13'} each independently represent a substituted or unsubstituted alkyl or alkylene group having from 1 to 6 carbon atoms, or a substituted or unsubstituted aryl group having from 6 to 10 carbon atoms; Y¹⁴ and Y^{14'} each are a substituted or unsubstituted alkyl group having from 1 to 6 carbon atoms, an amino group mono- or di-substituted with alkyl group(s) having from 1 to 4 carbon atoms, a carboxyl group, a halogen atom, or a carboxylate residue having from 1 to 4 carbon atoms; Ar¹ and Ar^{1'} each are a substituted or unsubstituted aryl group having from 6 to 10 carbon atoms; Q² and Q^{2'} each are O, S or Se; m³ and m⁴ each are 0 or 1; n⁴ falls between 1 and 3; and L² is an alkyl-substituted amino group having from 0 to 3 carbon atoms.

Preferably, the cyclic structure of formula (A-3) is a 5- to 7-membered hetero ring.

More preferably in formulae (A-1) and (A-2), Y¹², Y^{12'}, Y¹³ and Y^{13'} each independently represent a substituted or unsubstituted alkyl or alkylene group having from 1 to 4 carbon atoms; Y¹⁴ and Y^{14'} each are an unsubstituted alkyl group having from 1 to 4 carbon atoms, or a monoamino-substituted or diamino-substituted alkyl group having from 1 to 4 carbon atoms; Ar¹ and Ar^{1'} each are a substituted or unsubstituted aryl group having from 6 to 10 carbon atoms; Q² and Q^{2'} each are O or S; m³ and m⁴ are both 0; n⁴ is 1; and L² is an alkyl-substituted amino group having from 0 to 3 carbon atoms.

Also more preferably, the cyclic structure of formula (A-3) is a 5- or 6-membered hetero ring.

In formula (I), when X is represented by any of formula (A-1) or (A-2), the moiety of A bonding to X or L is selected from Y¹², Y¹³, Ar¹, Y^{12'}, Y^{13'} and Ar^{1'}.

Examples of A in formula (I) are mentioned below, to which, however, A employable in the first embodiment of the invention is not limited.

B in formula (I) is described in detail.

In case where B is a hydrogen atom, the compound of formula (I) is, after oxidized, deprotonated by the internal base to give a radical A·.

Preferably, B is a hydrogen atom or a group represented by any of the following general formulae (B-1), (B-2) and (B-3):

In formulae (B-1), (B-2) and (B-3), W represents Si, Sn or Ge; each Y¹⁶ independently represents an alkyl group; and each Ar² independently represents an aryl group.

The group of formula (B-2) or (B-3) may be bonded to the adsorbing group X in formula (I).

Formulae (B-1), (B-2) and (B-3) are described in detail. In these formulae, the alkyl group for Y¹⁶ includes, for example, a substituted or unsubstituted, linear or branched alkyl group having from 1 to 6 carbon atoms (e.g., methyl, ethyl, isopropyl, n-propyl, n-butyl, tert-butyl, 2-pentyl, n-hexyl, n-octyl, tert-octyl, 2-ethylhexyl, 2-hydroxyethyl, 1-hydroxyethyl, n-butoxyethyl, methoxymethyl), and a substituted or unsubstituted aryl group having from 6 to 12 carbon atoms (e.g., phenyl, 2-methylphenyl).

Y¹⁶ and Ar² in formulae (B-1), (B-2) and (B-3) may be substituted with any of the substituents Y.

Preferred examples of formulae (B-1), (B-2) and (B-3) are mentioned below.

Preferably in formulae (B-2) and (B-3), Y¹⁶ is a substituted or unsubstituted alkyl group having from 1 to 4 carbon atoms; Ar² is a substituted or unsubstituted aryl group having from 6 to 10 carbon atoms; and W is Si or Sn.

More preferably in formulae (B-2) and (B-3), Y¹⁶ is a substituted or unsubstituted alkyl group having from 1 to 3 carbon atoms; Ar² is a substituted or unsubstituted aryl group having from 6 to 8 carbon atoms; and W is.

Of formulae (B-1), (B-2) and (B-3), most preferred are COO- of formula (B-1), and Si-(Y¹⁶)₃ of formula (B-2).

Preferably in formula (1), n is 1.

Examples of (A-B) in formula (I) are mentioned below, to which, however, (A-B) employable in the first embodiment of the invention is not limited.

The counter ion necessary for the charge balance of (A-B) in formula (I) includes, for example, sodium, potassium, triethylammonium, diisopropylammonium, tetrabutylammonium and tetramethylguanidinium ions.

Preferably, the oxidation potential of (A-B) falls between 0 and 1.5 V, more preferably between 0 and 1.0 V, even more preferably between 0.3 and 1.0 V.

Also preferably, the oxidation potential of the radical A·(E₂) resulting from the bond cleavage reaction falls between -0.6 and -2.5 V, more preferably between -0.9 and -2 V, even more preferably between -0.9 and -1.6 V.

The oxidation potential may be measured as follows:
E¹ may be measured through cyclic voltammetry. Concretely, the electron donor A is dissolved in a solution of water 80 %/20 % (by volume) that contains acetonitrile/0.1 M lithium perchlorate. A glassy carbon disc is used for the working electrode; a platinum wire is for the counter electrode; and a saturated calomel electrode (SCE) is for the reference electrode. At 25°C, this is measured at a potential scanning speed of 0.1 V/sec. The ratio of oxidation potential/SCE is read at the peak of the cyclic voltammetric curve. The value E¹ of the compound (A-B) is described in EP 93,731A1.

The oxidation potential of the radical is measured through transitional electrochemical and pulse-radiation decomposition. This is reported in J. Am. Chem. Soc., 1988, 110, 132; ibid., 1974, 96, 1287; and ibid., 1974, 96, 1295.

Examples of the compound of formula (I) are mentioned below, to which, however, the compounds employable in the first embodiment of the invention are not limited.

For their production, the compounds of formula (I) may be produced according to the methods described in, for example, USP 5,747,235, 5,747,235, EP 786,692A1, 893,731A1, 893,732A1, and WO99/05570, or according to those similar to the methods.

In producing the photothermographic material of the first embodiment of the invention, the compound of formula (I) may be added to the material in any stage, for example, while the coating emulsion for the material is prepared, or while the material is produced. Concretely, it may be added in any step of grain formation, de-salting or chemical sensitization, or even prior to emulsion coating. In these steps, the compound may be added twice or more.

Preferably, the compound of formula (I) is added, after dissolved in water or a water-soluble solvent such as methanol or ethanol or in a mixed solvent of these. In case where the compound is dissolved in water, the pH of the solution may be high for the compounds having a higher degree of solubility in water at a higher pH. In that case, however, the pH of the solution may be lowered for the compounds having a higher degree of solubility in water at a lower pH.

Preferably, the compound of formula (I) is in the image-forming layer (emulsion layer) of the photothermographic material. If desired, it may also be in the protective layer and/or the interlayer of the material so that the compound may diffuse in the image-forming layer while the layers are formed. The time for adding the compound of formula (I) is not specifically defined, irrespective of before and after addition of a sensitizing dye to the image-forming layer. Preferably, the compound of formula (I) is added to the silver halide-containing image-forming layer of the material, and its amount falls between 1 × 10⁻⁹ and 5 × 10⁻¹ mols, more preferably between 1 × 10⁻⁸ and 2 × 10⁻¹ mols per mol of the silver halide in the layer. <*Photosensitive Silver Halide*>

The photosensitive silver halide for use in the first embodiment of the invention is described in detail.

### <<Halogen Composition>>

Preferably, the mean silver iodide content of the photosensitive silver halide for use in the first embodiment of the invention falls between 5 and 100 mol%, more preferably between 10 and 100 mol%, even more preferably between 70 and 100 mol%, most preferably between 90 and 100 mol%.

Regarding the halogen composition distribution in each silver halide grain, the composition may be uniform throughout the grain, or may stepwise vary, or may continuously vary. Core/shell structured silver halide grains are also preferred for use herein. Preferably, the core/shell structure of the grains has from 2 to 5 layers, more preferably from 2 to 4 layers.

Solid solution of halogen compositions other than iodine is limited. However, the iodine content of core/ shell structured silver halide grains as above or of conjugate structured silver halide grains can be controlled in any desired manner.

Preferably, the photosensitive silver halide in the first embodiment of the invention has a direct transition absorption derived from the silver iodide crystal structure therein, in a wavelength range of from 350 nm to 450 nm. Silver halides having such a direct transition for light absorption can be readily differentiated from any others by analyzing them as to whether to not they show an exciton absorption caused by their direction transition at around 400 nm to 430 nm.

The high silver iodide phase of such a type of direct transition light absorption may exist alone in the silver halide emulsion for use herein, but may be conjugated with any other silver halide phase having an indirect transition absorption in a wavelength range of from 350 nm to 450 nm, for example, with silver bromide, silver chloride, silver bromoiodide, silver chloroiodide or their mixed crystals. Any of these are preferred for use herein.

As so mentioned above, the silver halide grains for use herein may preferably have a core/shell structure. Also preferably, the grains may have an amorphous structure through iodine ion conversion.

In any case, it is desirable that the halogen composition of the silver halide grains has a total silver iodide content of from 5 to 100 mol%. More preferably, the silver iodide content of the grains falls between 10 and 100 mol%, even more preferably between 40 and 100 mol%, still more preferably between 70 and 100 mol%, most preferably between 90 and 100 mol%.

The silver halide phase of the type of direct transition light absorption generally absorbs much light, but as compared with other silver halide phases of the other type of indirect transition light absorption that absorb only a little light, its sensitivity is low and therefore its industrial use has not heretofore been taken into much consideration.

We, the present inventors have found that, when the silver halide phase of that type of direct transition light absorption is combined with at least one compound of formula (I), then its sensitivity is increased. On the basis of this finding, we have completed the first embodiment of the invention.

### <<Grain Size>>

More preferably, the photosensitive silver halide in the first embodiment of the invention has a mean grain size of from 5 nm to 80 nm for more effectively attaining its effect. We, the present inventors have found that, especially when the silver halide grains having the phase that has a direct transition absorption have a grain size of not larger than 80 nm and are small, then their sensitivity is more increased.

Even more preferably, the mean grain size of the photosensitive silver halide falls between 5 nm and 70 nm, still more preferably between 10 nm and 50 nm. The grain size referred to herein is meant to indicate the diameter of the circular image having the same area as the projected area of each silver halide grain (for tabular grains, the main face of each grain is projected to determine the projected area of the grain). The data of all the silver halide grains thus analyzed are averaged to obtain the mean grain size thereof. The mean grain size may be hereinafter referred to simply as "grain size".

### <<Method of Forming Grains>>

Methods of forming the photosensitive silver halide are well known in the art, for example, as in Research Disclosure 17029 (June 1978), and USP 3,700,458, and any known method is employable in the invention. Concretely, a silver source compound and a halogen source compound are added to gelatin or any other polymer solution to prepare a photosensitive silver halide, and it is then mixed with an organic silver salt. This method is preferred for the invention. Also preferred are the method described in JP-A 119374/ 1999, paragraphs [0217] to [0244]; and the methods described in JP-A 11-352627 and 2000-347335.

### <<Grain Morphology>>

Silver halide grains generally have different types of morphology, including, for example, cubic grains, octahedral grains, tabular grains, spherical grains, rod-like grains, and potato-like grains. In the first embodiment of the invention, cubic silver halide grains are especially preferred. Also preferred are corner-rounded silver halide grains. The surface index (Miller index) of the outer surface of the photosensitive silver halide grains for use herein is not specifically defined, but is desirably such that the proportion of {100} plane, which ensures higher spectral sensitization when it has adsorbed a color-sensitizing dye, in the outer surface is larger. Preferably, the proportion of {100} plane in the outer surface is at least 50 %, more preferably at least 65 %, even more preferably at least 80 %. The Miller index indicated by the proportion of {100} plane can be identified according to the method described by T. Tani in J. Imaging Sci., 29, 165 (1985), based on the adsorption dependency of sensitizing dye onto {111} plane and {100} plane.

### <<Heavy Metal>>

In the first embodiment of the invention, preferred are silver halide grains having a hexacyano-metal complex in their outermost surface. Preferred examples of the hexacyano-metal complex are [Fe(CN)₆]⁴⁻, [Fe(CN)₆]³⁻, [Ru(CN)₆]⁴⁻, [Os(CN)₆]⁴⁻, [Co(CN)₆]³⁻, [Rh(CN)_{6]}³⁻, [Ir(CN)₆]³⁻, [Cr(CN)₆]³⁻, [Re(CN)₆]³⁻. Of those, hexacyano-Fe complexes are more preferred in the first embodiment of the invention.

As hexacyano-metal complexes exist in the form of ions in their aqueous solutions, their counter cations are of no importance. Preferably, however, the counter cations for the complexes are any of alkali metal ions such as sodium, potassium, rubidium, cesium and lithium ions; ammonium ions, and alkylammonium ions (e.g., tetramethylammonium, tetraethylammonium, tetrapropylammonium and tetra(n-butyl)ammonium ions), as they are well miscible with water and are favorable to the operation of precipitating silver halide emulsions.

The hexacyano-metal complex may be added to silver halide grains in the form of a solution thereof in water or in a mixed solvent of water and an organic solvent miscible with water (for example, alcohols, ethers, glycols, ketones, esters, amides), or in the form of a mixture thereof with gelatin.

The amount of the hexacyano-metal complex to be added to the silver halide grains preferably falls between 1 × 10⁻⁵ mols and 1 × 10⁻² mols, per mol of silver of the grains, more preferably between 1 × 10⁻⁴ mols and 1 × 10⁻³ mols.

In order to make the hexacyano-metal complex exist in the outermost surfaces of the silver halide grains, the complex is added to an aqueous silver nitrate solution from which are formed the silver halide grains, after the solution has been added to a reaction system to give the grains but before the grains having been formed are finished for chemical sensitization such as chalcogen sensitization with sulfur, selenium or tellurium or noble metal sensitization with gold or the like, or is directly added to the grains while they are rinsed or dispersed but before they are finished for such chemical sensitization. To prevent the silver halide grains formed from growing too much, it is desirable that the hexacyano-metal complex is added to the grains immediately after they are formed. Preferably, the complex is added thereto before the grains formed are finished for post-treatment.

Adding the hexacyano-metal complex to the silver halide grains may be started after 96 % by weight of the total of silver nitrate, from which are formed the grains, has been added to a reaction system to give the grains, but is preferably started after 98 % by weight of silver nitride has been added thereto, more preferably after 99 % by weight thereof has been added thereto.

The hexacyano-metal complex added to the silver halide grains after an aqueous solution of silver nitrate has been added to the reaction system to give the grains but just before the grains are completely formed is well adsorbed by the grains formed, and may well exist in the outermost surfaces of the grains. Most of the complex added in that manner forms a hardly-soluble salt with the silver ions existing in the surfaces of the grains. The silver salt of hexacyano-iron(II) is more hardly soluble than AgI, and the fine grains formed are prevented from re-dissolving and aggregating into large grains. Accordingly, the intended fine silver halide grains having a small grain size can be formed.

The photosensitive silver halide grains for use in the first embodiment of the invention may contain a metal or metal complex of Groups 8 to 10 of the Periodic Table (including Groups 1 to 18). The metal of Groups 8 to 10, or the center metal of the metal complex is preferably rhodium, ruthenium or iridium. In this embodiment, one metal complex may be used alone, or two or more metal complexes of one and the same type of metal or different types of metals may also be used as combined. The metal or metal complex content of the grains preferably falls between 1 × 10⁻⁹ mols and 1 × 10⁻³ mols per mol of silver of the grains. Such heavy metals and metal complexes, and methods of adding them to the silver halide grains are described in, for example, JP-A 7-225449, JP-A 11-65021, paragraphs [0018] to [0024], and JP-A 11-119374, paragraphs [0227] to [0240].

The metal atoms (e.g., in [Fe(CN)₆]⁴⁻) that may be added to the silver halide grains for use in the first embodiment of the invention, as well as the methods of desalting or chemical sensitization of the silver halide emulsions are described, for example, in JP-A 11-84574, paragraphs [0046] to [0050], JP-A 11-65021, paragraphs [0025] to [0031], and JP-A 11-119374, paragraphs [0242] to [0250].

### <<Gelatin>>

Gelatin of different types may be used in preparing the photosensitive silver halide emulsions for use in the first embodiment of the invention. For better dispersion of the photosensitive silver halide emulsion in an organic silver salt-containing coating liquid in producing the photothermographic material of the invention, preferred is low-molecular gelatin having a molecular weight of from 500 to 60,000. The low-molecular gelatin of the type may be used in forming the silver halide grains or in dispersing the grains after the grains have been desalted. Preferably, it is used in dispersing the grains after they have been desalted.

### <<Sensitizing Dye>>

The photothermographic material of the first embodiment of the invention may contain a sensitizing dye. Usable herein are sensitizing dyes which, after adsorbed by the silver halide grains, can spectrally sensitize the grains within a desired wavelength range. Depending on the spectral characteristics of the light source to be used for exposure, favorable sensitizing dyes having good spectral sensitivity are selected for use in the photothermographic material. For the details of sensitizing dyes usable herein and methods for adding them to the photothermographic material, referred to are paragraphs [0103] to [0109] in JP-A 11-65021; compounds of formula (II) in JP-A 10-186572; dyes of formula (I) and paragraph [0106] in JP-A 11-119374; dyes described in USP 5,510,236, 3,871,887 (Example 5); dyes described in JP-A 2-96131, 59-48753; from page 19, line 38 to page 20, line 35 in EP Laid-Open 0803764A1; Japanese Patent Application Nos. 2000-86865, 2000-102560 and 2000-205399. One or more such sensitizing dyes may be used herein either singly or as combined. Regarding the time at which the sensitizing dye is added to the silver halide emulsion in the invention, it is desirable that the sensitizing dye is added thereto after the desalting step but before the coating step, more preferably after the desalting step but before the chemical ripening step.

The amount of the sensitizing dye to be in the photothermographic material of the first embodiment of the invention varies, depending on the sensitivity and the fogging resistance of the material. In general, it preferably falls between 10⁻⁶ and 1 mol, more preferably between 10⁻⁴ and 10⁻¹ mols, per mol of the silver halide in the image-forming layer of the material.

For its better spectral sensitization, the photothermographic material of the first embodiment of the invention may contain a supersensitizer. For the supersensitizer, for example, usable are the compounds described in EP Laid-Open 587,338, USP 3,877,943, 4,873,184, and JP-A 5-341432, 11-109547 and 10-111543.

### <<Chemical Sensitization>>

Preferably, the photosensitive silver halide grains for use in the first embodiment of the invention are chemically sensitized with, for example, sulfur, selenium or tellurium. For such sulfur, selenium or tellurium sensitization, any known compounds are usable. For example, preferred are the compounds described in JP-A 7-128768. The grains for use in the first embodiment of the invention are especially preferably sensitized with tellurium, for which more preferred are the compounds described in JP-A 11-65021, paragraph [0030], and the compounds of formulae (II), (III) and (IV) given in JP-A 5-313284.

Preferably, the photosensitive silver halide grains for use in the first embodiment of the invention are chemically sensitized with gold alone or with gold combined with chalcogen. Gold in the gold sensitizer for them preferably has a valence of +1 or +3. Any ordinary gold compounds for gold sensitization are usable herein. Preferred examples of the gold sensitizer for use herein are chloroauric acid, bromoauric acid, potassium chloroaurate, potassium bromoaurate, auric trichloride, potassium auric thiocyanate, potassium iodoaurate, tetracyanoauric acid, ammonium aurothiocyanate, pyridyltrichlorogold. Also preferred for use herein are the gold sensitizers described in USP 5,858,637, and Japanese Patent Application No. 2001-79450.

In the first embodiment of the invention, the photosensitive silver halide grains may be chemically sensitized in any stage after their formation but before their coating. For example, they may be chemically sensitized after desalted, but (1) before spectral sensitization, or (2) along with spectral sensitization, or (3) after spectral sensitization, or (4) just before coating.

The amount of the sulfur, selenium or tellurium sensitizer for such chemical sensitization in the first embodiment of the invention varies, depending on the type of the silver halide grains to be sensitized therewith and the condition for chemically ripening the grains, but may fall generally between 10⁻⁸ and 10⁻² mols, preferably between 10⁻⁷ and 10⁻³ mols or so, per mol of the silver halide.

The amount of the gold sensitizer to be added to the silver halide grains also varies depending on various conditions. In general, it may fall between 10⁻⁷ and 10⁻³ mols, preferably between 10⁻⁶ and 5 × 10⁻⁴ mols, per mol of the silver halide.

Though not specifically defined, the condition for chemical sensitization in the first embodiment of the invention may be such that the pH falls between 5 and 8, the pAg falls between 6 and 11, and the temperature falls between 40 and 95°C or so.

If desired, a thiosulfonic acid compound may be added to the silver halide emulsions for use in the first embodiment of the invention, according to the method described in EP Laid-Open 293,917.

Preferably, the photosensitive silver halide grains in the first embodiment of the invention are processed with a reducing agent. Concretely, preferred examples of compounds for such reduction sensitization are ascorbic acid, thiourea dioxide, as well as stannous chloride, aminoimimomethanesulfinic acid, hydrazine derivatives, borane compounds, silane compounds and polyamine compounds. The reduction sensitizer may be added to the grains in any stage of preparing the photosensitive emulsions including the stage of grain growth to just before coating the emulsions. Preferably, the emulsions are subjected to such reduction sensitization while they are kept ripened at a pH of 7 or more and at a pAg of 8.3 or less. Also preferably, they may be subjected to reduction sensitization while the grains are formed with a single addition part of silver ions being introduced thereinto.

The photothermographic material of the first embodiment of the invention may contain only one type or two or more different types of photosensitive silver halide grains (these will differ in their mean grain size, halogen composition or crystal habit, or in the condition for their chemical sensitization), either singly or as combined. Combining two or more types of photosensitive silver halide grains differing in their sensitivity will enable to control the gradation of the images to be formed in the photothermographic material.

For the technique relating to it, referred to are JP-A 57-119341, 53-106125, 47-3929, 48-55730, 46-5187, 50-73627, 57-150841. The sensitivity difference between the combined silver halide grains is preferably such that the respective emulsions differ from each other at least by 0.2 logE.

### <<Amount of Silver Halide in Photothermographic Material>>

The amount of the photosensitive silver halide to be in the photothermographic material of this embodiment is, in terms of the amount of silver per m² of the material, preferably from 0.03 to 0.6 g/m², more preferably from 0.07 to 0.4 g/m², most preferably from 0.05 to 0.3 g/m². Relative to one mol of the organic silver salt therein, the amount of the photosensitive silver halide grains to be in the material preferably falls between 0.01 mols and 0.3 mols, more preferably between 0.02 mols and 0.2 mols, even more preferably between 0.03 mols and 0.15 mols.

### <<Mode of Mixing Photosensitive Silver Halide and Organic Silver Salt>>

Regarding the method and the condition for mixing the photosensitive silver halide grains and an organic silver salt having been prepared separately, for example, employable is a method of mixing them in a high-performance stirrer, a ball mill, a sand mill, a colloid mill, a shaking mill, a homogenizer or the like; or a method of adding the photosensitive silver halide grains having been prepared to the organic silver salt being prepared, in any desired timing to produce the organic silver salt mixed with the silver halide grains.

Preferably, the silver halide for use in the first embodiment of the invention is formed in the absence of the organic silver salt as in the manner as above. Mixing two or more different types of aqueous, organic silver salt dispersions with two or more different types of aqueous, photosensitive silver salt dispersions is also preferred for suitably controlling the photographic properties of the photothermographic material of this embodiment.

### <<Mode of Mixing Photosensitive Silver Halide in Coating Liquid>>

The preferred time at which the silver halide grains are added to the coating liquid which is to form the image-forming layer on the support of the photothermographic material of the first embodiment of the invention may fall between 180 minutes before coating the liquid and a time just before the coating, more preferably between 60 minutes before the coating and 10 seconds before it. However, there is no specific limitation thereon, so far as the method and the condition employed for adding the grains to the coating liquid ensure the advantages of the first embodiment of the invention.

Concretely for mixing them, employable is a method of adding the grains to the coating liquid in a tank in such a controlled manner that the mean residence time for the grains in the tank, as calculated from the amount of the grains added and the flow rate of the coating liquid to a coater, could be a predetermined period of time; or a method of mixing them with a static mixer, for example, as in N. Harunby, M. F. Edwards & A. W. Nienow's Liquid Mixing Technology, Chap. 8 (translated by Koji Takahasi, published by Nikkan Kogyo Shinbun, 1989).

### <<Gradation and Mean Contrast>>

The image gradation of the photothermographic material is not specifically defined, but is preferably such that the mean contrast of the images formed on the material to have a density of from 1.5 to 3.0 falls between 1.5 and 10, in order that the material produces better results of this embodiment.

The mean image contrast referred to herein is represented by the degree of inclination of the line drawn to connect the optical density 1.5 and the optical density 3.0 on the characteristic curve in a graph that indicates the image characteristic of the processed photothermographic material. In the graph, the horizontal axis indicates the logarithmic number of the amount of laser to which the material is exposed for image formation, and the vertical axis indicates the optical density of the image formed on the laser-exposed and thermally-developed material.

Preferably, the mean image contrast falls between 1.5 and 10 for sharp letters and images, more preferably between 2.0 and 7, even more preferably between 2.5 and 6.

### <Non-photosensitive Organic Silver Salt>

The organic silver salt for use in the first embodiment of the invention is relatively stable to light, but, when heated at 80°C or higher in the presence of an exposed photocatalyst (e.g., latent image of photosensitive silver halide) and a reducing agent, it forms a silver image. The organic silver salt may be any and every organic substance that contains a source having the ability to reduce silver ions.

Some non-photosensitive organic silver salts of that type are described, for example, in JP-A 10-62899, paragraphs [0048] to [0049]; EP Laid-Open 0803764A1, from page 18, line 24 to page 19, line 37; EP Laid-Open 0962812A1; JP-A 11-349591, 2000-7683, 2000-72711. Preferred for use herein are silver salts of organic acids, especially silver salts of long-chain (C10 to C30, preferably C 15 to C28) aliphatic carboxylic acids. Preferred examples of silver salts of such fatty acids are silver behenate, silver arachidate, silver stearate, silver oleate, silver laurate, silver caproate, silver myristate, silver palmitate, and their mixtures.

Of those, especially preferred for use in the first embodiment of the invention are silver salts of fatty acids having a silver behenate content of at least 50 mol%, more preferably at least 80 mol%, even more preferably at least 90 mol%.

The organic silver salt for use in the first embodiment of the invention is not specifically defined for its morphology, and may be in any form of acicular, rod-like, tabular or scaly solids.

Scaly organic silver salts are preferred in the first embodiment of the invention. Also preferred are short acicular grains having a ratio of major axis to minor axis of at most 5, or rectangular-parallelepiped or cubic grains, or amorphous grains such as potato-like grains. These organic silver grains are characterized in that they are fogged little through thermal development as compared with long acicular grains having a ratio of major axis to minor axis of more than 5.

In this description, the scaly organic silver salts are defined as follows: A sample of an organic silver salt to be analyzed is observed with an electronic microscope, and the grains of the salt seen in the field are approximated to rectangular parallelopipedons. The three different edges of the thus-approximated, one rectangular parallelopipedone are represented by a, b and c. a is the shortest, c is the longest, and c and b may be the same. From the shorter edges a and b, x is obtained according to the following equation: $x = b / a .$

About 200 grains seen in the field are analyzed to obtain the value x, and the data of x are averaged. Samples that satisfy the requirement of x (average) ≥ 1.5 are scaly. For scaly grains, preferably, 30 ≥ x (average) ≥ 1.5, more preferably 20 ≥ x (average) ≥ 2.0. In this connection, the value x of acicular (needle-like) grains falls within a range of 1 ≤ x (average) < 1.5.

In the scaly grains, it is understood that a corresponds to the thickness of tabular grains of which the main plane is represented by b × c. In the scaly organic silver salt grains for use herein, a (average) preferably falls between 0.01 µm and 0.23 µm, more preferably between 0.1 µm and 0.20 µm; and c/b (average) preferably falls between 1 and 6, more preferably between 1.05 and 4, even more preferably between 1.1 and 3, still more preferably between 1.1 and 2.

Regarding its grain size distribution, the organic silver salt is preferably a mono-dispersed one. Mono-dispersion of grains referred to herein is such that the value (in terms of percentage) obtained by dividing the standard deviation of the minor axis and the major axis of each grain by the minor axis and the major axis thereof, respectively, is preferably at most 100 %, more preferably at most 80 %, even more preferably at most 50 %. To determine its morphology, a dispersion of the organic silver salt may be analyzed on its image taken by the use of a transmission electronic microscope.

Another method for analyzing the organic silver salt for mono-dispersion morphology comprises determining the standard deviation of the volume weighted mean diameter of the salt grains. In the method, the value in terms of percentage (coefficient of variation) obtained by dividing the standard deviation by the volume weighted mean diameter of the salt grains is preferably at most 100 %, more preferably at most 80 %, even more preferably at most 50 %.

Concretely, for example, a sample of the organic silver salt is dispersed in a liquid, the resulting dispersion is exposed to a laser ray, and the self-correlation coefficient of the salt grains relative to the time-dependent change of the degree of fluctuation of the scattered ray is obtained. Based on this, the grain size (volume weighted mean diameter) of the salt grains is obtained.

For preparing and dispersing the organic silver salts for use in the first embodiment of the invention, employable is any known method. For it, for example, referred to are JP-A 10-62899; EP Laid-Open 0803763A1 and 962812A1; JP-A 11-349591, 2000-7683, 2000-72711; and Japanese Patent Application Nos. 11-348228, 11-348229, 11-348230, 11-203413, 2000-90093, 2000-195621, 2000-191226, 2000-213813, 2000-214155, 2000-191226.

It is desirable that the organic silver salt is dispersed substantially in the absence of a photosensitive silver salt, since the photosensitive silver salt, if any in the dispersing system, will be fogged and its sensitivity will be significantly lowered.

For the photothermographic material of the first embodiment of the invention, it is desirable that the amount of the photosensitive silver salt that may be in the aqueous dispersion of the organic silver salt is at most 0.1 mol% relative to one mol of the organic silver salt therein, and it is more desirable that any photosensitive silver salt is not forcedly added to the aqueous dispersion.

In the first embodiment of the invention, an aqueous dispersion of the organic silver salt may be mixed with an aqueous dispersion of the photosensitive silver salt to prepare the photothermographic material. The blend ratio of the organic silver salt to the photosensitive silver salt in the mixture may be suitably determined depending on the object of the invention. Preferably, the blend ratio of the photosensitive silver salt to the organic silver salt in the mixture falls between 1 and 30 mol%, more preferably between 2 and 20 mol%, even more preferably between 3 and 15 mol%.

Mixing two or more different types of aqueous, organic silver salt dispersions with two or more different types of aqueous, photosensitive silver salt dispersions is preferred for controlling the photographic properties of the resulting mixture.

The amount of the organic silver salt to be in the photothermographic material of the first embodiment of the invention is not specifically defined, and may be any desired one. Preferably, the amount of the salt falls between 0.1 and 5 g/m², more preferably between 0.3 and 3 g/m², even more preferably between 0.5 and 2 g/m² in terms of the amount of silver in the salt.

### <Reducing Agent>

The photothermographic material of the first embodiment of the invention preferably contains a thermal developing agent that serves as a reducing agent for the organic silver salt therein. The reducing agent for the organic silver salt may be any and every substance capable of reducing silver ions into metal silver, but is preferably an organic substance.

Some examples of the reducing agent are described in JP-A 11-65021, paragraphs [0043] to [0045], and in EP Laid-Open 0803764A1, from page 7, line 34 to page 18, line 12.

Especially preferred for the reducing agent in the first embodiment of the invention are hindered phenol-type reducing agents and bisphenol-type reducing agents that have an ortho-positioned substituent relative to the phenolic hydroxyl group therein, and more preferred are compounds of the following general formula (R):

In formula (R), R¹¹ and R^{11'} each independently represent an alkyl group having from 1 to 20 carbon atoms; R¹² and R^{12'} each independently represent a hydrogen atom, or a substituent substitutable to the benzene ring; L represents -S- or -CHR¹³-; R¹³ represents a hydrogen atom, or an alkyl group having from 1 to 20 carbon atoms; X¹ and X^{1'} each independently represent a hydrogen atom, or a substituent substitutable to the benzene ring.

Formula (R) is described in detail.

R¹¹ and R^{11'} each independently represent a substituted or unsubstituted alkyl group having from 1 to 20 carbon atoms. The substituent for the alkyl group is not specifically defined, but preferably includes, for example, an aryl group, a hydroxyl group, an alkoxy group, an aryloxy group, an alkylthio group, an arylthio group, an acylamino group, a sulfonamido group, a sulfonyl group, a phosphoryl group, an acyl group, a carbamoyl group, an ester group, an ureido group, an urethane group, and a halogen atom.

R¹² and R^{12'} each independently represent a hydrogen atom, or a substituent substitutable to the benzene ring; X¹ and X^{1'} each independently represent a hydrogen atom, or a substituent substitutable to the benzene ring. Preferred examples of the substituent substitutable to the benzene ring are an alkyl group, an aryl group, a halogen atom, an alkoxy group, and an acylamino group.

L represents a group of -S- or -CHR¹³-. R¹³ represents a hydrogen atom or an alkyl group having from 1 to 20 carbon atoms. The alkyl group may be substituted.

Specific examples of the unsubstituted alkyl group for R¹³ are methyl, ethyl, propyl, butyl, heptyl, undecyl, isopropyl, 1-ethylpentyl and 2,4,4-trimethylpentyl groups. For the substituent for the substituted alkyl group for it, referred to are those mentioned hereinabove for the substituted alkyl group for R¹¹.

For R¹¹ and R^{11'}, preferred is a secondary or tertiary alkyl group having from 3 to 15 carbon atoms. Concretely, preferred examples of the alkyl group are isopropyl, isobutyl, t-butyl, t-amyl, t-octyl, cyclohexyl, cyclopentyl, 1-methylcyclohexyl and 1-methylcyclopropyl groups.

For R¹¹ and R^{11'}, more preferred is a tertiary alkyl group having from 4 to 12 carbon atoms; even more preferred is any of t-butyl, t-amyl and 1-methylcycohexyl groups; and most preferred is a t-butyl group.

Preferably, R¹² and R^{12'} each are an alkyl group having from 1 to 20 carbon atoms, concretely including, for example, methyl, ethyl, propyl, butyl, isopropyl, tert-butyl, tert-amyl, cyclohexyl, 1-methylcyclohexyl, benzyl, methoxymethyl and methoxyethyl groups. For these, more preferred are methyl, ethyl, propyl, isopropyl and tert-butyl groups.

Also preferably, X¹ and X^{1'} each are a hydrogen atom, a halogen atom or an alkyl group; and more preferably, they are both hydrogen atoms.

L is preferably -CHR¹³-.

Also preferably, R¹³ is a hydrogen atom, or an alkyl group having from 1 to 15 carbon atoms. Preferred examples of the alkyl group are methyl, ethyl, propyl, isopropyl and 2,4,4-trimethylpentyl groups. More preferably, R¹³ is a hydrogen atom, a methyl group, an ethyl group, a propyl group or an isopropyl group.

In case where R¹³ is a hydrogen atom, R¹² and R^{12'} each are preferably an alkyl group having from 2 to 5 carbon atoms, more preferably an ethyl or propyl group, most preferably, they are both ethyl groups.

In case where R¹³ is a primary or secondary alkyl group having from 1 to 8 carbon atoms, R¹² and R^{12'} are preferably both methyl groups. The primary or secondary alkyl group having from 1 to 8 carbon atoms for R¹³ is preferably a methyl, ethyl, propyl or isopropyl group, more preferably a methyl, ethyl or propyl group.

In case where R¹¹, R^{11'}, R¹² and R^{12'} are all methyl groups, R¹³ is preferably a secondary alkyl group. The secondary alkyl group for R¹³ is preferably an isopropyl, isobutyl or 1-ethylpentyl group, more preferably an isopropyl group.

Depending on the combination of R¹¹, R^{11'}, R¹², R^{12'} and R¹³ therein, the reducing agents differ in their thermal developability and in the tone of developed silver. Combining two or more different types of reducing agents enables to control the developability and the developed silver tone. Depending on their object, therefore, combining them will be preferred in the invention.

Examples of the compounds of formula (R) and other reducing agents for use in the first embodiment of the invention are mentioned below, to which, however, the invention of this embodiment is not limited.

Preferably, the amount of the reducing agent to be in the photothermographic material of the first embodiment of the invention falls between 0.1 and 3.0 g/m², more preferably between 0.2 and 1.5 g/m², even more preferably between 0.3 and 1.0 g/m².

Also preferably, the amount of the reducing agent to be in the material falls between 5 and 50 mol%, more preferably between 8 and 30 mol%, even more preferably between 10 and 20 mol% per mol of silver existing in the face of the image-forming layer of the material.

The reducing agent may be in any form of solution, emulsified dispersion or fine solid particle dispersion, and may be added to the coating liquid in any known method so as to be incorporated into the photothermographic material of the invention.

One well known method of emulsifying the reducing agent to prepare its dispersion comprises dissolving the reducing agent in an auxiliary solvent such dibutyl phthalate, tricresyl phosphate, glyceryl triacetate, diethyl phthalate or the like oily solvent, or in ethyl acetate or cyclohexanone, followed by mechanically emulsifying it into a dispersion.

For preparing a fine solid particle dispersion of the reducing agent, for example, employable is a method that comprises dispersing a powder of the reducing agent in water or in any other suitable solvent by the use of a ball mill, a colloid mill, a shaking ball mill, a sand mill, a jet mill or a roller mill, or ultrasonically dispersing it therein to thereby prepare the intended solid dispersion of the reducing agent. In this method, optionally used is a protective colloid (e.g., polyvinyl alcohol), and a surfactant (e.g., anionic surfactant such as sodium triisopropylnaphthalenesulfonate - this is a mixture of the salts in which the three isopropyl groups are all in different positions). In these mills, generally used are beads of zirconia or the like that serve as a dispersion medium. Zr or the like may dissolve out of the beads and will often contaminate the dispersion formed. Though varying depending on the dispersion condition, the contaminant content of the dispersion formed may generally fall between 1 ppm and 1000 ppm. So far as the Zr content of the photothermographic material finally fabricated herein is not larger than 0.5 mg per gram of silver in the material, the contaminant will cause no practical problem.

Preferably, the aqueous dispersion contains a preservative (e.g., sodium benzoisothiazolinone).

### <Development Accelerator>

Preferably, the photothermographic material of the first embodiment of the invention contains a development accelerator. Preferred examples of the development accelerator are sulfonamidophenol compounds of formula (A) in JP-A 2000-267222 and 2000-330234; hindered phenol compounds of formula (II) in JP-A 2001-92075; compounds of formula (I) in JP-A 10-62895 and 11-15116; hydrazine compounds of formula (I) in Japanese Patent Application No. 2001-074278; and phenol or naphthol compounds of formula (2) in Japanese Patent Application No. 2000-76240. The amount of the development accelerator to be in the material may fall between 0.1 and 20 mol%, but preferably between 0.5 and 10 mol%, more preferably between 1 and 5 mol% relative to the reducing agent therein. The development accelerator may be introduced into the material like the reducing agent thereinto. Preferably, however, it is added to the material in the form of its solid dispersion or emulsified dispersion. In case where it is added to the material in the form of its emulsified dispersion, the emulsified dispersion thereof is preferably prepared by emulsifying and dispersing the development accelerator in a mixed solvent of a high-boiling point solvent that is solid at room temperature and an auxiliary solvent having a low boiling point; or the emulsified dispersion is preferably an oilless dispersion with no high-boiling-point solvent therein.

Of the development accelerators mentioned above, especially preferred for use in the first embodiment of the invention are hydrazine compounds of formula (I) described in Japanese Patent Application No. 2001-074278, and phenol or naphthol compounds of formula (2) described in Japanese Patent Application No. 2000-76240.

Preferred examples of the development accelerators for use in the first embodiment of the invention are mentioned below, to which, however, this embodiment is not limited.

### <Hydrogen Bonding Type Compound>

A Hydrogen bonding type compound may be in the photothermographic material of the first embodiment of the invention, and the compound is described.

In case where the reducing agent in the first embodiment of the invention has an aromatic hydroxyl group (-OH), especially when it is any of the above-mentioned bisphenols, the reducing agent is preferably combined with a non-reducing compound that has a group capable of forming a hydrogen bond with the group in the reducing agent.

The group capable of forming a hydrogen bond with the hydroxyl group or the amino group in the reducing agent includes, for example, a phosphoryl group, a sulfoxide group, a sulfonyl group, a carbonyl group, an amido group, an ester group, an urethane group, an ureido group, a tertiary amino group, and a nitrogen-containing aromatic group.

Of those, preferred are a phosphoryl group, a sulfoxide group, an amido group (not having a group of >N-H but is blocked to form >N-Ra, in which Ra is a substituent except H), an urethane group (not having a group of >N-H but is blocked to form >N-Ra, in which Ra is a substituent except H), an ureido group (not having a group of >N-H but is blocked to form >N-Ra, in which Ra is a substituent except H).

Especially preferred examples of the Hydrogen bonding type compound for use in the first embodiment of the invention are those of the following general formula (D):

In formula (D), R²¹ to R²³ each independently represent an alkyl group, an aryl group, an alkoxy group, an aryloxy group, an amino group or a heterocyclic group. These may be unsubstituted or substituted.

The substituents for the substituted groups for R²¹ to R²³ are, for example, a halogen atom, an alkyl group, an aryl group, an alkoxy group, an amino group, an acyl group, an acylamino group, an alkylthio group, an arylthio group, a sulfonamido group, an acyloxy group, an oxycarbonyl group, a carbamoyl group, a sulfamoyl group, a sulfonyl group and a phosphoryl group. Of the substituents, preferred are an alkyl group and an aryl group; and more preferred are methyl, ethyl, isopropyl, t-butyl, t-octyl, phenyl, 4-alkoxyphenyl and 4-acyloxyphenyl groups.

The alkyl group for R²¹ to R²³ includes, for example, methyl, ethyl, butyl, octyl, dodecyl, isopropyl, t-butyl, t-amyl, t-octyl, cyclohexyl, 1-methylcyclohexyl, benzyl, phenethyl and 2-phenoxypropyl groups.

The aryl group for these includes, for example, phenyl, cresyl, xylyl, naphthyl, 4-t-butylphenyl, 4-t-octylphenyl, 4-anisidyl and 3,5-dichlorophenyl groups.

The alkoxy group for these includes, for example, methoxy, ethoxy, butoxy, octyloxy, 2-ethylhexyloxy, 3,5,5-trimethylhexyloxy, dodecyloxy, cyclohexyloxy, 4-methylcyclohexyloxy and benzyloxy groups.

The aryloxy group for these includes, for example, phenoxy, cresyloxy, isopropylphenoxy, 4-t-butylphenoxy, naphthoxy and biphenyloxy groups. The amino group for these includes, for example, dimethylamino, diethylamino, dibutylamino, dioctylamino, N-methyl-N-hexylamino, dicyclohexylamino, diphenylamino and N-methyl-N-phenylamino groups.

For R²¹ to R²³, preferred are an alkyl group, an aryl group, an alkoxy group and an aryloxy group. From the viewpoint of the advantages of the first embodiment of the invention, it is preferable that at least one of R²¹ to R²³ is an alkyl group or an aryl group, and it is more desirable that at least two of them are any of an alkyl group and an aryl group. Even more preferably, R²¹ to R²³ are the same as the compounds of the type are inexpensive.

Specific examples of the compounds of formula (D) and other Hydrogen bonding type compounds usable in the first embodiment of the invention are mentioned below, to which, however, this embodiment is not limited.

Apart from the above, other Hydrogen bonding type compounds such as those described in EP 1096310 and in Japanese Patent Application Nos. 2000-270498 and 2001-124796 are also usable herein.

Like the reducing agent mentioned above, the compound of formula (D) may be added to the coating liquid for the photothermographic material of the first embodiment of the invention, for example, in the form of its solution, emulsified dispersion or solid particle dispersion. In its solution, the compound of formula (D) may form a hydrogen-bonding complex with a compound having a phenolic hydroxyl group or an amino group. Depending on the combination of the reducing agent and the compound of formula (D) for use herein, the complex may be isolated as its crystal. Thus isolated, the crystal powder may be formed into its solid particle dispersion, and the dispersion is especially preferred for use herein for stabilizing the photothermographic material of the first embodiment of the invention. As the case may be, the reducing agent and the compound of formula (D) may be mixed both in powder optionally along with a suitable dispersant added thereto in a sand grinder mill or the like to thereby form the intended complex in the resulting dispersion. The method is also preferred in this embodiment.

Preferably, the amount of the compound of formula (D) to be added to the reducing agent in this embodiment falls between 1 and 200 mol%, more preferably between 10 and 150 mol%, even more preferably between 30 and 100 mol% relative to the reducing agent.

### <Binder>

The photothermographic material of first embodiment of the invention contains a binder, and the binder is described below.

The binder to be in the organic silver salt-containing layer in the first embodiment of the invention may be polymer of any type, but is preferably transparent or semitransparent and is generally colorless. For it, for example, preferred are natural resins, polymers and copolymers; synthetic resins, polymers and copolymers; and other film-forming media. More concretely, they include, for example, gelatins, rubbers, poly(vinyl alcohols), hydroxyethyl celluloses, cellulose acetates, cellulose acetate butyrates, poly(vinylpyrrolidones), casein, starch, poly(acrylic acids), poly(methyl methacrylates), poly(vinyl chlorides), poly(methacrylic acids), styrene-maleic anhydride copolymers, styrene-acrylonitrile copolymers, styrene-butadiene copolymers, poly(vinylacetals) (e.g., poly(vinylformal), poly(vinylbutyral)), poly(esters), poly(urethanes), phenoxy resins, poly(vinylidene chlorides), poly(epoxides), poly(carbonates), poly(vinyl acetates), poly(olefins), cellulose esters, and poly(amides). The binder may be prepared from water or an organic solvent or an emulsion through microencapsulation.

The glass transition point of the binder to be in the organic silver salt-containing layer in the first embodiment of the invention preferably falls between 10°C and 80°C (the binder of the type will be hereinafter referred to as a high-Tg binder), more preferably between 15°C and 70°C, even more preferably between 25°C and 65°C.

In this description, Tg is calculated according to the following equation: $1 / Tg = Σ \left(Xi/Tgi\right)$

The polymer of which the glass transition point Tg is calculated as in the above comprises n's monomers copolymerized (i indicates the number of the monomers copolymerized, falling between 1 and n); Xi indicates the mass fraction of i'th monomer (ΣXi = 1); Tgi indicates the glass transition point (in terms of the absolute temperature) of the homopolymer of i'th monomer alone; and E indicates the sum total of i falling between 1 and n. For the glass transition point (Tgi) of the homopolymer of each monomer alone, referred to is the description in Polymer Handbook (3rd edition) (written by J. Brandrup, E. H. Immergut (Wiley-Interscience, 1989)).

One and the same polymer may be used for the binder, but, if desired, two or more different types of polymers may be combined for it. For example, a polymer having a glass transition point of 20°C or higher and a polymer having a glass transition point of lower than 20°C may be combined. In case where at least two polymers that differ in Tg are blended for use herein, it is desirable that the weight-average Tg of the resulting blend falls within the range defined as above.

In the first embodiment of the invention, it is desirable that the organic silver salt-containing layer is formed by applying a coating liquid, in which at least 30 % by weight of the solvent is water, onto the support followed by drying it.

In case where the organic silver salt-containing layer in the first embodiment of the invention is formed by using such a coating liquid in which at least 30 % by weight of the solvent is water, followed by drying it, and in case where the binder in the organic silver salt-containing layer is soluble or dispersible in an aqueous solvent (watery solvent), especially when the binder in the organic silver salt-containing layer is a polymer latex that has an equilibrium water content at 25°C and 60 % RH of at most 2 % by weight, the photothermographic material having the layer of the type enjoys better properties. Most preferably, the binder for use in this embodiment is so designed that its ionic conductivity is at most 2.5 mS/cm. For preparing the binder of the type, for example, employable is a method of preparing a polymer for the binder followed by purifying it through a functional membrane for fractionation.

The aqueous solvent in which the polymer binder is soluble or dispersible is water or a mixed solvent of water and at most 70 % by weight of a water-miscible organic solvent.

The water-miscible organic solvent includes, for example, alcohols such as methyl alcohol, ethyl alcohol, propyl alcohol; cellosolves such as methyl cellosolve, ethyl cellosolve, butyl cellosolve; ethyl acetate, and dimethylformamide.

The terminology "aqueous solvent" referred to herein can apply also to polymer systems in which the polymer is not thermodynamically dissolved but is seemingly dispersed.

The "equilibrium water content at 25°C and 60 % RH" referred to herein for polymer latex is represented by the following equation, in which W₁ indicates the weight of a polymer in humidity-conditioned equilibrium at 25°C and 60 % RH, and W₀ indicates the absolute dry weight of the polymer at 25°C. $\begin{matrix}Equilibrium water content at 25 ⁢ °C and 60 % RH = \left\{\left({W}_{1}-{W}_{0}\right)/{W}_{0}\right\} \times 100 \left(wt.%\right)\end{matrix}$

For the details of the definition of water content and the method for measuring it, for example, referred to is Polymer Engineering, Lecture 14, Test Methods for Polymer Materials (by the Polymer Society of Japan, Chijin Shokan Publishing).

Preferably, the equilibrium water content at 25°C and 60 % RH of the binder polymer for use in the first embodiment of the invention is at most 2 % by weight, more preferably from 0.01 to 1.5 % by weight, even more preferably from 0.02 to 1 % by weight.

Polymers that serve as the binder in the first embodiment of the invention are preferably dispersible in aqueous solvents. Polymer dispersions include, for example, a type of hydrophobic polymer latex with water-insoluble fine polymer particles being dispersed, and a type of molecular or micellar polymer dispersion with polymer molecules or micelles being dispersed. Any of these may be employed herein, but preferred is polymer latex dispersion.

The particles in the polymer dispersions may have a mean particle size falling between 1 and 50000 nm, but preferably between 5 and 1000 nm, more preferably between 10 and 500 nm, even more preferably between 50 and 200 nm. The particle size distribution of the dispersed polymer particles is not specifically defined. For example, the dispersed polymer particles may have a broad particle size distribution, or may have a narrow particle size distribution of monodispersion. Combining two or more different types of mono-dispersed polymer particles both having a narrow particle size distribution is preferred for suitably controlling the physical properties of the coating liquids for use herein.

For the photothermographic material of the first embodiment of the invention, favorably used are hydrophobic polymers that are dispersible in aqueous media. The hydrophobic polymers of the type include, for example, acrylic polymers, poly(esters), rubbers (e.g., SBR resins), poly(urethanes), poly(vinyl chlorides), poly(vinyl acetates), poly(vinylidene chlorides), and poly(olefins). These polymers may be linear, branched or crosslinked ones. They may be homopolymers from one type of monomer, or copolymers from two or more different types of monomers. The copolymers may be random copolymers or block copolymers.

The polymers for use herein preferably have a number-average molecular weight falling between 5000 and 1000000, more preferably between 10000 and 200000. Polymers having a too small molecular weight are unfavorable to the invention, since the mechanical strength of the emulsion layer comprising such a polymer is low; but others having a too large molecular weight are also unfavorable since their workability into films is not good. Especially preferred for use herein is crosslinked polymer latex.

Preferred examples of polymer latex for use herein are mentioned below, to which, however, the first embodiment of the invention is not limited.

The following examples are expressed by the constituent monomers, in which each numeral parenthesized indicates the proportion, in terms of % by weight, of the monomer unit, and the molecular weight of each constituent monomer is in terms of the number-average molecular weight thereof. Polyfunctional monomers form a crosslinked structure in polymer latex comprising them, to which, therefore, the concept of molecular weight does not apply. The polymer latex of the type is referred to as "crosslinked", and the molecular weight of the constituent monomers is omitted. Tg indicates the glass transition point of the polymer latex.
P-1: Latex of -MMA(70)-EA(27)-MAA(3)- (molecular weight 37000, Tg 61°C)
P-2: Latex of -MMA(70)-2EHA(20)-St(5)-AA(5)- (molecular weight 40000, Tg 59°C)
P-3: Latex of -St(50)-Bu(47)-MMA(3)- (crosslinked, Tg -17°C)
P-4: Latex of -St(68)-Bu(29)-AA(3)- (crosslinked, Tg 17°C)
P-5: Latex of -St(71)-Bu(26)-AA(3)- (crosslinked, Tg 24°C)
P-6: Latex of -St(70)-Bu(27)-IA(3)- (crosslinked)
P-7: Latex of -St(75)-Bu(24)-AA(1)- (crosslinked, Tg 29°C)
P-8: Latex of -St(60)-Bu(35)-DVB(3)-MAA(2)- (crosslinked)
P-9: Latex of -St(70)-Bu(25)-DVB(2)-AA(3)- (crosslinked)
P-10: Latex of -VC(50)-MMA(20)-EA(20)-AN-(5)-AA(5)- (molecular weight 80000)
P-11: Latex of -VDC(85)-MMA(5)-EA(5)-MAA(5)- (molecular weight 67000)
P-12: Latex of -Et(90)-MAA(10)- (molecular weight 12000)
P-13: Latex of -St(70)-2EHA(27)-AA(3)- (molecular weigh: 130000, Tg 43°C)
P-14: Latex of -MMA(63)-EA(35)-AA(2)- (molecular weight 33000, Tg 47°C)
P-15: Latex of -St(70.5)-Bu(26.5)-AA(3)- (crosslinked, Tg 23°C)
P-16: Latex of -St(69.5)-Bu(27.5)-AA(3)- (crosslinked, Tg 20.5°C)

Abbreviations of the constituent monomers are as follows:
- MMA:: methyl methacrylate
- EA:: ethyl acrylate
- MAA:: methacrylic acid
- 2EHA:: 2-ethylhexyl acrylate
- St:: styrene
- Bu:: butadiene
- AA:: acrylic acid
- DVB:: divinylbenzene
- VC:: vinyl chloride
- AN:: acrylonitrile
- VDC:: vinylidene chloride
- Et:: ethylene
- IA:: itaconic acid

The polymer latexes mentioned above are available on the market. Some commercial products employable herein are mentioned below. Examples of acrylic polymers are CEBIAN A-4635, 4718, 4601 (all from Daicel Chemical Industries), and Nipol Lx811, 814, 821, 820, 857 (all from Nippon Zeon); examples of poly(esters) are FINETEX ES650, 611, 675, 850 (all from Dai-Nippon Ink & Chemicals), and WD-size, WMS (both from Eastman Chemical); examples of poly(urethanes) are HYDRAN AP10, 20, 30, 40 (all from Dai-Nippon Ink & Chemicals); examples of rubbers are LACSTAR 7310K, 3307B, 4700H, 7132C (all from Dai-Nippon Ink & Chemicals), and Nipol Lx416, 410, 438C, 2507 (all from Nippon Zeon); examples of poly(vinyl chlorides) are G351, G576 (both from Nippon Zeon); examples of poly(vinylidene chlorides) are L502, L513 (both from Asahi Kasei); and examples of poly(olefins) are CHEMIPEARL S120, SA100 (both from Mitsui Petrochemical).

These polymer latexes may be used either singly or as combined in any desired manner.

For the polymer latex for use in the first embodiment of the invention, especially preferred is styrene-butadiene copolymer latex. In the styrene-butadiene copolymer, the ratio of styrene monomer units to butadiene monomer units preferably falls between 40/60 and 95/5 by weight. Also preferably, the styrene monomer units and the butadiene monomer units account for from 60 to 99 % by weight of the copolymer. Still preferably, the polymer latex for use in the first embodiment of the invention contains from 1 to 6 % by weight, more preferably from 2 to 5 % by weight of acrylic acid or methacrylic acid relative to the sum of styrene and butadiene therein. Even more preferably, the polymer latex for use in the first embodiment of the invention contains acrylic acid.

Preferred examples of the styrene-butadiene-acid copolymer latex for use in the first embodiment of the invention are the above-mentioned P-3 to P-8, and commercial products, LACSTAR-3307B, 7132C, and Nipol Lx416.

The styrene-butadiene-acid copolymer latex of the type preferably has Tg falling between 10°C and 30°C, more preferably between 17°C and 25°C.

The organic silver salt-containing layer of the photothermographic material of the first embodiment of the invention may optionally contain a hydrophilic polymer such as gelatin, polyvinyl alcohol, methyl cellulose, hydroxypropyl cellulose or carboxymethyl cellulose. The amount of the hydrophilic polymer that may be in the layer is preferably at most 30 % by weight, more preferably at most 20 % by weight of all the binder in the organic silver salt-containing layer.

Preferably, the polymer latex as above is used in forming the organic silver salt-containing layer (that is, the image-forming layer) of the photothermographic material of the first embodiment of the invention. Concretely, the amount of the binder in the organic silver salt-containing layer is such that the ratio by weight of total binder/organic silver salt falls between 1/10 and 10/1, more preferably between 1/3 and 5/1, even more preferably between 1/1 and 3/1.

The organic silver salt-containing layer is a photosensitive layer (emulsion layer) generally containing a photosensitive silver salt, that is, a photosensitive silver halide. In the layer, the ratio by weight of total binder/silver halide preferably falls between 5 and 400, more preferably between 10 and 200.

The overall amount of the binder in the image-forming layer of the photothermographic material of the first embodiment of the invention preferably falls between 0.2 and 30 g/m², more preferably between 1 and 15 g/m², even more preferably between 2 and 10 g/m². The image-forming layer in this embodiment may optionally contain a crosslinking agent, and a surfactant which is for improving the coatability of the coating liquid for the layer.

### <Solvent Preferred for Coating Liquid>

Preferably, the solvent for the coating liquid for the organic silver salt-containing layer of the photothermographic material of the first embodiment of the invention is an aqueous solvent that contains at least 30 % by weight of water. The solvent referred to herein is meant to indicate both solvent and dispersion medium for simple expression.

Except water, the other components of the aqueous solvent may be any organic solvents that are miscible with water, including, for example, methyl alcohol, ethyl alcohol, isopropyl alcohol, methyl cellosolve, ethyl cellosolve, dimethylformamide, ethyl acetate. The water content of the solvent for the coating liquid is preferably at least 50 % by weight, more preferably at least 70 % by weight.

Preferred examples of the solvent composition are water alone, water/methyl alcohol = 90 / 10, water/methyl alcohol = 70/ 30, water/methyl alcohol/dimethylformamide = 80/15/5, water/methyl alcohol/ethyl cellosolve = 85/ 10/5, water/methyl alcohol/isopropyl alcohol = 85/10/5. The ratio is by weight.

### <Antifoggant and Others>

Antifoggants usable in the first embodiment of the invention are described.

For the antifoggants, stabilizers and stabilizer precursors employable in this embodiment, referred to are the compounds in JP-A 10-62899, paragraph [0070]; EP Laid-Open 0803764A1, from page 20, line 57 to page 21, line 7; JP-A 9-281637, 9-329864, and also referred to are the compounds in USP 6,083,681, 6,083,681, and EP 1048975.

Antifoggants preferred for use in the first embodiment of the invention are organic halides. These are described, for example, in JP-A 11-65021, paragraphs [0111] to [0112]. Especially preferred are organic halogen compounds of formula (P) in JP-A 2000-284399; organic polyhalogen compounds of formula (II) in JP-A 10-339934; and organic polyhalogen compounds in JP-A 2001-31644 and 2001-33911.

Organic polyhalogen compounds preferred for use in the first embodiment of the invention are described concretely. Preferably, the polyhalogen compounds for use in the first embodiment of the invention are represented by the following general formula (H):

General Formula (H) Q-(Y)n-C(Z₁)(Z₂)X

wherein Q represents an alkyl, aryl or heterocyclic group; Y represents a divalent linking group; n indicates 0 or 1; Z₁ and Z₂ each represent a halogen atom; and X represents a hydrogen atom or an electron-attracting group.

In formula (H), Q is preferably a phenyl group substituted with an electron-attracting group having a positive Hammett's substituent constant σₚ. For the Hammett's substituent constant, referred to is, for example, Journal of Medicinal Chemistry, 1973, Vol. 16, No. 11, 1207-1216.

Examples of the electron-attracting group of the type are a halogen atom (fluorine atom with σₚ of 0.06, chlorine atom with σₚ of 0.23, bromine atom with σₚ of 0.23, iodine atom with σₚ of 0.18), a trihalomethyl group (tribromomethyl with σₚ of 0.29, trichloromethyl with σₚ of 0.33, trifluoromethyl with σₚ of 0.54), a cyano group (with σₚ of 0.66), a nitro group (with σₚ of 0.78), an aliphatic, aryl or heterocyclic sulfonyl group (e.g., methanesulfonyl with σₚ of 0.72), an aliphatic, aryl or heterocyclic acyl group (e.g., acetyl with σₚ of 0.50, benzoyl with σₚ of 0.43), an alkynyl group (e.g., C≡CH with σₚ of 0.23), an aliphatic, aryl or heterocyclic oxycarbonyl group (e.g., methoxycarbonyl with σₚ of 0.45, phenoxycarbonyl with σₚ of 0.44), a carbamoyl group (with σₚ of 0.36), a sulfamoyl group (with σₚ of 0.57), a sulfoxide group, a heterocyclic group, and a phosphoryl group. The σₚ value of the electron-attracting group preferably falls between 0.2 and 2.0, more preferably between 0.4 and 1.0.

Of the preferred examples of the electron-attracting group mentioned above, more preferred are a carbamoyl group, an alkoxycarbonyl group, an alkylsulfonyl group and an alkylphosphoryl group, and most preferred is a carbamoyl group.

In formula (H), X is preferably an electron-attracting group, more preferably a halogen atom, an aliphatic, aryl or heterocyclic sulfonyl group, an aliphatic, aryl or heterocyclic acyl group, an aliphatic, aryl or heterocyclic oxycarbonyl group, a carbamoyl group, or a sulfamoyl group. Even more preferably, it is a halogen atom. For the halogen atom for X, preferred are chlorine, bromine and iodine atoms, more preferred are chlorine and bromine atoms, and even more preferred is a bromine atom.

In formula (H), Y is preferably -C(=O)-, -SO- or -SO₂-, more preferably -C(=O)- or -SO₂-, even more preferably -SO₂-. n is 0 or 1, but preferably 1.

Specific examples of the compounds of formula (H) for use in the first embodiment of the invention are mentioned below.

Preferably, the amount of the compound of formula (H) to be in the photothermographic material of the first embodiment of the invention falls between 1 × 10⁻⁴ and 0.5 mols, more preferably between 10⁻³ and 0.1 mols, even more preferably between 5 × 10⁻³ and 0.05 mols per mol of the non-photosensitive silver salt in the image-forming layer of the material.

The antifoggant may be incorporated into the photothermographic material of the first embodiment of the invention in the same manner as that mentioned hereinabove for incorporating the reducing agent thereinto. Preferably, the organic polyhalogen compound is in the form of a fine solid particle dispersion when it is incorporated into the material.

### <Other Antifoggants>

Other antifoggants usable herein are mercury(II) salts as in JP-A 11-65021, paragraph [0113]; benzoic acids as in JP-A 11-65021, paragraph [0114]; salicylic acid derivatives as in JP-A 2000-206642; formalin scavenger compounds of formula (S) in JP-A 2000-221634; triazine compounds claimed in claim 9 in JP-A 11-352624; compounds of formula (III) in JP-A 6-11791; and 4-hydroxy-6-methyl-1,3,3a,7-tetrazaindene.

The photothermographic material of the first embodiment of the invention may also contain an azolium salt serving as an antifoggant. The azolium salt includes, for example, compounds of formula (XI) in JP-A 59-193447, compounds as in JP-B 55-12581, and compounds of formula (II) in JP-A 60-153039. The azolium salt may be present in any site of the photothermographic material, but is preferably in a layer adjacent to the photosensitive layer in the material. More preferably, it is added to the organic silver salt-containing layer of the material.

Regarding the time at which the azolium salt is added to the material, it may be added to the coating liquid at any stage of preparing the liquid. In case where it is to be present in the organic silver salt-containing layer, the azolium salt may be added to any of the reaction system to prepare the organic silver salt or the reaction system to prepare the coating liquid at any stage of preparing them. Preferably, however, it is added to the coating liquid after the stage of preparing the organic silver salt and just before the stage of coating the liquid. The azolium salt to be added may be in any form of powder, solution or fine particle dispersion. It may be added along with other additives such as sensitizing dye, reducing agent and toning agent, for example, in the form of their solution.

The amount of the azolium salt to be added to the photothermographic material of the first embodiment of the invention is not specifically defined, but preferably falls between 1 × 10⁻⁶ mols and 2 mols, more preferably between 1 × 10⁻³ mols and 0.5 mols per mol of silver in the material.

### <Other Additives>

### <<Mercapto, Disulfide and Thione Compounds>>

The photothermographic material of the first embodiment of the invention may optionally contain any of mercapto compounds, disulfide compounds and thione compounds which are for retarding, promoting or controlling the developability of the material, or for enhancing the spectral sensitivity thereof, or for improving the storage stability thereof before and after development. For the additive compounds, for example, referred to are JP-A 10-62899, paragraphs [0067] to [0069]; compounds of formula (I) in JP-A 10-186572, and their examples in paragraphs [0033] to [0052]; and EP Laid-Open 0803764A1, page 20, lines 36 to 56. Above all, preferred are mercapto-substituted heteroaromatic compounds such as those in JP-A 9-297367, 9-304875, 2001-100358, and in Japanese Patent Application Nos. 2001-104213 and 2001-104214.

### <<Toning Agent>>

Adding a toning agent to the photothermographic material of the first embodiment of the invention is preferred. Examples of the toning agent usable herein are described in JP-A 10-62899, paragraphs [0054] to [0055], EP Laid-Open 0803764A1, page 21, lines 23 to 48; and JP-A 2000-356317; and Japanese Patent Application No. 2000-187298. Especially preferred for use herein are phthalazinones (phthalazinone, phthalazinone derivatives and their metal salts, e.g., 4-(1-naphthyl)phthalazinone, 6-chlorophthalazinone, 5,7-dimethoxyphthalazinone, 2,3-dihydro-1,4-phthalazinedione); combinations of phthalazinones and phthalic acids (e.g., phthalic acid, 4-methylphthalic acid, 4-nitrophthalic acid, diammonium phthalate, sodium phthalate, potassium phthalate, tetrachlorophthalic anhydride); phthalazines (phthalazine, phthalazine derivatives and their salts, e.g., 4-(1-naphthyl)phthalazine, 6-isopropylphthalazine, 6-tert-butylphthalazine, 6-chlorophthalazine, 5,7-dimethoxyphthalazine, 2,3-dihydrophthalazine); combinations of phthalazines and phthalic acids. More preferred are combinations of phthalazines and phthalic acids. Above all, especially preferred are a combination of 6-isopropylphthalazine and phthalic acid or 4-methylphthalic acid.

### <<Plasticizer, Lubricant>>

Plasticizers and lubricants that may be in the photosensitive layer of the photothermographic material of the first embodiment of the invention are described in, for example, JP-A 11-65021, paragraph [0117]. Lubricants that may be in the layer are also described in JP-A 11-84573, paragraphs [0061] to [0064], and JP-A 11-106881, paragraphs [0049] to [0062].

### <<Dye, pigment>>

The photosensitive layer in the first embodiment of the invention may contain various types of dyes and pigments (e.g., C.I. Pigment Blue 60, C.I. Pigment Blue 64, C.I. Pigment Blue 15:6) for improving the image tone, for preventing interference fringes during laser exposure, and for preventing irradiation. The details of such dyes and pigments are described in, for example, WO98/36322, and JP-A 10-268465 and 11-338098.

### <<Super-hardener>>

For forming super-hard images suitable to printing plates, a super-hardener is preferably added to the image-forming layer of the photothermographic material. For such super-hardeners for forming super-hard images, methods of using them, and their amounts applicable to the invention, for example, referred to are JP-A 11-65021, paragraph [0118]; JP-A 11-223898, paragraphs [0136] to [0193]; compounds of formula (H), those of formulae (1) to (3) and those of formulae (A) and (B) in JP-A 2000-284399; compounds of formulae (III) to (V) in Japanese Patent Application No. 11-91652, especially concrete compounds in [Formula 21] to [Formula 24] therein. For hardening promoters also applicable to the invention, referred to are JP-A 11-65021, paragraph [0102]; and JP-A 11-223898, paragraphs [0194] to [0195].

In case where formic acid or its salt is used for a strong foggant in the invention, it may be added to the photosensitive silver halide-containing, image-forming layer of the material, and its amount is preferably at most 5 mmols, more preferably at most 1 mmol per mol of silver in the layer.

In case where a super-hardener is used in the photothermographic material of the first embodiment of the invention, it is preferably combined with an acid formed through hydration of diphosphorus pentoxide or its salt.

The acid to be formed through hydration of diphosphorus pentoxide and its salts include, for example, metaphosphoric acid (and its salts), pyrophosphoric acid (and its salts), orthophosphoric acid (and its salts), triphosphoric acid (and its salts), tetraphosphoric acid (and its salts), and hexametaphosphoric acid (and its salts).

For the acid to be formed through hydration of diphosphorus pentoxide and its salts, preferred for use herein are orthophosphoric acid (and its salts), and hexametaphosphoric acid (and its salts).

Concretely, their salts are sodium orthophosphate, sodium dihydrogen-orthophosphate, sodium hexametaphosphate, and ammonium hexametaphosphate.

The amount of the acid to be formed through hydration of diphosphorus pentoxide or its salt to be used herein (that is, the amount thereof to be in the unit area, one m², of the photothermographic material) may be any desired one and may be defined in any desired manner depending on the sensitivity, the fogging resistance and other properties of the material. Preferably, however, it falls between 0.1 and 500 mg/m², more preferably between 0.5 and 100 mg/m².

### <<Preparation of Coating Liquid>>

In the first embodiment of the invention, the coating liquid for the image-forming layer is prepared preferably at a temperature falling between 30°C and 65°C, more preferably between 35°C and lower than 60°C, even more preferably between 35°C and 55°C. Also preferably, the coating liquid for the image-forming layer is kept at a temperature falling between 30°C and 65°C just after addition of polymer latex thereto.

### <Layer Constitution>

One or more image-forming layers are formed on one support to produce the photothermographic material of the first embodiment of the invention. In case where the material has one image-forming layer, the layer must contain an organic silver salt, a photosensitive silver halide, a reducing agent and a binder, and may contain optional additives such as a toning agent, a coating aid and other auxiliary agents. In case where the material has two or more image-forming layers, the first image-forming layer (in general, this is directly adjacent to the support) must contain an organic silver salt and a photosensitive silver halide, and the second image-forming layer or the two layers must contain the other ingredients.

The photothermographic material for multi-color expression of the invention may have combinations of these two layers for the respective colors, or may contain all the necessary ingredients in a single layer, for example, as in USP 4,708,928. For the photothermographic material of a type containing multiple dyes for multi-color expression, the individual emulsion layers are differentiated and spaced from the others via a functional or non-functional barrier layer between the adjacent emulsion layers, for example, as in USP 4,460,681.

In general, the photothermographic material has non-photosensitive layers in addition to photosensitive layers. Depending on their positions, the non-photosensitive layers are classified into (1) a protective layer to be disposed on a photosensitive layer (remoter from the support than the photosensitive layer); (2) an interlayer to be disposed between adjacent photosensitive layers or between a photosensitive layer and a protective layer; (3) an undercoat layer to be disposed between a photosensitive layer and a support; (4) a back layer to be disposed on a support opposite to a photosensitive layer. The layers (1) and (2) are filter layers that are in the photothermographic material. The layers (3) and (4) are antihalation layers in the material.

### <<Surface Protective Layer>>

The photothermographic material of the first embodiment of the invention may have a surface protective layer for preventing the image-forming layer from being blocked. The surface protective layer may have a single-layered or multi-layered structure. The details of the surface protective layer are described, for example, in JP-A 11-65021, paragraphs [0119] to [0120], and in Japanese Patent Application No. 2000-171936.

Gelatin is preferred for the binder in the surface protective layer in the first embodiment of the invention, but for it, polyvinyl alcohol (PVA) is also usable alone or combined with gelatin. Gelatin for use herein may be inert gelatin (e.g., Nitta Gelatin 750), or gelatin phthalide (e.g., Nitta Gelatin 801).

Examples of PVA usable herein are described in, for example, JP-A 2000-171936, paragraphs [0009] to [0020]. Preferred example of PVA for use herein are completely saponified PVA-105; partially saponified PVA-205, PVA-355; and modified polyvinyl alcohol, MP-203 (all commercial products of Kuraray). The polyvinyl alcohol content (per m² of the support) of one protective layer preferably falls between 0.3 and 4.0 g/ m², more preferably between 0.3 and 2.0 g/m².

In case where the photothermographic material of the first embodiment of the invention is used in the field of printing that require high-level dimensional stability, it is desirable to use a polymer latex in the surface protective layer or the back layer of the material.

The polymer latex for that purpose is described in, for example, Synthetic Resin Emulsions (by Taira Okuda & Hiroshi Inagaki, the Polymer Publishing Association of Japan, 1978); Applications of Synthetic Latexes (by Takaaki Sugimura, Yasuo Kataoka, Sohichi Suzuki & Keiji Kasahara, the Polymer Publishing Association of Japan, 1993); and Chemistry of Synthetic Latexes (by Sohichi Muroi, the Polymer Publishing Association of Japan, 1970). Concretely, it includes, for example, methyl methacrylate (33.5 wt.%)/ethyl acrylate (50 wt.%)/methacrylic acid (16.5 wt.%) copolymer latex; methyl methacrylate (47.5 wt.%)/butadiene (47.5 wt.%)/itaconic acid (5 wt.%) copolymer latex; ethyl acrylate/methacrylic acid copolymer latex; methyl methacrylate (58.9 wt.%)/2-ethylhexyl acrylate (25.4 wt.%)/styrene (8.6 wt.%) / 2-hydroxyethyl methacrylate (5.1 wt.%)/acrylic acid (2.0 wt.%) copolymer latex; and methyl methacrylate (64.0 wt.%)/styrene (9.0 wt.%)/butyl acrylate (20.0 wt.%)/2-hydroxyethyl methacrylate (5.0 wt.%)/acrylic acid (2.0 wt.%) copolymer latex.

To the binder for the surface protective layer in this embodiment, for example, applicable are the polymer latex combinations as in Japanese Patent Application No. 11-6872; the techniques as in Japanese Patent Application No. 11-143058, paragraphs [0021] to [0025]; the techniques as in Japanese Patent Application No. 11-6872, paragraphs [0027] to [0028]; and the techniques as in Japanese Patent Application No. 10-199626, paragraphs [0023] to [0041].

The ratio of the polymer latex in the surface protective layer preferably falls between 10 % by weight and 90 % by weight, more preferably between 20 % by weight and 80 % by weight of all the binder in the layer.

The overall binder content (including water-soluble polymer and latex polymer, per m² of the support) of one protective layer preferably falls between 0.3 and 5.0 g/ m², more preferably between 0.3 and 2.0 g/m².

### <<Antihalation Layer>>

Preferably, the photothermographic material of the first embodiment of the invention has an antihalation layer remoter from the light source to which it is exposed than its photosensitive layer.

The details of the antihalation layer are described in, for example, JP-A 11-65021, paragraphs [0123] to [0124]; JP-A 11-223898, 9-230531, 10-36695, 10-104779, 11-231457, 11-352625, 11-352626.

The antihalation layer contains an antihalation dye capable of absorbing the light to which the photothermographic material is exposed. In this embodiment, the photothermographic material is exposed to laser rays having a peak wavelength range of from 350 nm to 440 nm. Therefore, it is desirable that the antihalation dye to be in the antihalation layer of the material may absorb the light falling within that wavelength range.

In case where visible light-absorbing dyes are used for antihalation in this embodiment, it is desirable that the dyes used are substantially decolored after image formation on the material, for which, for example, usable are decoloring agents that have the ability to decolor the dyes when heated in the step of thermal development. Preferably, a thermal decoloring dye and a base precursor are added to the non-photosensitive layers so that the layers containing them may function as antihalation layers. The details of this technique are described in, for example, JP-A 11-231457.

The amount of the decoloring dye to be added shall be determined, depending on the use of the dye. In general, its amount is so determined that the dye added could ensure an optical density (absorbance), measured at an intended wavelength, of larger than 1.0. The optical density preferably falls between 0.15 and 2, more preferably between 0.2 and 1. The amount of the dye capable of ensuring the optical density falling within the range may be generally from 0.001 to 1 g/m² or so.

Decoloring the dyes in the photothermographic material in that manner can lower the optical density of the material to 0.1 or less after thermal development. Two or more different types of decoloring dyes may be in the thermodecoloring recording material or the photothermographic material. Similarly, two or more different types of base precursors may be in the material.

In the thermodecoloring material of the type that contains a decoloring dye and a base precursor, it is desirable in view of the thermodecoloring ability of the material that the base precursor therein is combined with a substance which, when mixed with the base precursor, can lower the melting point of the mixture by at most 3°C (e.g., diphenyl sulfone, 4-chlorophenyl(phenyl) sulfone, 2-naphtyl benzoate), for example, as in JP-A 11-352626.

### <<Back Layer>>

For the details of the back layer applicable to the first embodiment of the invention, referred to is JP-A 11-65021, paragraphs [0128] to [0130].

In the first embodiment of the invention, a coloring agent that has an absorption maximum in the range falling between 300 and 450 nm may be added to the photothermographic material for improving the silver tone and the image stability of the material. The coloring agent is described in, for example, JP-A 62-210458, 63-104046, 63-1003235, 63-208846, 63-306436, 63-314535, 01-61745, and Japanese Patent Application No. 11-276751.

In general, the amount of the coloring agent to be added to the material falls between 0.1 mg/m² and 1 g/m². Preferably, it is added to the back layer that is opposite to the photosensitive layer of the material.

Preferably, the photothermographic material of the first embodiment of the invention has, on one surface of its support, at least one photosensitive layer that contains a photosensitive silver halide emulsion, and has a back layer on the other surface thereof. This is referred to as a single-sided photothermographic material.

### <<Matting Agent>>

Also preferably, the photothermographic material of the first embodiment of the invention contains a matting agent which is for improving the transferability of the material. Matting agents are described in JP-A 11-65021, paragraphs [0126] to [0127]. The amount of the matting agent to be added to the photothermographic material preferably falls between 1 and 400 mg/m², more preferably between 5 and 300 mg/m² of the material.

Regarding its morphology, the matting agent to be used in the first embodiment of the invention may be shaped or amorphous, but is preferably shaped. More preferably, it is spherical. The mean grain size of the spherical matting agent preferably falls between 0.5 and 10 µm, more preferably between 1.0 and 8.0 µm, even more preferably between 2.0 and 6.0 µm. The size distribution fluctuation coefficient thereof is preferably at most 50 %, more preferably at most 40 %, even more preferably at most 30 %. The fluctuation coefficient is represented by (grain size standard deviation) / (mean grain size) × 100. Combining two different types of matting agents both having a small size distribution fluctuation coefficient is preferred for use in this embodiment. Concretely, the ratio of the mean grain size of the two matting agents combined is larger than 3.

The degree to which the emulsion surface of the photothermographic material of this embodiment is matted is not specifically defined, so far as the matted layer surface is free from star dust trouble, but is preferably such that the Beck's smoothness of the matted surface could fall between 30 seconds and 2000 seconds, more preferably between 40 seconds and 1500 seconds. The Beck's smoothness is readily obtained according to JIS P8119 (method of testing surface smoothness of paper and paper boards with Beck tester), and to TAPPI Standard T479.

Regarding the matting degree of the back layer of the photothermographic material of the first embodiment of the invention, the Beck's smoothness of the matted back layer preferably falls between 10 seconds and 1200 seconds, more preferably between 20 seconds and 800 seconds, even more preferably between 40 seconds and 500 seconds.

Preferably, the photothermographic material of the first embodiment of the invention contains such a matting agent in the outermost surface layer, or in a layer functioning as an outermost surface layer, or in a layer nearer to the outermost surface. Also preferably, it may contain a matting agent in a layer functioning as a protective layer.

### <<pH of Film Surface>>

Also preferably, the surface of the photothermographic material of the first embodiment of the invention has a pH of at most 7.0, more preferably at most 6.6, before developed under heat. The lowermost limit of the pH is not specifically defined, but may be at least 3 or so. Most preferably, the pH range falls between 4 and 6.2.

For controlling the surface pH of the photothermographic material, employable are nonvolatile acids, for example, organic acids such as phthalic acid derivatives, or sulfuric acid, or nonvolatile bases such as ammonia. These are preferred as effective for reducing the surface pH of the material. Especially preferred for the surface pH-lowering agent is ammonia, as it is highly volatile, and therefore can be readily removed while the coating liquids containing it are coated and surely before thermal development.

Also preferred is combining ammonia with a nonvolatile base such as sodium hydroxide, potassium hydroxide or lithium hydroxide. For measuring the surface pH of the photothermographic material, referred to is the description in Japanese Patent Application No. 11-87297, paragraph [0123].

### <<Hardening Agent>>

A hardening agent may be added to the photosensitive layer, the protective layer, the back layer and other layers constituting the photothermographic material of the first embodiment of the invention. The details of the hardening agent applicable to the invention are described in T.H. James' The Theory of the Photographic Process, 4th Ed. (Macmillan Publishing Co., Inc., 1977), pp. 77-87. For example, preferred for use herein are chromium alum, 2,4-dichloro-6-hydroxy-s-triazine sodium salt, N,N-ethylenebis(vinylsulfonacetamide), N,N-propylenebis(vinylsulfonacetamide); as well as polyvalent metal ions described on page 78 of that reference; polyisocyanates described in USP 4,281,060 and JP-A 6-208193; epoxy compounds described in USP 4,791,042; and vinylsulfone compounds described in JP-A 62-89048.

The hardening agent is added to the coating liquids in the form of its solution. The time at which the solution is added to the coating liquid for the protective layer may fall between 180 minutes before coating the liquid and a time just before the coating, preferably between 60 minutes before the coating and 10 seconds before it. However, there is no specific limitation thereon, so far as the method and the condition employed for adding the hardening agent to the coating liquid ensure the advantages of the first embodiment of the invention.

Concretely for adding it, employable is a method of mixing a hardening agent with a coating liquid in a tank in such a controlled manner that the mean residence time for the agent as calculated from the amount of the agent added and the flow rate of the coating liquid to a coater could be a predetermined period of time; or a method of mixing them with a static mixer, for example, as in N. Harunby, M. F. Edwards & A. W. Nienow's Liquid Mixing Technology, Chap. 8 (translated by Koji Takahasi, published by Nikkan Kogyo Shinbun, 1989).

### <<Surfactants>>

Surfactants applicable to the photothermographic material of the first embodiment of the invention are described in JP-A 11-65021, paragraph [0132].

In the first embodiment of the invention, preferably used are fluorine-containing surfactants. Examples of fluorine-containing surfactants are given, for example, in JP-A 10-197985, 2000-19680 and 2000-214554. Also preferred for use herein are fluorine-containing polymer surfactants such as those in JP-A 9-281636. In the first embodiment of the invention, especially preferred are fluorine-containing surfactants described in Japanese Patent Application No. 2000-206560.

Solvents applicable to the first embodiment of the invention are described in JP-A 11-65021, paragraph [0133]; supports applicable thereto are in the same but in paragraph [0134]; antistatic and electroconductive layers applicable thereto are in the same but in paragraph [0135]; methods of forming color images applicable thereto are in the same but in paragraph [0136]; lubricants applicable thereto are in JP-A 11-84573, paragraphs [0061] to [0064] and in Japanese Patent Application No. 11-106881, paragraphs [0049] to [0062].

### <<Electroconductive Layer>>

Preferably, the photothermographic material of the first embodiment of the invention has an electroconductive layer with a metal oxide therein. For the electroconductive material for the electroconductive layer, preferred are metal oxides which are specifically so processed that they have oxygen defects and/ or different metal atoms introduced thereinto to increase their electroconductivity.

Preferred examples of the metal oxides are ZnO, TiO₂ and SnO₂. To ZnO, preferably added is any of Al or In; to SnO₂, any of Sb, Nb, P or halogen elements; and TiO₂, any of Nb or Ta. Especially preferred is SnO₂ with Sb added thereto.

Preferably, the amount of the different atom to be added to the metal oxide falls between 0.01 and 30 mol%, more preferably between 0.1 and 10 mol%. Regarding their morphology, the metal oxides may be spherical, acicular or tabular, but they are preferably acicular grains having a ratio of major axis/minor axis of at least 2.0, more preferably from 3.0 to 50 as their electroconductivity is high.

The amount of the metal oxide to be in the layer preferably falls between 1 mg/m² and 1000 mg/m², more preferably between 10 mg/m² and 500 mg/m², even more preferably between 20 mg/m² and 200 mg/m². In the first embodiment of the invention, the electroconductive layer may be formed on any side of emulsion-coated face or back face, but is preferably formed between the support and the back layer. Specific examples of the electroconductive layer applicable to the first embodiment of the invention are described in, for example, JP-A 7-295146 and 11-223901.

### <<Support>>

Various supports are employable in the photothermographic material of the first embodiment of the invention. They include, for example, polyesters such as polyethylene terephthalate (PET), polyethylene naphthalate; cellulose nitrate, cellulose esters, polyvinyl acetal, syndiotactic polystyrene, polycarbonates; and paper of which both surfaces are coated with polyethylene.

Preferably, the support of the photothermographic material of this embodiment is undercoated, for example, with a water-soluble polyester as in JP-A 11-84574; a styrene-butadiene copolymer as in JP-A 10-186565; or a vinylidene chloride copolymer as in JP-A 2000-39684 or in Japanese Patent Application No. 11-106881, paragraphs [0063] to [0080].

For the transparent supports for the photothermographic material, preferred are biaxially-stretched films of polyesters, especially polyethylene terephthalate heated at a temperature falling between 130 and 185°C. The heat treatment is for removing the internal strain that may remain in the biaxially-stretched films and for preventing the film supports from being thermally shrunk during thermal development of the material. In case where the photothermographic material is for medical treatment, the transparent support for it may be colored with a blue dye (for example, with Dye-1 used in the examples in JP-A 8-240877), or may not be colored.

For the antistatic layer and the undercoat layer to be formed in the photothermographic material of the first embodiment of the invention, for example, referred to are the techniques disclosed in JP-A 56-143430, 56-143431, 58-62646, 56-120519, 11-84573, paragraphs [0040] to [0051]; USP 5,575,957; and JP-A 11-223898, paragraphs [0078] to [0084].

Preferably, the photothermographic material is of a monosheet type. The monosheet type does not require any additional sheet to receive images thereon, but may directly form images on itself.

### <<Other Additives>>

The photothermographic material may optionally contain an antioxidant, a stabilizer, a plasticizer, a UV absorbent or a coating aid. Such additives may be in any of the photosensitive layers or the non-photosensitive layers of the material. For the additives, for example, referred to are WO98/36322, EP 803764A1, JP-A 10-186567 and 10-18568.

### <Fabrication of Photothermographic Material>

To fabricate the photothermographic material of the first embodiment of the invention, the coating liquids may be applied onto a support in any desired manner. Concretely, various types of coating techniques are employable herein, including, for example, extrusion coating, slide coating, curtain coating, dipping, knife coating, and flow coating. Various types of hoppers for extrusion coating employable herein are described in USP 2,681,294. Preferred for the photothermographic material is extrusion coating or slide coating described in Stephen F. Kistler & Petert M. Schweizer's Liquid Film Coating (Chapman & Hall, 1997), pp. 399-536. More preferred is slide coating. One example of the shape of a slide coater for slide coating is in Figure 11b-1, on page 427 of that reference. If desired, two or more layers may be formed at the same time, for example, according to the methods described from page 399 to page 536 of that reference, or to the methods described in USP 2,761,791 and BP 837,095.

Preferably, the coating liquid for the organic silver salt-containing layer in the first embodiment of the invention is a thixotropic flow. For it, referred to is the technique described in JP-A 11-52509.

Preferably, the coating liquid for the organic silver salt-containing layer in the first embodiment of the invention has a viscosity falling between 400 mPa·s and 100,000 mPa·s, more preferably between 500 mPa·s and 20,000 mPa·s, at a shear rate of 0.1 sec⁻¹. Also preferably, the viscosity falls between 1 mPa·s and 200 mPa·s, more preferably between 5 mPa·s and 80 mPa·s, at a shear rate of 1000 sec⁻¹.

Other techniques applicable to the photothermographic material of the first embodiment of the invention are, for example, in EP 803764A1, EP 883022A1, WO98/36322; JP-A 56-62648, 58-62644, 9-43766, 9-281637, 9-297367, 9-304869, 9-311405, 9-329865, 10-10669, 10-62899, 10-69023, 10-186568, 10-90823, 10-171063, 10-186565, 10-186567, 10-186569 to 10-186572, 10-197974, 10-197982, 10-197983, 10-197985 to 10-197987, 10-207001, 10-207004, 10-221807, 10-282601, 10-288823, 10-288824, 10-307365, 10-312038, 10-339934, 11-7100, 11-15105, 11-24200, 11-24201, 11-30832, 11-84574, 11-65021, 11-109547, 11-125880, 11-129629, 11-133536 to 11-133539, 11-133542, 11-133543, 11-223898, 11-352627, 11-305377, 11-305378, 11-305384, 11-305380, 11-316435, 11-327076, 11-338096, 11-338098, 11-338099, 11-343420; and Japanese Patent Application Nos. 2000-187298, 2000-10229, 2000-47345, 2000-206642, 2000-98530, 2000-98531, 2000-113059, 2000-112060, 2000-112104, 2000-112064, 2000-171936.

### <Packaging Material for Photothermographic Material>

Preferably, the photothermographic material of the first embodiment of the invention is wrapped with a material of low oxygen and/or moisture permeability for preventing its photographic properties from varying and for preventing it from curling or from having a curled habit while stored as raw films.

Preferably, the oxygen permeability at 25°C of the packaging material for use herein is at most 50 ml/atm·m²·day, more preferably at most 10 ml/atm·m²·day, even more preferably at most 1.0 ml/atm·m²·day. Also preferably, the moisture permeability thereof is at most 10 g/atm·m²·day, more preferably at most 5 g/atm·m²·day, even more preferably at most 1 g/atm·m²·day.

Preferred examples of the packaging material of low oxygen and/or moisture permeability for use herein are described, for example, in JP-A 8-254793, 2000-206653.

### <Exposure and Thermal Development>

A seventh embodiment of the present invention is a method of thermal development of a photothermographic material, which comprises a support having thereon a layer including at least a non-photosensitive organic silver salt, a photosensitive silver halide, a reducing agent and a binder; wherein the photosensitive silver halide has a mean silver iodide content of 5 to 100 mol %, and which further comprises at least one compound of the following general formula (I), wherein the highest temperature at thermal development of the photothermographic material is 100 to 120°C.

General formula (I) (X)ₖ―L)ₘ―(A-B)ₙ

wherein X represents a silver halide-adsorbing group or a light-absorbing group that has at least one atom each of N, S, P, Se and Te; L represents a (k + n)-valent linking group having at least one atom each of C, N, S and O; A represents an electron-donating group; B represents a leaving group or a hydrogen group; A-B is oxidized and then cleaved or deprotonated to generate a radical A; k represents an integer from 0 to 3; m represents 0 or 1; n represents 1 or 2; and when k = 0 and n = 1, then m = 0;

In the method of the present invention, the highest temperature of thermal development of the photothermographic material is preferably 105 to 115°C.

In the method of the present invention, preferably, the photothermographic material is thermally developed while being conveyed through a thermal development zone that comprises from 2 to 6 plate heaters for thermal development and while being kept in contact with the plate heaters in that zone.

In the method of the present invention, the mean grain size of the silver halide is preferably 5 to 80 nm, more preferably 5 nm to 70 nm.

The photothermographic material of the first embodiment of the invention may be developed in any manner. In general, after having been imagewise exposed, it is developed under heat. Preferably, the temperature for the thermal development falls between 80 and 250°C, more preferably between 100 and 140°C, even more preferably between 100 and 120°C, most preferably between 105 and 115°C. The time for the development preferably falls between 1 and 60 seconds, more preferably between 5 and 25 seconds, even more preferably between 7 and 15 seconds.

For thermal development for the photothermographic material, employable is any of a drum heater system or a plate heater system, but preferred is a plate heater system. For the plate heater system for the material, preferred is the method described in JP-A 11-133572. The plate heater system described therein is for thermal development of photothermographic materials, in which a photothermographic material having been exposed to have a latent image thereon is brought into contact with a heating unit in the zone for thermal development to thereby convert the latent image into a visible image. In this, the heating unit comprises a plate heater, and multiple presser rolls are disposed in series on one surface of the plate heater. The exposed photothermographic material is passed between the multiple pressure rolls and the plate heater, whereby it is developed under heat. The plate heater is sectioned into 2 to 6 stages, and it is desirable that the temperature of the top stage is kept lower by 1 to 10°C or so than that of the others.

For example, four pairs of plate heaters of which the temperature is independently controllable may be used, and they are set at 112°C, 119°C, 121°C and 120°C. The system of the type is described in JP-A 54-30032. In the plate heater system, water and organic solvent that remain in the photothermographic material being processed can be removed out of the material. In this, in addition, the support of the photothermographic material rapidly heated is prevented from being deformed.

Preferably, the photothermographic material of the first embodiment of the invention is exposed to high-intensity light of at least 1 mW/mm² within a short period of time. The sensitivity of the photothermographic material of this embodiment that contains a high-iodide silver halide emulsion and a non-photosensitive organic silver salt is enough for exposure to such high-intensity light. For the photothermographic material of this embodiment, exposure to high-intensity light is preferred to exposure to low-intensity light in point of the sensitivity of the material.

More preferably, the intensity of light to which the material is exposed falls between 2 mW/mm² and 50 mW/mm², even more preferably between 10 mW/mm² and 50 mW/mm².

The light source for the photothermographic material of this embodiment may be any and every one of the type, for which, however, preferred are laser rays as producing better results.

For the laser rays to which the photothermographic material of the first embodiment of the invention is exposed, preferred are gas lasers (Ar⁺, He-Ne), YAG lasers, color lasers, or semiconductor lasers. Also employable is a combination of semiconductor lasers and secondary harmonics generators. Especially preferred are gas or semiconductor lasers for red to infrared emission. Also preferred are semiconductor lasers for blue to violet emission. One example of high-power semiconductor lasers for blue to violet emission that are employable herein is a Nichia Chemical's semiconductor laser, NLHV300E.

One example of laser imagers for medical treatment equipped with an exposure unit and a thermal development unit that are applicable to this embodiment of the invention is Fuji Medical Dry Laser Imager FM-DP L.

The system FM-DP L is described in Fuji Medical Review No. 8, pp. 39-55. Needless-to-say, the technique disclosed therein is applicable to laser imagers for the photothermographic material of the first embodiment of the invention. In addition, the photothermographic material of this embodiment can be processed in the laser imager in the AD Network which Fuji Medical System has proposed for a network system under DICOM Standards.

The photothermographic material of the first embodiment of the invention forms a monochromatic image based on silver, and is favorable for use in medical diagnosis, industrial photography, printing, and COM.

### EXAMPLES

### -Examples of First Embodiment-

Hereinafter, a first embodiment of a photothermographic material according to the present invention will be explained in more detail with reference to examples. However, the first embodiment according to the invention is by no means limited to these examples.

### Example 1

### Preparation of PET Support

PET with an intrinsic viscosity (IV) of 0.66 (measured in phenol/tetrachloroethane=6/4 (ratio by mass) at 25°C) was obtained by a general procedure by using terephthalic acid and ethylene glycol. The thus-obtained PET was pelletized, dried at 130°C for 4 hours, melted at 300°C, extruded from a T-die and rapidly cooled to obtain an unstretched film having a thickness of 175 µm on an after-heat-setting basis.

The film was then longitudinally stretched 3.3 times by using rollers which are different in a peripheral speed from each other and then transversely stretched 4.5 times by using a tenter. Temperatures applied in these cases were 110°C and 130°C, respectively. Subsequently, the film was heat-set at 240°C for 20 seconds, and then relaxed by 4% in the transverse direction at a same temperature. Thereafter, a portion chucked by the tenter was slit off and the film was knurled at both edges thereof and then taken up at a rate of 4 kg/cm² to obtain a rolled support having a thickness of 175 µm.

### Surface Corona Treatment

Using a solid state corona treatment apparatus (model: 6KVA; available from Pillar Corporation), both surfaces of the support were subjected to a corona treatment at 20 m/minute at room temperature. Referring to read values of current and voltage, it was confirmed that the support was treated at 0.375 kVA·minute/m². Frequency for the treatment was 9.6 kHz and a gap clearance between an electrode and a dielectric roll was 1.6 mm.

### Preparation of Undercoated Support

### Preparation of Coating Liquid for Undercoat Layer

### <Formulation 1: for Undercoat Layer on Photosensitive Layer Side>

| | |
|---|---|
| "PESRESIN A-520" available from Takamatsu Oil & Fat Co., Ltd. (30 mass% solution) | 59 g |
| polyethylene glycol monononylphenyl ether (average ethylene oxide number: 8.5) 10 mass% solution | 5.4 g |
| "MP-1000" (polymer fine particles; average particle diameter: 0.4µm) available from Soken Chemical & Engineering Co., Ltd.) | 0.91 g |
| distilled water | 935 ml |

### <Formulation 2: for First Layer on Back Surface Side>

| | |
|---|---|
| styrene-butadiene copolymer latex (solid content: 40 mass%; a ratio of styrene / butadiene by mass: 68 / 32) | 158 g |
| 2,4-dichloro-6-hydroxy-S-triazine sodium salt (8 mass% aqueous solution) | 20 g |
| sodium laurylbenzene sulfonate (1 mass% aqueous solution) | 10 ml |
| distilled water | 854 ml |

### <Formulation 3: for Second Layer on Back Surface Side>

| | |
|---|---|
| SnO₂/SbO (ratio by mass: 9/1; average particle dismeter: 0.038 µm; 17 mass% dispersion) | 84 g |
| gelatin (10 mass% aqueous solution) | 89.2 g |
| "METHOLLOSE TC-5" available from Shin-Etsu Chemical Co., Ltd. (2 mass% aqueous solution) | 8.6 g |
| "MP-1000" available from Soken Chemical & Engineering Co., Ltd. | 0.01 g |
| Sodium dodecylbenzene sulfonate (1 mass% aqueous solution) | 10 ml |
| NaOH (1 mass%) | 6 ml |
| "PROXEL" available from ICI Corporation | 1 ml |
| distilled water | 805 ml |

After both surfaces of the biaxially stretched polyethylene terephthalate film of 175 µm thick were individually subjected to the corona discharge treatment, the composition 1 of the coating liquid for undercoat was coated on one surface (photosensitive layer side) by using a wire bar in a wet coated amount of 6.6 ml/m² (for one side) and was allowed to dry at 180°C for 5 minutes. The composition 2 of the coating liquid for undercoat was coated on a back surface by using a wire bar in a wet coated amount of 5.7 ml/m² and, then, allowed to dry at 180°C for 5 minutes and, further, the composition 3 of the coating liquid for undercoat was coated on the back surface by using a wire bar in a wet coated amount of 7.7 ml/m² and, then, allowed to dry at 180°C for 6 minutes, thereby to obtain an undercoated support.

### Preparation of Coating Liquid for Back Surface

### Preparation of Solid Fine Particle Dispersion (a) of Basic Precursor

1.5 kg of a basic precursor compound 1, 225 g of an surfactant (trade name: DEMOL-N; available from Kao Corporation), 937.5 g of diphenylsulfone and 15 g of parahydroxy benzoic acid butyl ester (trade name: Mekkinsu; available from Ueno Pharmaceutical Co., Ltd.) were mixed and, further, made up to be 5.0 kg in a total weight by being added with distilled water and, then, the resultant mixture was bead-dispersed by using a lateral sand mill (UVM-2; available from Aimex, Ltd.). As for a dispersion method, the mixture was fed to the UVM-2 filled with zirconia beads having an average diameter of 0.5 mm by using a diaphragm pump and dispersed under an inner pressure of 50 hPa or more until a desired average particle diameter was obtained.

Such dispersion processing has been performed until a dispersion in which, as a result of spectral absorption measurements, a ratio (D450/D650) of absorbance at 450 nm against that at 650 nm derived from spectral absorption of the dispersion was 2.2 or more was obtained. The thus-obtained dispersion was diluted with distilled water such that a concentration of the basic precursor was 20 mass %, filtered (using a filter made of polypropylene having an average pore diameter of 3 µm) to remove dust and put for practical use.

### Preparation of Solid Fine Particle Dispersion of Dye

6.0 kg of a cyanine dye compound-1, 3.0 kg of sodium p-dodecylbenzene sulfonate, 0.6 kg of a surfactant DEMOL SNB available from Kao Corporation and 0.15 kg of an antifoaming agent (trade name: Surfynol 104E; available from Nissin Chemical Industry Co., Ltd.) were mixed and made up to be 60 kg in a total weight by being added with distilled water. The resultant mixture was dispersed by zirconia beads by using a lateral sand mill (UVM-2; available from Aimex, Limited).

Such dispersion processing has been performed until a dispersion in which, as a result of spectral absorption measurements, a ratio (D650/D750) of absorbance at 650 nm against that at 750 nm derived from spectral absorption of the dispersion was 5.0 or more was obtained. The thus-obtained dispersion was diluted with distilled water such that a concentration of the cyanine dye was 6 mass %, filtered (average pore diameter of filter: 1 µm) to remove dust and put for practical use.

### Preparation of Coating Liquid for Anti-halation Layer

30 g of gelatin, 24.5 g of polyacrylamide, 2.2 g of 1 mol/l caustic soda, 2.4 g of monodispersed polymethyl methacrylate fine particles (average particle size: 8 µm; particle diameter standard deviation: 0.4), 0.08 g of benzoisothiazolinone, 35.9 g of the above-described solid fine particle dispersion of dye, 74.2 g of the above-described solid fine particle dispersion (a) of the basic precursor, 0.6 g of sodium polyethylenesulfonate, 0.21 g of a blue dye compound-1, 0.15 g of a yellow dye compound-1 and 8.3 g of acrylic acid/ethyl acrylate copolymerization latex (copolymerization ratio: 5/95) were mixed and made up to be 8183 ml in a total volume by being added with water, thereby to prepare a coating liquid for the anti-halation layer.

### Preparation of Coating Liquid for Protective Layer on Back Surface

While keeping a temperature of a vessel at 40°C, 40 g of gelatin, 1.5 g of liquid paraffin emulsion in terms of liquid paraffin, 35 mg of benzoisothiazolinone, 6.8 g of 1 mol/l caustic soda, 0.5 g of sodium t-octylphenoxyethoxyethane sulfonate, 0.27 g of sodium polystyrene sulfonate, 37 mg of a fluorinated surfactant (F-1: N-perfluorooctylsulfonyl-N-propylalanine potassium salt), 150 mg of a fluorinated surfactant (F-2: polyethylene glycol mono(N-perfluorooctylsulfonyl-N-propyl-2-aminoethyl) ether [average degree of polymerization of ethylene oxide: 15], 64 mg of a fluorinated surfactant (F-3), 32 mg of a fluorinated surfactant (F-4), 6.0 g of acrylic acid/ethyl acrylate copolymer (copolymerization ratio by mass: 5/95) and 2.0 g of N,N-ethylenebis(vinyl sulfone acetamide) were mixed and made up to be 10 liter by being added with water, thereby to obtain a coating liquid for the protective layer on the back surface.

### Preparation of Silver Halide Emulsion

### <Preparation of Silver Halide Emulsion 1>

To 1,421 ml of water, added were 3.1 ml of a 1 mass% potassium bromide solution, 3.5 ml of a 0.5 mol/L concentration of sulfuric acid and 31.7 g of phthalized gelatin; while the resultant liquid was kept stirring in a stainless-steel reaction vessel at a constant liquid temperature of 35°C, was added thereto an entire volume of a solution A in which 22.22 g of silver nitrate was diluted by distilled water to be 195.6 ml and a solution B in which 13.7 g of potassium bromide and 2.6 g of potassium iodide were diluted by distilled water to be 218 ml at a constant flow rate over 45 seconds. Thereafter, the resultant solution was added with 10 ml of a 3.5 mass% aqueous hydrogen peroxide solution and, further, with 10.8 ml of a 10 mass% aqueous solution of benzoimidazole.

Further, was added thereto an entire volume of a solution C in which 51.86 g of silver nitrate was diluted with distilled water to be 317.5 ml and a solution D in which 31.9 g of potassium bromide and 6.1 g of potassium iodide were diluted with distilled water to be 600 ml such that an entire volume of the solution C was added thereto at a constant flow rate over 120 minutes and the solution D was added thereto by a controlled double jet method while a pAg thereof is kept at 8.1. Further, added thereto was an entire volume of potassium hexachloroiridate(III) 10 minutes after the solution C and the solution D started to be added so as to attain a concentration of 1X10⁻⁴ mol/mol of Ag. Furthermore, an entire volume of 3X10⁻⁴ mol/mol of Ag of an aqueous solution of potassium iron (II) hexacyanate was added 5 minutes after completion of such an addition of the solution C. At the point of time when the pH of the resultant mixture was adjusted to be 3.8 by using a 0.5 mol/L concentration of sulfuric acid, stirring is stopped and the resultant mixture was subjected to sedimentation/desalting/rinsing operations. Thereafter, the pH of the mixture was adjusted to be 5.9 by using a 1 mol/L concentration of sodium hydroxide to prepare a silver halide dispersion having a pAg of 8.0.

Subsequently, while the thus-prepared silver halide dispersion was kept stirring at 38°C, the dispersion was added with 5 ml of a 0.34 mass% methanol solution of 1,2-benzisothiazolin-3-one and, 40 minutes after such an addition, added with a methanol solution of mixture of a spectral sensitizing dye A and a spectral sensitizing dye B at a mixing ratio of 1:1 in an amount of 1.2X10⁻³ mol/mol of Ag and, one minute after the above addition, a temperature of the resultant dispersion was raised to 47°C. 20 minute after such temperature raising, the resultant dispersion was added with a methanol solution of sodium benzene thiosulfonate in an amount of 7.6X10⁻⁵ mol/mol of Ag and, further, 5 minutes after such an addition, added with a methanol solution of a tellurium sensitizer C in an amount of 2.9X10⁻⁴ mol/mol of Ag and, then, ripened for 91 minutes. Thereafter, the resultant dispersion was added with 1.3 ml of a 0.8 mass% methanol solution of N,N'-dihydroxy-N"-diethylmelamine and, 4 minutes after such an addition, added with a methanol solution of 5-methyl-2-mercaptobenzoimidazole in an amount of 4.8X10⁻³ mol/mol of Ag, a methanol solution of 1-phenyl-2-heptyl-5-mercapto-1,3,4-triazole in an amount of 5.4X10⁻³ mol/mol of Ag and an aqueous solution of a mercapto compound-2 in an amount of 1.5X10⁻² mol/mol of Ag, thereby to obtain a silver halide emulsion 1.

Particles contained in the thus-prepared silver halide emulsion were silver iodobromide particles uniformly containing 12 mol% of iodide having an average sphere-equivalent diameter of 0.042 µm and a sphere-equivalent coefficient of variation of 18%. On this occasion, a particle size and the like were determined based on an average of 1000 particles under an electron microscopic observation.

### <Preparation of Mixed Emulsion A for Coating Liquid>

The silver halide emulsion 1 was dissolved and, then, added with a 1 mass% aqueous solution of benzothiazolium iodide in an amount of 7X10⁻³ mol/mol of Ag. Subsequently, the resultant emulsion was added with a compound expressed by a general formula (1) shown in Table 1 in an amount of 1X10⁻³ mol/mol of Ag and, further, added with water such that a content of silver halide becomes 38.2 g in terms of silver per kg of the mixed emulsion for coating liquid.

### <Preparation of Fatty Acid Silver Dispersion>

87.6 kg of behenic acid (trade name: "Edenor C22-85R"; available from Henkel Corporation), 423 L of distilled water, 49.2 L of a 5 mol/L concentration of an aqueous NaOH solution and 120 L of t-butyl alcohol were mixed and, then, the resultant mixture was stirred at 75°C for one hour to allow the mixture to react, thereby to obtain a sodium behenate solution. Separately, 206.2 L (pH 4.0) of an aqueous solution containing 40.4 kg of silver nitrate was prepared and kept at 10°C. A reaction vessel containing 635 L of distilled water and 30 L of t-butyl alcohol was kept at 30°C and, then, was added with an entire volume of the thus-obtained sodium behenate solution and an entire volume of the aqueous silver nitrate solution each at a constant flow rate over 93 minutes and 15 seconds and over 90 minutes, respectively, while being thoroughly mixed.

On this occasion, only the aqueous silver nitrate solution was added in a first 11-minute period after the start of addition thereof and, then, the sodium behenate solution was started to be added and only the sodium behenate solution was added in a last 14-minute-and-15 second period after the end of addition of the aqueous silver nitrate solution. At this time, a temperature in the reaction vessel was kept at 30°C and was controlled externally so as to keep the liquid temperature constant.

A piping in a feeding system of the sodium behenate solution was heated by circulating hot water in an outer portion of a double pipe and controlled such that an outlet liquid temperature at the end of the feed nozzle was 75°C. Further, A piping in a feeding system of the aqueous silver nitrate solution was cooled by circulating cold water in an outer portion of the double pipe. A point of addition of the sodium behenate solution and a point of addition of the aqueous silver nitrate solution were symmetrically arranged centered around a stirring axis and these points were adjusted high enough to prevent them from contacting the reaction solution.

After completion of such an addition of the sodium behenate solution, the resultant mixture was allowed to stand for 20 minutes under stirring with a temperature thereof unchanged, and, then, the temperature was elevated to 35°C over 30 minutes and, thereafter, ripened for 210 minutes. Immediately after completion of such ripening, a solid content was separated by centrifugal filtration and, then, rinsed with water until electric conductivity of a filtrate became 30 µS/cm. Thus, a fatty acid silver salt was obtained. The thus-obtained solid content was stored in wet cake form without being dried.

When a state of the thus-obtained silver behenate particles was observed by a microscopic photographing, the obtained silver behenate particles were found to be a scaly crystal having average values of a=0.14 µm, b=0.4 µm and c=0.6 µm, an average aspect ratio of 5.2, an average sphere-equivalent diameter of 0.52 µm and a sphere-equivalent coefficient of variation of 15% (a, b and c being defined in this specification).

To the wet cake equivalent to dry weight of 260 kg, 19.3 kg of polyvinyl alcohol (trade name; "PVA-217") was added and water was further added to make a total volume up to be 1000 kg and, then, the resultant mixture was changed into a slurry state by using a dissolver blade and, thereafter, preliminarily dispersed by using a pipeline mixer ("PM-10"; available from Mizuho Industrial Co., Ltd.).

Next, such a preliminarily dispersed stock solution was dispersed three times by using a dispersion apparatus (trade name: "Micro Fluidizer-M-610"; available from Micro Fluidex International Corporation) equipped with a Z type interaction chamber under a pressure of 1260 kg/cm², thereby to obtain a silver behenate dispersion. During the dispersion, cooling operation was performed such that coiled heat exchangers were attached each to an inlet and an outlet of the interaction chamber and a temperature of coolant was controlled to keep the dispersion temperature at 18°C.

### Preparation of Reducing Agent Dispersion

### <Preparation of Reducing Agent-1 Dispersion>

10 kg of a reducing agent-1, that is, 6,6'-di-t-butyl-4,4'-dimethyl-2,2'-butylidene diphenol and 16 kg of a 10 mass% aqueous solution of a modified polyvinylalcohol ("Poval MP203"; available from Kuraray Co., Ltd.) were added with 10 kg of water and, then, mixed thoroughly to prepare a slurry. The thus-prepared slurry was fed by using a diaphragm pump to a lateral sand mill ("UVM-2"; available from Aimex, Ltd.) filled with zirconia beads having an average diameter of 0.5 mm, dispersed for 3 hours and 30 minutes, added with 0.2 g of a benzoisothiazolinone sodium salt and water such that a concentration of the reducing agent was adjusted to be 25 mass%, thereby to obtain a reducing agent-2 dispersion. Reducing agent particles contained in the thus-obtained reducing agent dispersion were found to have a median diameter of 0.40 µm and a maximum particle diameter of 1.5 µm or less. The obtained reducing agent dispersion was filtered through a polypropylene filter having a pore diameter of 3.0 µm to separate dust or other foreign matters and then stored.

### <Preparation of Hydrogen Bonding Type Compound-1 Dispersion>

10 kg of a hydrogen bonding type compound-1, that is, tri(4-t-butylphenyl)phosphine oxide and 16 kg of a 10 mass% aqueous solution of a modified polyvinylalcohol ("Poval MP203"; available from Kuraray Co., Ltd.) were added with 10 kg of water and, then, mixed thoroughly to prepare a slurry. The thus-prepared slurry was fed by using a diaphragm pump to a lateral sand mill ("UVM-2"; available from Aimex, Ltd.) filled with zirconia beads having an average diameter of 0.5 mm, dispersed for 3 hours and 30 minutes, added with 0.2 g of a benzoisothiazolinone sodium salt and water such that a concentration of the reducing agent was adjusted to be 25 mass%, thereby to obtain a hydrogen bonding type compound-1 dispersion. Reducing agent particles contained in the thus-obtained reducing agent dispersion were found to have a median diameter of 0.35 µm and a maximum particle diameter of 1.5 µm or less. The obtained hydrogen bonding type compound dispersion was filtered through a polypropylene filter having a pore diameter of 3.0 µm to separate dust or other foreign matters and then stored.

### <Preparation of Development Accelerator-1 Dispersion>

10 kg of a development accelerator-1 and 20 kg of a 10 mass% aqueous solution of a modified polyvinylalcohol (Poval MP203; available from Kuraray Co., Ltd.) were added with 10 kg of water and, then, mixed thoroughly to prepare a slurry. The thus-prepared slurry was fed by using a diaphragm pump to a lateral sand mill (UVM-2; available from Aimex, Ltd.) filled with zirconia beads having an average diameter of 0.5 mm, dispersed for 3 hours and 30 minutes, added with 0.2 g of a benzoisothiazolinone sodium salt and water such that a concentration of the reducing agent was adjusted to be 20 mass%, thereby to obtain a development accelerator-1 dispersion. Reducing agent particles contained in the thus-obtained reducing agent dispersion were found to have a median diameter of 0.48 µm and a maximum particle diameter of 1.4 µm or less. The obtained reducing agent dispersion was filtered through a polypropylene filter having a pore diameter of 3.0 µm to separate dust or other foreign matters and then stored.

As for respective solid dispersions of a development accelerator-2, a development accelerator-3 and a color tone controlling agent-1, dispersion operations were performed in a same manner as in the development accelerator-1 to obtain respective 20 mass% dispersions.

### Preparation of Polyhalogen Compound

### <Preparation of Organic Polyhalogen Compound-1 Dispersion>

10 kg of an organic polyhalogen compoun-1, that is, tribromomethane sulfonylbenzene, 10 kg of a 20 mass% aqueous solution of a modified polyvinylalcohol (Poval MP203; available from Kuraray Co., Ltd.) and 0.4 kg of a 20 mass% aqueous solution of sodium triisopropylnaphthalene sulfonate were added with 14 kg of water and, then, mixed thoroughly to prepare a slurry. The thus-prepared slurry was fed by using a diaphragm pump to a lateral sand mill (UVM-2; available from Aimex, Ltd.) filled with zirconia beads having an average diameter of 0.5 mm, dispersed for 5 hours, added with 0.2 g of a benzoisothiazolinone sodium salt and water such that a concentration of an organic polyhalogen compound was adjusted to be 26 mass%, thereby to obtain an organic polyhalogen compound-1 dispersion. Organic polyhalogen compound particles contained in the thus-obtained polyhalogen compound dispersion were found to have a median diameter of 0.41 µm and a maximum particle diameter of 2.0 µm or less. The obtained organic polyhalogen compound dispersion was filtered through a polypropylene filter having a pore size of 3.0 µm to separate dust or other foreign matters and then stored.

### <Preparation of Organic Polyhalogen Compound-2 Dispersion>

10 kg of an organic polyhalogen compound-2, that is, N-butyl-3-tribromomethane sulfonylbenzamide, 20 kg of a 10 mass% aqueous solution of a modified polyvinylalcohol (Poval MP203; available from Kuraray Co., Ltd.) and 0.4 kg of a 20 mass% aqueous solution of sodium triisopropylnaphthalene sulfonate were added to one another and, then, mixed thoroughly to prepare a slurry. The thus-prepared slurry was fed by using a diaphragm pump to a lateral sand mill (UVM-2; available from Aimex, Ltd.) filled with zirconia beads having an average diameter of 0.5 mm, dispersed for 5 hours, added with 0.2 g of a benzoisothiazolinone sodium salt and water such that a concentration of an organic polyhalogen compound was adjusted to be 30 mass%. The resultant dispersion was heated at 40°C for 5 hours to obtain an organic polyhalogen compound-2 dispersion. Organic polyhalogen compound particles contained in the thus-obtained polyhalogen compound dispersion were found to have a median diameter of 0.40 µm and a maximum particle diameter of 1.3 µm or less. The obtained organic polyhalogen compound dispersion was filtered through a polypropylene filter having a pore size of 3.0 µm to separate dust or other foreign matters and then stored.

### <Preparation of Phthalazine Compound-1 Solution>

8 kg of a modified polyvinyl alcohol MP203 (available from Kuraray Co., Ltd.) was dissolved in 174.57 kg of water and, then, added with 3.15 kg of a 20 mass% aqueous solution of sodium triisopropylnaphthalene sulfonate and 14.28 kg of a 70 mass% aqueous solution of a phthalazine compound-1, that is, 6-isopropylphthalazine, thereby to prepare a 5 mass% solution of the phthalazine compound-1.

### Preparation of Mercapto Compound

### <Preparation of Mercapto Compound-1 Aqueous Solution>

7 g of a mercapto compound-1, that is, a 1-(3-sufophehyl)-5-mercaptotetrazole sodium salt was dissolved in 993 g of water to prepare a 0.7 mass% aqueous solution.

### <Preparation of Mercapto Compound-2 Aqueous Solution>

20 g of a mercapto compound-2, that is, a 1-(3-methylureido)-5-mercaptotetrazole sodium salt was dissolved in 980 g of water to prepare a 2.0 mass% aqueous solution.

### <Preparation of Pigment-1 Dispersion>

64 g of C. I. Pigment Blue 60 and 6.4 g of DEMOL-N (available from Kao Corporation) were added with 250 g of water and, then, mixed thoroughly to prepare a slurry. The thus-prepared slurry was then fed into a vessel of a dispersion apparatus (1/4G Sand Grinder Mill; available from Aimex, Ltd.) together with 800 g of previously-prepared zirconia beads having an average diameter of 0.5 mm and, then, dispersed for 25 hours to obtain a pigment-1 dispersion. Pigment particles contained in the thus-obtained dispersion were found to have an average particle diameter of 0.21 µm.

### <Preparation of SBR Latex Liquid>

SBR latex having a Tg of 22°C was prepared in such a manner as described below.

70.0 mass of styrene, 27.0 mass of butadiene and 3.0 mass of acrylic acid were emulsion-polymerized by using ammonium persulfate as a polymerization initiator and an anionic surfactant as an emulsifier and, then, ripened at 80°C for 8 hours. Thereafter, the resultant polymer solution was cooled down to 40°C, adjusted so as to have a pH of 7.0 by using ammonia water, added with Sandet-BL (available from Sanyo Chemical Industries) so as to attain a concentration of 0.22% and, then, further added with a 5% NaOH aqueous solution so as to adjust a pH of the solution to be 8.3 and, thereafter, with ammonia water so as to adjust a pH thereof to be 8.4. A molar ratio of Na⁺ ion: NH₄⁺ ion was 1: 2.3. Further, 0.15ml of a 7% aqueous solution of a bonzoisothiazolinnone sodium salt, based on 1 kg of the resultant solution, was added to the resultant solution, thereby to prepare an SBR latex liquid.
SBR latex: -St(70.0)-Bu(27.0)-AA(3.0)-latex, Tg: 22°C
an average particle diameter: 0.1 µm; a concentration: 43 mass%; an equilibrium water content at 25°C, 60%RH: 0.6 mass%; ion conductivity: 4.2 mS/cm (measured on a latex stock liquid (43 mass%) at 25°C by using a conductometer CM-30S (available from Toa Electronics Ltd.); pH: 8.4.

An SBR latex having a different Tg can be prepared in a same manner as in the above-described preparation by appropriately changing a ratio of styrene and butadiene.

### <Preparation of Coating Liquid-1 for Emulsion Layer (Photosensitive Layer)>

1000 g of the above-obtained fatty acid silver dispersion, 276 ml of water, 32.8 g of the pigment-1 dispersion, 21 g of the organinc polyhalogen compound-1 dispersion, 58 g of the organinc polyhalogen compound-2 dispersion, 173 g of the phthalazine compound-1 solution, 1082 g of the SBR latex (Tg: 20°C) liquid; 155 g of the reducing agent-2 dispersion, 55 g of the hydrogen bonding type compound-1 dispersion, 6 g of the development accelerator-1 dispersion, 2 g of the development accelerator-2 dispersion, 3 g of the development accelerator-3 dispersion, 2 g of the color tone adjusting agent-1 dispersion, 9 ml of the mercapto compound-1 aqueous solution and 27 ml of the mercapto compound-2 aqueous solution were mixed in order of precedence and, then, 117 g of a silver halide mixed emulsion A was added to the resultant mixture just before it was applied and, thereafter, thoroughly mixed to obtain a coating liquid for the emulsion layer which was then directly fed to a coating die and applied.

Viscosity of the coating liquid for the emulsion layer was measured by using a B type viscometer (available from Tokyo Keiki K.K.) at 40°C (with No. 1 rotor at 60 rpm) and found to be 40 mPa·s.

Viscosities of the coating liquid measured under shearing velocities of 0.1, 1, 10, 100 and 1,000 (1/second) at 25°C by using RFS Fluid Spectrometer (available from Rheometrix Far East Inc.) were 530, 144, 96, 51 and 28 mPa·s, respectively.

A quantity of zirconium in the coating liquid was 0.25 mg based on 1 g of silver.

### <Preparation of Coating Liquid for Intermediate Layer for Emulsion Surface>

A coating liquid for an intermediate layer was prepared by mixing 1000 g of polyvinyl alcohol PVA-205 (available from Kuraray Co., Ltd.), 272 g of a 5 mass% of a pigment, 4200 ml of a 19 mass% liquid of methyl methacrylate/styrene/ butyl acrylate/hydroxyethyl methacrylate/acrylic acid copolymer (copolymerization ratio by mass of 64/9/20/5/2) latex and 27 ml of a 5 mass% aqueous solution of Aerosol OT (available from American Cyanamide Corporation), 135 ml of a 20 mass% aqueous solution of diammonium phthalate and, then, the thus-prepared coating liquid was added with water to make a total quantity thereof up to 10000 g and, thereafter, adjusting a pH of the thus-made up coating liquid to be 7.5 by NaOH. Then, the thus-prepared coating liquid for the intermediate layer was fed to a coating die so as to attain a coating amount of 9.1 ml/m².

Viscosity of the coating liquid measured at 40°C using a B type viscometer (with No. 1 rotor at 60 rpm) was 58 mPa·s.

### <Preparation of Coating Liquid for First Layer of Protective Layer for Emulsion Surface>

64 g of inert gelatin was dissolved in water and, then, added to the resultant solution were 80 g of a 27.5 mass% solution of methyl methacrylate/styrene/butylacrylate/hydroxyethyl methacrylate/acrylic acid copolymer (copolymerization ratio by mass of 64/9/20/5/2) latex, 23 ml of a 10 mass% methanol solution of phthalic acid, 23 ml of a 10 mass% aqueous solution of 4-methyl phthalic acid, 28 ml of a 0.5 mol/L concentration of sulfuric acid, 5 ml of a 5 mass% aqueous solution of Aerosol 0T (available from American Cyanamide Corporation), 0.5 g of phenoxy ethanol and 0.1 g of benzoisothiazolinone, and, then, a total weight of the resultant coating liquid was made up to 750 g by adding water, thereby to prepare a coating liquid. The thus-prepared coating liquid was mixed with 26 ml of a 4 mass% chrome alum solution by using a static mixer immediately before the coating and fed to a coating die so as to attain a coating amount of 18.6 ml/m².

Viscosity of the coating liquid measured at 40°C by using a B type viscometer (with No. 1 rotor at 60 rpm) was 20 mPa·s.

### <Preparation of Coating Liquid for Second Layer of Protective Layer for Emulsion Surface>

80 g of inert gelatin was dissolved in water and, then, added to the resultant solution were 102 g of a 27.5 mass% solution of methyl methacrylate / styrene / butylacrylate/ hydroxyethyl methacrylate/acrylic acid copolymer (copolymerization ratio by mass of 64/9/20/5/2) latex, 3.2ml of a 5 mass% solution of the fluorinated surfactant (F-1: N-perfluorooctylsulfonyl-N-propylalanine potassium salt), 32 ml of a 2 mass% aqueous solution of the fluorinated surfactant (F-2: polyethylene glycol mono(N-perfluorooctylsulfonyl-N-propyl-2-aminoethyl) ether [average degree of polymerization of ethylene oxide: 15], 23 ml of a 5 mass% solution of Aerosol OT (available from American Cyanamide Corporation), 4 g of polymethylmethacrylate fine particles (average particle diameter: 0.7 µm), 21 g of polymethylmethacrylate fine particles (average particle diameter: 4.5 µm), 1.6 g of 4-methylphthalic acid, 4.8 g of phthalic acid, 44 ml of a 0.5 mol/L concentration of sulfuric acid and 10 mg of benzoisothiazolinone, and, then, a total weight of the resultant coating liquid was made up to 650 g by adding water, thereby to prepare a coating liquid. The thus-prepared coating liquid was mixed with 445 ml of an aqueous solution containing 4 mass% of chrome alum solution and 0.67 mass% of phthalic acid by using a static mixer immediately before the coating and fed to a coating die so as to attain a coating amount of 8.3 ml/m².

Viscosity of the coating liquid measured at 40°C by using a B type viscometer (with No. 1 rotor at 60 rpm) was 19 mPa·s.

### <Preparation of Photothermographic Material-1>

On a back surface side of the above-described undercoated support, a coating liquid for an anti-halation layer and a coating liquid for a back surface protective layer were simultaneously applied in a stacked manner such that coating quantities of gelatin became 0.44 g/m² and 1.7 g/m², respectively and, then, dried to prepare a back surface layer.

On a surface opposite to the back surface, an emulsion layer, an intermediate layer, a first layer of a protective layer and a second layer of the protective layer were simultaneously coated in a stacked manner in this order as viewed from an undercoated surface by using a slide bead application method and dried, thereby to obtain a sample of the photothermographic material. At this time, temperatures of the emulsion layer and the intermediate layer were adjusted to be 31°C, while temperatures of the first layer of the protective layer and the first layer of the protective layer were adjusted to be 36°C and 37°C, respectively.

Coated quantities (g/m²) of respective compounds in the emulsion layer are as follows:

| | |
|---|---|
| silver behenate | 5.55 |
| pigment (C. I. Pigment Blue 60) | 0.036 |
| polyhalogen compound-1 | 0.12 |
| polyhalogen compound-2 | 0.37 |
| phthalazine compound-1 | 0.19 |
| SBR latex | 9.97 |
| reducing agent-1 | 0.81 |
| hydrogen bonding type compound-1 | 0.30 |
| development accelerating agent-1 | 0.024 |
| development accelerating agent-2 | 0.010 |
| development accelerating agent-3 | 0.015 |
| color tone adjusting agent-1 | 0.010 |
| mercapto compound-1 | 0.002 |
| mercapto compound-2 | 0.012 |
| silver halide (in terms of Ag) | 0.091 |

### Coating and drying conditions are as follows:

Coating was performed at a speed of 160 m/min while keeping a gap between an end of a coating die and a support to be from 0.10 mm to 0.30 mm and keeping a pressure in a reduced pressure chamber lower by from 196 Pa to 882 Pa than the atmospheric pressure. The support was blown with ion wind before the coating to cancel electricity.

Next, the coated liquid was cooled in a chilling zone by blowing wind having a dry-bulb temperature of from 10°C to 20°C and, then, transferred in a non-contact type manner and, thereafter, dried by a drying wind having a dry-bulb temperature of from 23°C to 45°C and a wet-bulb temperature of from 15°C to 21°C in a helical non-contact type drying apparatus.

After the coating liquid was dried, the thus-dried coating liquid was conditioned at 25°C, from 40 %RH to 60 %RH and, then, a surface of the resultant layer was heated up to from 70°C to 90°C and, subsequently, cooled down to 25°C.

A degree of matting expressed by Beck smoothness of the thus-prepared photothermographic material was found to be 550 seconds for the photosensitive layer side and 130 seconds for the back surface side. Further, a pH of the layer surface on a photosensitive layer side was measured and found to be 6.0.

Chemical structures of compounds used in embodiments according to the invention are shown below.

The obtained sample was cut into a half-cut size, packaged by a packaging material described below under an atmosphere of 25°C and 50% RH and stored at normal temperature for 2 weeks.

### Packaging Material

PET: 10 µm/PE: 12 µm / aluminum foil: 9 µm/ Ny: 15 µm/polyethylene containing 3% of carbon: 50 µm;
oxygen permeability: 0.02 ml/atm·m²·25°C·day; and
water permeability: 0.10 g/atm·m²·25°C·day.

### <Preparation of photothermographic materials-2 to -8>

Silver halide emulsions-2 and -3 each having a uniform halogen composition as shown in Table 1 were prepared in a same manner as in preparation of silver halide emulsion 1 by changing respective halogen compositions to be added.

Silver halide having an average sphere-equivalent diameter of 0.040 µm as a particle size was prepared by changing a temperature at the time of particle formation.

The photothermographic materials-2 to -8 were prepared in a same manner as in the photothermographic material-1 except that compounds expressed by a general formula (1) were changed as shown in Table 1.

### <Evaluation of Photothermographic Material>

The obtained samples were exposed by Fuji Medical Dry Laser Imager "FM-DPL" (equipped with a 660-nm semiconductor laser device having a maximum output of 60 mW (IIIB)) and thermally developed for 14 seconds in total by 4 panels constituting a panel heater in which respective temperatures were set to be 112°C, 119°C, 121°C and 121°C, respectively.

### Evaluation of Samples

Density measurements were performed on the obtained samples by using a densitometer to construct a characteristic curve of density against a logarithm of an exposure amount. An optical density of an unexposed portion was defined as fog and a reciprocal number of an exposure amount which can obtain an optical density of 3.0 was defined as sensitivity which was shown as a relative value when the sensitivity of the photothermographic material 1 was taken as 100. Further, an average contrast of an optical density of 1.5 and an optical density of 3.0 was measured. The results are shown in Table 1.

### Evaluation of Print-out Performance

The photothermographic material which has been subjected to development processing was left to stand in a room at 25°C and 60% RH under a fluorescent lamp of 100 luxes for 30 days. A difference of a fog density just after the development processing and a fog density after such a 30-day left-over was defined as a print-out performance. It is preferable that the fog is increased to a small extent even after such left-over under these conditions. The results are shown in Table 1.

**[Table 1]**

| Photothermographic Material | Emulsion No. | Average Iodine Content (%) | Particle Size | Compound of General Formula (I) | Sensitivity | Fog | Average Contrast | Print-Out | Remarks |
|---|---|---|---|---|---|---|---|---|---|
| 1 | 1 | 12 | 40nm | Chemical Formula I-1 | 100 | 0.17 | 3.7 | 0.02 | Present Invention |
| 2 | 1 | 12 | 40nm | No | 25 | 0.17 | 3 | 0.02 | Comparison |
| 3 | 1 | 12 | 40nm | Chemical Formula I-2 | 97 | 0.18 | 3.5 | 0.02 | Present Invention |
| 4 | 1 | 12 | 40nm | Chemical Formula I-3 | 95 | 0.17 | 3.3 | 0.02 | Present Invention |
| 5 | 2 | 3.5 | 40nm | No | 52 | 0.19 | 2.8 | 0.06 | Comparison |
| 6 | 2 | 3.5 | 40nm | Chemical Formula I-1 | 72 | 0.22 | 3.1 | 0.10 | Comparison |
| 7 | 3 | 0 | 40nm | No | 62 | 0.19 | 2.5 | 0.08 | Comparison |
| 8 | 3 | 0 | 40nm | Chemical Formula I-1 | 75 | 0.26 | 2.9 | 0.12 | Comparison |

As is apparent from Table 1, it was found that the photothermographic material of the first embodiment according to the invention is excellent in print-out properties such that it has a high sensitivity, a low fog and a favorable gradation.

### Example 2

### <Preparation of Silver Halide Emulsion 4>

To 1,421 ml of water, added were 4.3 ml of a 1 mass% potassium iodide solution, 3.5 ml of a 0.5 mol/L concentration of sulfuric acid and 36.7 g of phthalized gelatin; while the resultant liquid was kept stirring in a stainless-steel reaction vessel at a liquid temperature of 42°C, was added thereto an entire volume of a solution A in which 22.22 g of silver nitrate was diluted by distilled water to be 195.6 ml and a solution B in which 21.8 g of potassium iodide was diluted by distilled water to be 218 ml at a constant flow rate over 9 minutes.

Thereafter, the resultant solution was added with 10 ml of a 3.5 mass% aqueous hydrogen peroxide solution and, further, with 10.8 ml of a 10 mass% aqueous solution of benzoimidazole. Further, was added thereto an entire volume of a solution C in which 30.64 g of silver nitrate was diluted with distilled water to be 187.6 ml and a solution D in which 40.0 g of potassium bromide was diluted with distilled water to be 400 ml such that an entire volume of the solution C was added thereto at a constant flow rate over 12 minutes and the solution D was added by a controlled double jet method while pAg thereof is kept at 8.1.

Thereafter, was added thereto a solution E in which 22.2 g of silver nitrate was diluted with distilled water to be 130.0 ml and a solution Fto in which 21.7 g of potassium iodide was diluted with distilled water to be 217 ml by a controlled double jet method while a pAg is kept at 6.3.

Further, added thereto was an entire volume of potassium hexachloroiridate(III) 10 minutes after the solution C and the solution D started to be added so as to attain a concentration of 1X10⁻⁴ mol/mol of Ag. Furthermore, an entire volume of 3X10⁻⁴ mol/mol of Ag of an aqueous solution of potassium iron (II) hexacyanate was added thereto 5 seconds after completion of such an addition of the solution C.

Thereafter, a pH of the resultant mixture was adjusted to be 3.8 by using a 0.5 mol/L concentration of sulfuric acid, stirring was stopped and the resultant mixture was subjected to sedimentation/desalting/rinsing operations. Then, the pH of the mixture was adjusted to be 5.9 by using a 1 mol/L concentration of sodium hydroxide to prepare a silver halide dispersion having a pAg of 8.0.

While the thus-prepared silver halide dispersion was kept stirring at 38°C, the dispersion was added with 5 ml of a 0.34 mass% methanol solution of 1,2-benzisothiazolin-3-one and, one minute after the above addition, a temperature of the resultant dispersion was raised to 47°C. 20 minute after such temperature raising, the resultant dispersion was added with a methanol solution of sodium benzene thiosulfonate in an amount of 7.6X10⁻⁵ mol/mol of Ag and, further, 5 minutes after such an addition, added with a methanol solution of a tellurium sensitizer B in an amount of 2.9X10⁻⁴ mol/mol of Ag and, then, ripened for 91 minutes.

Thereafter, the resultant dispersion was added with 1.3 ml of a 0.8 mass% methanol solution of N,N'-dihydroxy-N"-diethylmelamine and, further 4 minutes after such an addition, added with a methanol solution of 5-methyl-2-mercaptobenzoimidazole in an amount of 4.8X10⁻³ mol/mol of Ag, a methanol solution of 1-phenyl-2-heptyl-5-mercapto-1,3,4-triazole in an amount of 5.4X10⁻³ mol/mol of Ag and an aqueous solution of a mercapto compound-2 in an amount of 1.5X10⁻² mol/mol of Ag to obtain a silver halide emulsion 1.

Particles contained in the thus-prepared silver halide emulsion were pure silver iodide particles having an average sphere-equivalent diameter of 0.042 µm and a sphere-equivalent coefficient of variation of 18%. On this occasion, a particle size and the like were determined based on an average of 1000 particles under an electron microscopic observation.

### <Preparation of Silver Halide Emulsions 5 to 17>

Silver halide emulsions 5 to 17 each having a halogen structure as shown in Table 2 were prepared in a same manner as in <Preparation of Silver Halide Emulsion 4> except for a step of changing halogen compositions of the solutions B, D and F.

The silver halide was formed such that it has an average sphere-equivalent diameter of 0.04 µm as a particle size.

### <Preparation of Silver Halide Emulsions 18 to 21>

Emulsions in each of which particles were formed in a same manner as in <Preparation of Silver Halide Emulsion 9> were added with an aqueous solution of potassium iodide such that they have respective average iodine compositions as shown in Table 2 and, then, subjected to sedimentation/desalting/rinsing operations to prepare silver halide emulsions 18 and 19. Silver halide emulsions 20 and 21 as shown in Table 2 were also prepared in a same manner as in <Preparation of Silver Halide Emulsion 6>.

Among these silver halide emulsions 5 to 21, emulsions which have a crystal structure of silver halide structure had an intense light absorption by direct transition.

**[Table 2]**

| Emulsion No. | Core Iodine Content (%) | First Shell Iodine Content (%) | Second Shell Iodine Content (%) | Average Iodine Quantity (%) | Direct Transition Absorption Attributable to Silver Iodide Crystal Structure | Particle Size |
|---|---|---|---|---|---|---|
| 4 | 100 | 100 | 100 | 100 | Yes | 40nm |
| 5 | 95 | 95 | 95 | 95 | Yes | 40nm |
| 6 | 40 | 40 | 40 | 40 | No | 40nm |
| 7 | 10 | 10 | 10 | 10 | No | 40nm |
| 8 | 3.5 | 3.5 | 3.5 | 3.5 | No | 40nm |
| 9 | 0 | 0 | 0 | 0 | No | 40nm |
| 10 | 0 | 0 | 100 | 30 | Yes | 40nm |
| 11 | 0 | 100 | 0 | 40 | Yes | 40nm |
| 12 | 0 | 100 | 100 | 70 | Yes | 40nm |
| 13 | 100 | 0 | 0 | 30 | Yes | 40nm |
| 14 | 100 | 100 | 0 | 70 | Yes | 40nm |
| 15 | 0 | 0 | 40 | 8 | No | 40nm |
| 16 | 0 | 40 | 0 | 12 | No | 40nm |
| 17 | 40 | 0 | 0 | 8 | No | 40nm |
| 18 | Conversion Method | | | 10 | No | 40nm |
| 19 | Conversion Method | | | 30 | No | 40nm |
| 20 | Conversion Method | | | 60 | Yes | 40nm |
| 21 | Conversion Method | | | 90 | Yes | 40nm |

### <Preparation of Photothermographic Materials-9 to -31>

Photothermographic materials-9 to -31 as shown in Table 3 were prepared in a same manner as in <Preparation of Photothermographic Materials-1> of Example 1 while compounds expressed by the general formula (1) are same as those in the photothermographic material-1.

The thus-prepared photothermographic materials were evaluated in such a manner as described below.

### Exposure of Photothermographic material

The photothermographic materials obtained in Example 2 were subjected to exposure processing in such a manner as described below.

The photothermographic materials were exposed for 10⁻⁶ second by Fuji Medical Dry Laser Imager "FM-DPL" equipped with a semiconductor laser device "NLHV3000E" (available from Nichia Corporation) as a semiconductor laser beam supply in an exposure portion thereof while illuminance of laser beams on a surface of the photothermographic materials is allowed to change from 0 and 1 mW/mm² to 1000 mW/mm² by stopping down a beam diameter. An emission wavelength of the laser beams was 405 nm.

### Development of Photothermographic Material

The thus-exposed photothermographic materials were subjected to thermal development processing in such a manner as described below.

In a thermal development portion of Fuji Medical Dry Laser Imager "FM-DPL", temperatures of 4 panels which constitute a panel heater were set to be 112°C, 110°C, 110°C and 110°C, respectively, and, then, the thermal development was performed such that a total thermal development time becomes 14 seconds by increasing a film transfer speed.

Evaluations of samples was performed in a same manner as in Example 1 and the results thereof are shown in Table 3.

**[Table 3]**

| Photothermographic Material | Emulsion No. | Average Iodine Quantity (%) | Direct Transition Absorption Attributable to Silver Iodide Crystal Structure | Compound of General Formula (I) | Sensitivity | Fog | Average Contrast | Print-out | Remarks |
|---|---|---|---|---|---|---|---|---|---|
| 9 | 4 | 100 | Yes | Chemical Formula I-1 | 100 | 0.16 | 3.6 | 0.00 | Present Invention |
| 10 | 4 | 100 | Yes | No | 25 | 0.17 | 3.0 | 0.00 | Comparison |
| 11 | 5 | 95 | Yes | Chemical Formula I-1 | 98 | 0.17 | 3.5 | 0.01 | Present Invention |
| 12 | 6 | 40 | No | Chemical Formula I-1 | 64 | 0.17 | 3.4 | 0.02 | Present Invention |
| 13 | 7 | 10 | No | Chemical Formula I-1 | 42 | 0.18 | 3.3 | 0.03 | Present Invention |
| 14 | 8 | 3.5 | No | Chemical Formula I-1 | 36 | 0.25 | 3.0 | 0.10 | Comparison |
| 15 | 8 | 3.5 | No | No | 22 | 0.18 | 2.8 | 0.06 | Comparison |
| 16 | 9 | 0 | No | Chemical Formula I-1 | 41 | 0.26 | 2.8 | 0.12 | Comparison |
| 17 | 10 | 30 | Yes | Chemical Formula I-1 | 77 | 0.18 | 3.3 | 0.02 | Present Invention |
| 18 | 11 | 40 | Yes | Chemical Formula I-1 | 82 | 0.18 | 3.4 | 0.02 | Present Invention |
| 19 | 12 | 70 | Yes | Chemical Formula I-1 | 93 | 0.17 | 3.5 | 0.01 | Present Invention |
| 20 | 12 | 70 | Yes | No | 37 | 0.17 | 3.0 | 0.01 | Comparison |
| 21 | 13 | 30 | Yes | Chemical Formula I-1 | 74 | 0.18 | 3.3 | 0.02 | Present Invention |
| 22 | 14 | 70 | Yes | Chemical Formula I-1 | 92 | 0.17 | 3.5 | 0.01 | Present Invention |
| 23 | 15 | 8 | No | Chemical Formula I-1 | 42 | 0.19 | 3.2 | 0.03 | Present Invention |
| 24 | 16 | 12 | No | Chemical Formula I-1 | 52 | 0.18 | 3.3 | 0.03 | Present Invention |
| 25 | 16 | 12 | No | No | 14 | 0.18 | 2.9 | 0.03 | Comparison |
| 26 | 17 | 8 | No | Chemical Formula I-1 | 42 | 0.18 | 3.2 | 0.03 | Present Invention |
| 27 | 18 | 10 | No | Chemical Formula I-1 | 44 | 0.18 | 3.3 | 0.03 | Present Invention |
| 28 | 19 | 30 | No | Chemical Formula I-1 | 57 | 0.18 | 3.3 | 0.02 | Present Invention |
| 29 | 20 | 60 | Yes | Chemical Formula I-1 | 82 | 0.17 | 3.5 | 0.02 | Present Invention |
| 30 | 21 | 90 | Yes | Chemical Formula I-1 | 94 | 0.16 | 3.5 | 0.01 | Present Invention |
| 31 | 21 | 90 | Yes | No | 28 | 0.17 | 3.5 | 0.01 | Comparison |

As is apparent from Table 3, it was found that the photothermographic materials according the invention shows an excellent performance also by a blue color laser exposure.

### Example 3

Pure silver halide emulsion 22 having an average particle size of 100 nm was prepared in a same manner as in <Preparation of Silver Halide Emulsion 4> of Example 2 except for a step of changing temperatures at the time of forming particles. Photothermographic materials 32, 33 and 34 as shown in Table 4 were prepared in a same manner as in the photothermographic material 9 of Example 2 except for a step of changing a quantity to be applied of the pure silver halide emulsion 22.

Photographic evaluations were performed in a same manner as in Example 2. On this occasion, a maximum optical density of samples after subjected to thermal development processing was designated as Dmax. The results are shown in Table 4.

**[Table 4]**

| Photothermographic Material | Exposure Condition | Iodine Content | Br Content | Silver Halide Particle Size | Silver Halide Quantity to be Applied (in terms of Ag) | Direct Transition Absorption Attributable to Silver Iodide Crystal Structure | Fog | Sensitivity | Dₘₐₓ |
|---|---|---|---|---|---|---|---|---|---|
| 1 | Laser Exposure 405nm | 100 | 0 | 40nm | 0.091 mg/m² | Yes | 0.18 | 100 | 4.2 |
| 32 | Laser Exposure 405nm | 100 | 0 | 100nm | 0.091 mg/m² | Yes | 0.18 | Not Capable of Performing Evaluation Due to Absence of Density | 2 |
| 33 | Laser Exposure 405nm | 100 | 0 | 100nm | 0.18 mg/m² | Yes | 0.18 | 120 | 3.2 |
| 34 | Laser Exposure 405nm | 100 | 0 | 100nm | 0.36 mg/m² | Yes | 0.17 | 75 | 3.6 |

As is apparent from Table 4, when an average particle size of the silver iodide emulsion was as low as 100 nm, the silver iodide emulsion can not attain a sufficient sensitivity, thereby to decrease Dmax. Ordinarily, since absorption of a silver halide is proportional to a third power of an average particle size, as a silver halide becomes larger in size, the silver halide is considered to have a higher sensitivity; however, it is not always true with a high silver iodide type emulsion according to the invention.

It is preferable that, by allowing the average particle size to be small, sensitivity is rather enhanced when a particle size is taken into consideration and, at the same time, Dmax is also enhanced.

### Example 4

A pure silver iodide emulsion 23 having an average particle size of 70 nm and a coefficient of variation of 8% was prepared in a same manner as in <Preparation of Silver Halide Emulsion 4> of Example 2 except for a step of elevating a temperature at the time of forming particles. In like manner, by changing temperatures at the time of forming particles, a pure silver iodide emulsion 24 having an average particle size of 28 nm and a coefficient of variation of 12% was prepared.

A photothermographic material 35 was prepared in a same manner as in Example 2 except that a mixture of the silver halide emulsions 4, 23 and 24 at a mixing ratio of 60:15:25 was added instead of the silver halide emulsion 4 in the photothermographic material-9. When same evaluations were performed as in Example 2, a favorable result was obtained. An average contrast of the photothermographic material 35 was 2.7.

In like manner, a photothermographic material 36 was prepared by mixing the silver halide emulsion 12 and the silver halide emulsion 23 at a mixing ratio of 85:15. Same evaluations as in Example 2 were performed. A favorable result was obtained.

Thus, the silver halide emulsions according to the first embodiment of the invention can be used by being mixed with each other at an arbitrary mixing ratio.

### Example 5

Silver halide emulsions 25 to 42 were prepared in a same manner as in <Preparation of Silver Halide Emulsions 4 to 21> of Example 2 except that, 3 minutes after the addition of the tellurium sensitizer, potassium iodooleate and potassium thiocyanate were added in amounts of 5X10⁻⁴ mol/mol of Ag and 2X10⁻³ mol/mol of Ag, respectively.

By using these emulsions, photothermographic materials 37 to 54 were prepared in a same manner as in the photothermographic material 9 of Example 2. As a result of performing same evaluations as those in Example 2, a favorable result that sensitivity was enhanced twofold while fog and print-out performances were not deteriorated was obtained.

### Example 6

A photothermographic material 55 was prepared in a same manner as in the photothermographic material 9 except that fluorine-type surfactants F-1, F-2, F-3 and F-4 in the protective layer for the back surface and the protective layer for the emulsion surface in the photothermographic material 9 of Example 2 were changed into F-5, F-6, F-7 and F-8.

When evaluations were performed in a same manner as in Example 2, a same favorable result as in the photothermographic material 9 was obtained.

F-4 C₈F₁₇SO₃K

According to the present invention, the first embodiment of the photothermographic material, comprising a high silver iodide type photothermographic material, which has a high sensitivity and a high image quality, and a thermal development method using the photothermographic material can be provided.

## Claims

1. A photothermographic material comprising a support having thereon a layer including at least a non-photosensitive organic silver salt, a photosensitive silver halide, a reducing agent and a binder;
wherein the photosensitive silver halide has a mean silver iodide content of 70 to 100 mol %
and further comprising at least one compound of the following general formula (I):
General formula (I) (X)ₖ―(L)ₘ―(A―B)ₙ
wherein X represents a silver halide-adsorbing group or a light-absorbing group that has at least one atom of N, S, P, Se and Te; L represents a (k + n)-valent linking group having at least one atom of C, N, S and O; A represents an electron-donating group; B represents a leaving group or a hydrogen group; A-B is oxidized and then cleaved or deprotonated to generate a radical A; k represents an integer from 0 to 3; m represents 0 or 1; n represents 1 or 2; and when k = 0 and n = 1, then m = 0.

2. The photothermographic material according to claim 1, wherein the mean silver iodide content of the silver halide is 90 to 100 mol %.

3. The photothermographic material according to claim 1, wherein the oxidation potential of (A-B) falls between 0 and 1.5 V.

4. The photothermographic material according to claim 1, wherein the photosensitive silver halide comprises a mean grain size of 5 to 80 nm.

5. The photothermographic material according to claim 1, wherein the mean grain size of the silver halide is 5 to 70 nm.

6. The photothermographic material according to claim 1, wherein the silver halide grains have a direct transition absorption derived from the high silver iodide crystal structure therein.

7. A method of thermal development of a photothermographic material, which comprises a support having thereon a layer including at least a non-photosensitive organic silver salt, a photosensitive silver halide, a reducing agent and a binder; wherein the photosensitive silver halide has a mean silver iodide content of 70 to 100 mol % , and which further comprises at least one compound of the following general formula (I),
wherein the highest temperature at thermal development of the photothermographic material is 100 to 120°C.
General formula (I) (X)ₖ―(L)ₘ―(A―B)ₙ
wherein X represents a silver halide-adsorbing group or a light-absorbing group that has at least one atom of N, S, P, Se and Te; L represents a (k + n)-valent linking group having at least one atom of C, N, S and O; A represents an electron-donating group; B represents a leaving group or a hydrogen group; A-B is oxidized and then cleaved or deprotonated to generate a radical A; k represents an integer from 0 to 3; m represents 0 or 1; n represents 1 or 2; and when k = 0 and n = 1, then m = 0.

8. The method of thermal development of the photothermographic material according to claim 7, wherein the highest temperature when thermally developing the photothermographic material is 105 to 115°C.

9. The method of thermal development of the photothermographic material according to claim 7, wherein the photothermographic material is thermally developed by being conveyed through a thermal development zone that comprises from 2 to 6 plate heaters for thermal development and by being kept in contact with the plate heaters in that zone.

10. The method of thermal development of the photothermographic material according to claim 7, wherein the mean grain size of the silver halide is 5 to 80 nm.

11. The method of thermal development of the photothermographic material according to claim 7, wherein the mean grain size of the silver halide is 5 to 70 nm.

## Patentansprüche

1. Fotothermografisches Material umfassend einen Träger mit einer darauf aufgebrachten Schicht, die wenigstens ein nicht-fotoempfindliches organisches Silbersalz, ein fotoempfindliches Silberhalogenid, ein Reduktionsmittel und ein Bindemittel umfaßt;
wobei das fotoempfindliche Silberhalogenid einen mittleren Silberiodidgehalt von 70 bis 100 mol% aufweist,
und ferner umfassend wenigstens eine Verbindung der folgenden allgemeinen Formel (I):
(X)ₖ―(L)ₘ―(A―B)ₙ (I)
wobei X eine Silberhalogenid-adsorbierende Gruppe oder eine lichtabsorbierende Gruppe darstellt, die wenigstens ein Atom aus N, S, P, Se und Te aufweist; L eine (k + n)-bindige Verbindungsgruppe mit wenigstens einem Atom aus C, N, S und 0 darstellt; A eine elektronenabgebende Gruppe darstellt; B eine Abgangsgruppe oder eine Wasserstoffgruppe darstellt; A-B oxidiert wird und dann abgespalten oder deprotoniert wird, um ein Radikal A zu erzeugen; k eine ganze Zahl von 0 bis 3 darstellt; m 0 oder 1 darstellt; n 1 oder 2 darstellt; und wenn k = 0 und n = 1, dann m = 0.

2. Fotothermografisches Material gemäß Anspruch 1, wobei der mittlere Silberiodidgehalt des Silberhalogenids 90 bis 100 mol% beträgt.

3. Fotothermografisches Material gemäß Anspruch 1, wobei das Oxidationspotential von (A-B) zwischen 0 und 1,5 V fällt.

4. Fotothermografisches Material gemäß Anspruch 1, wobei das fotoempfindliche Silberhalogenid eine mittlere Korngröße von 5 bis 80 nm umfaßt.

5. Fotothermografisches Material gemäß Anspruch 1, wobei die mittlere Korngröße des Silberhalogenids 5 bis 70 nm beträgt.

6. Fotothermografisches Material gemäß Anspruch 1, wobei die Silberhalogenidkörner eine direkte Übergangsabsorption aufweisen, die von der hohen Silberiodidkristallstruktur darin abgeleitet ist.

7. Verfahren zum thermischen Entwickelns eines fotothermografischen Materials, das einen Träger mit einer Schicht darauf umfaßt, die wenigstens ein nicht-fotoempfindliches organisches Silbersalz, ein fotoempfindliches Silberhalogenid, ein Reduktionsmittel und ein Bindemittel umfaßt, wobei das fotoempfindliche Silberhalogenid einen mittleren Silberiodidgehalt von 70 bis 100 mol% aufweist, und die ferner wenigstens eine Verbindung der allgemeinen Formel (I) umfaßt,
wobei die höchste Temperatur beim thermischen Entwickeln des fotothermografischen Materials 100 bis 120°C beträgt;
(X)ₖ―(L)ₘ―(A―B)ₙ (I)
wobei X eine Silberhalogenid-adsorbierende Gruppe oder eine lichtabsorbierende Gruppe darstellt, die wenigstens ein Atom aus N, S, P, Se und Te aufweist; L eine (k + n)-bindige Verbindungsgruppe mit wenigstens einem Atom aus C, N, S und 0 darstellt; A eine elektronenabgebende Gruppe darstellt; B eine Abgangsgruppe oder eine Wasserstoffgruppe darstellt; A-B oxidiert wird und dann abgespalten oder deprotoniert wird, um ein Radikal A zu erzeugen; k eine ganze Zahl von 0 bis 3 darstellt; m 0 oder 1 darstellt; n 1 oder 2 darstellt; und wenn k = 0 und n = 1, dann m = 0.

8. Verfahren zum thermischen Entwickeln des fotothermografischen Materials gemäß Anspruch 7, wobei die höchste Temperatur beim thermischen Entwickeln des fotothermografischen Materials 105 bis 115°C beträgt.

9. Verfahren zum thermischen Entwickeln des fotothermografischen Materials gemäß Anspruch 7, wobei das fotothermografische Material thermisch entwickelt wird, indem es durch eine thermische Entwicklungszone gefördert wird, die 2 bis 6 Plattenheizgeräte zum thermischen Entwickeln umfaßt und es in Kontakt mit den Plattenheizgeräten in dieser Zone gehalten wird.

10. Verfahren zum thermischen Entwickeln des fotothermografischen Materials gemäß Anspruch 7, wobei die mittlere Korngröße des Silberhalogenids 5 bis 80 nm beträgt.

11. Verfahren zum thermischen Entwickeln des fotothermografischen Materials gemäß Anspruch 7, wobei die mittlere Korngröße des Silberhalogenids 5 bis 70 nm beträgt.

## Revendications

1. Matière photothermographique comprenant un support sur lequel se trouve une couche incluant au moins un sel organique d'argent non photosensible, un halogénure d'argent photosensible, un agent réducteur et un liant ;
dans laquelle l'halogénure d'argent photosensible a une teneur moyenne en iodure d'argent comprise entre 70 et 100 mol %
et comprenant de plus au moins un composé de formule générale suivante (I) :
Formule générale (I) (X)ₖ―(L)ₘ―(A―B)ₙ
dans laquelle X représente un groupe accepteur d'halogénure d'argent ou un groupe absorbant de la lumière qui a au moins un atome de N, S, P, Se et Te ; L représente un groupe de liaison de valence (k + n) ayant au moins un atome de C, N, S et O ; A représente un groupe donneur d'électrons ; B représente un groupe départ ou un groupe hydrogène ; A-B est oxydé et ensuite clivé ou déprotoné pour générer un radical A ; k représente un entier de 0 à 3 ; m représente 0 ou 1 ; n représente 1 ou 2 ; et quand k = 0 et n = 1, alors m = 0.

2. Matière photothermographique selon la revendication 1, dans laquelle la teneur moyenne en iodure d'argent de l'halogénure d'argent est comprise entre 90 et 100 mol %.

3. Matière photothermographique selon la revendication 1, dans laquelle le potentiel d'oxydation de (A-B) tombe entre 0 et 1,5 V.

4. Matière photothermographique selon la revendication 1, dans laquelle l'halogénure d'argent photosensible comprend une taille de grain moyenne comprise entre 5 et 80 nm.

5. Matière photothermographique selon la revendication 1, dans laquelle la taille de grain moyenne de l'halogénure d'argent est comprise entre 5 et 70 nm.

6. Matière photothermographique selon la revendication 1, dans laquelle les grains d'halogénure d'argent ont une absorption de transition directe provenant de la structure hautement cristalline de l'iodure d'argent en leur sein.

7. Procédé de développement thermique d'une matière photothermographique, qui comprend un support sur lequel se trouve une couche incluant au moins un sel organique d'argent non photosensible, un halogénure d'argent photosensible, un agent réducteur et un liant ; dans lequel l'halogénure d'argent photosensible a une teneur moyenne en iodure d'argent comprise entre 70 et 100 mol % et qui comprend de plus au moins un composé de formule générale suivante (I),
dans lequel la température la plus élevée au moment du développement thermique de la matière photothermographique est comprise entre 100 et 120 °C.
Formule générale (I) (X)ₖ―(L)ₘ―(A―B)ₙ
dans laquelle X représente un groupe accepteur d'halogénure d'argent ou un groupe absorbant de la lumière qui a au moins un atome de N, S, P, Se et Te ; L représente un groupe de liaison de valence (k + n) ayant au moins un atome de C, N, S et O ; A représente un groupe donneur d'électrons ; B représente un groupe départ ou un groupe hydrogène ; A-B est oxydé et ensuite clivé ou déprotoné pour générer un radical A ; k représente un entier de 0 à 3 ; m représente 0 ou 1 ; n représente 1 ou 2 ; et quand k = 0 et n = 1, alors m = 0.

8. Procédé de développement thermique de la matière photothermographique selon la revendication 7, dans lequel la température la plus élevée quand on développe de manière thermique la matière photothermographique est comprise entre 105 et 115 °C.

9. Procédé de développement thermique de la matière photothermographique selon la revendication 7, dans lequel la matière photothermographique est développée de manière thermique en étant acheminée à travers une zone de développement thermique qui comprend de 2 à 6 réchauffeurs à plaques pour un développement thermique et en étant maintenu en contact avec les réchauffeurs à plaques dans cette zone.

10. Procédé de développement thermique de la matière photothermographique selon la revendication 7, dans lequel la taille de grain moyenne de l'halogénure d'argent est comprise entre 5 à 80 nm.

11. Procédé de développement thermique de la matière photothermographique selon la revendication 7, dans lequel la taille de grain moyenne de l'halogénure d'argent est comprise entre 5 et 70 nm.
